



US006177238B1

(12) **United States Patent**  
**Fuller et al.**

(10) **Patent No.:** **US 6,177,238 B1**  
(b4) **Date of Patent:** **Jan. 23, 2001**

(54) **INK JET PRINTHEADS CONTAINING ARYLENE ETHER ALCOHOL POLYMERS AND PROCESSES FOR THEIR FORMATION**

(75) Inventors: **Timothy J. Fuller**, Pittsford; **John F. Yanus**, Webster; **Damodar M. Pai**; **Markus R. Silvestri**, both of Fairport; **Ram S. Narang**, Macedon; **William W. Limburg**, Penfield; **Dale S. Renfer**, Webster, all of NY (US)

(73) Assignee: **Xerox Corporation**, Stamford, CT (US)

(\*) Notice: Under 35 U.S.C. 154(b), the term of this patent shall be extended for 0 days.

(21) Appl. No.: **09/325,837**

(22) Filed: **Jun. 4, 1999**

(51) **Int. Cl.<sup>7</sup>** ..... **B41J 2/16; B41J 2/01**

(52) **U.S. Cl.** ..... **430/320; 347/20; 347/65**

(58) **Field of Search** ..... **430/320; 347/20, 347/47, 65**

(56) **References Cited**

U.S. PATENT DOCUMENTS

|             |         |                |       |          |
|-------------|---------|----------------|-------|----------|
| 2,125,968   | 8/1938  | Theimer        | ..... | 260/153  |
| 3,367,914   | 2/1968  | Herbert        | ..... | 260/52   |
| 3,455,868   | 7/1969  | D'Alessandro   | ..... | 260/38   |
| 3,914,194   | 10/1975 | Smith          | ..... | 260/18 R |
| 4,086,209   | 4/1978  | Hara et al.    | ..... | 260/49   |
| 4,110,279   | 8/1978  | Nelson et al.  | ..... | 260/19 R |
| 4,435,496   | 3/1984  | Walls et al.   | ..... | 430/285  |
| 4,448,948   | 5/1984  | Tsubaki et al. | ..... | 528/95   |
| 4,623,558   | 11/1986 | Lin            | ..... | 427/44   |
| 4,667,010   | 5/1987  | Eldin          | ..... | 528/125  |
| 4,688,055 * | 8/1987  | Noguchi et al. | ..... | 347/65   |
| 4,739,032   | 4/1988  | Jones          | ..... | 528/230  |
| 4,801,517   | 1/1989  | Frechet et al. | ..... | 430/59   |
| 4,806,443   | 2/1989  | Yanus et al.   | ..... | 430/56   |

(List continued on next page.)

FOREIGN PATENT DOCUMENTS

|              |         |        |
|--------------|---------|--------|
| 0-281-808    | 9/1988  | (EP) . |
| 0 663 411 A1 | 7/1995  | (EP) . |
| 0 698 823 A1 | 2/1996  | (EP) . |
| 0 827 029 *  | 3/1998  | (EP) . |
| 56-050-928   | 5/1981  | (JP) . |
| 56-50-929    | 5/1981  | (JP) . |
| 6-57-826     | 5/1981  | (JP) . |
| 63-247757 A2 | 11/1988 | (JP) . |
| 0429148      | 10/1992 | (JP) . |

OTHER PUBLICATIONS

Daly, "Chloromethylation of Condensation Polymers Containing an Oxy-1,4-Phenylene Backbone," Polymers Preprints (1979), vol. 20, No. 1, pp. 835-837.  
Camps, "Chloromethylstyrene: Synthesis, Polymerization, Transformations, Applications," JMS-Rev. Macromol. Chem. Phys., C22(3), 343-407 (1982-83).

Tabata, "Pulse Radiolysis Studies on the Mechanism of the High Sensitivity of Chloromethylated Polystyrene as an Electron Negative Resist," 1984pp. 287-288.

(List continued on next page.)

Primary Examiner—John A. McPherson

(74) Attorney, Agent, or Firm—Judith L. Byorick

(57)

**ABSTRACT**

Disclosed is an ink jet printhead containing a polymer of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



or a mixture of



wherein R is a hydrogen atom, an alkyl group, an aryl group, or mixtures thereof, B is one of specified groups, such as



or mixtures thereof, and n is an integer representing the number of repeating monomer units.

**20 Claims, 3 Drawing Sheets**

## U.S. PATENT DOCUMENTS

|             |         |                             |         |
|-------------|---------|-----------------------------|---------|
| 4,806,444   | 2/1989  | Yanus et al. ....           | 430/56  |
| 4,818,650   | 4/1989  | Limburg et al. ....         | 430/56  |
| 4,935,487   | 6/1990  | Yanus et al. ....           | 528/203 |
| 4,956,440   | 9/1990  | Limburg et al. ....         | 528/99  |
| 5,030,532   | 7/1991  | Limburg et al. ....         | 430/56  |
| 5,268,444   | 12/1993 | Jensen et al. ....          | 528/125 |
| 5,336,577   | 8/1994  | Spiewak et al. ....         | 430/59  |
| 5,336,720   | 8/1994  | Richards ....               | 525/78  |
| 5,438,082   | 8/1995  | Helmer-Metzmann et al. .... | 552/149 |
| 5,561,202   | 10/1996 | Helmer-Metzmann et al. .... | 525/471 |
| 5,728,498   | 3/1998  | Yanus et al. ....           | 430/59  |
| 5,849,809 * | 12/1998 | Narang et al. ....          | 522/35  |

## OTHER PUBLICATIONS

- Jurke, "Deep UV Photochemistry of Copolymers of Trimethylsilylmethyl Methacrylate and Chloromethylstyrene," *Polymer Preprints*, 1988, pp. 546-547.
- Hergenrother, "Poly(arylene ethers)," *Polymer*, 1988, vol. 29, Feb.
- Havens, "Ethynyl-Terminated Polyarylates: Synthesis and Characterization," *Journal of Polymer Science: Polymer Chemistry Edition*, vol. 22 (1984), pp. 3011-3025.
- Hendricks, "Flare, A Low Dielectric Constant, High T<sub>g</sub>, Thermally Stable Poly(Arylene Ether) Dielectric for Microelectronic Circuit Interconnect Process Integration: Synthesis, Characterization, Thermomechanical Properties, and Thin-Film Processing Studies," *Polymer Preprints* 37(1) 150 (1996), vol. 37, No. 1, Mar. 1996, pp. 150-151.

Zupancic, "Styrene Terminated Resins as Interlevel Dielectrics for Multichip Modules," 1991, pp. 178-179.

Percec, "Functional Polymers and Sequential Copolymers by Phase Transfer Catalysis, 2a)," *Makromol Chem.*, 1984, pp. 1867-1880.

Percec, "Functional Polymers and Sequential Copolymers by Phase Transfer Catalysis, 3a)," *Makromol Chem.*, 1984, pp. 2319-2336.

Percec, "Functional Polymers and Sequential Copolymers by Phase Transfer Catalysis 4. A New and Convenient Synthesis of p- and m-Hydrozomethylphenylacetylene," *Polymer Bulletin* 10, 223-230, 1983.

Amato, "A New Preparation of Chloromethyl Methyl Ether Free of Bis(chloromethyl) Ether," 1979 *Georg Thieme Publishers*.

McKillop, "A Simple and Inexpensive Procedure for Chloromethylation of Certain Aromatic Compounds," *Tetrahedron Letters*, vol. 24, No. 18, 1983, pp. 1933-1936.

Tepeletsyna, "Synthesis of Intermediates for Production of Heat Resistant Polymers (Chloromethylation of Diphenyl Oxide)," *Zhurnal Prikladnoi Khimii*, vol. 40, No. 11, Nov. 1967, pp. 2540-2546.

\* cited by examiner

**FIG. 1**



FIG. 2



FIG. 3

INK JET PRINTHEADS CONTAINING  
ARYLENE ETHER ALCOHOL POLYMERS  
AND PROCESSES FOR THEIR FORMATION

## BACKGROUND OF THE INVENTION

5

The present invention is directed to high performance polymers, processes for the preparation thereof, and articles and processes for the use thereof. More specifically, the present invention is directed to high performance polymers suitable for applications such as photoresists, microelectronic devices, ink jet printheads, and the like. One embodiment of the present invention is directed to an ink jet printhead which comprises: (i) an upper substrate, and (ii) a lower substrate in which one surface thereof has an array of heating elements and addressing electrodes formed thereon, said lower substrate having an insulative layer deposited on the surface thereof and over the heating elements and addressing electrodes and patterned to form recesses there-through to expose the heating elements and terminal ends of the addressing electrodes, said upper and lower substrates being bonded together to form a thermal ink jet printhead having droplet emitting nozzles defined by the upper substrate, the insulative layer on the lower substrate, and the heating elements in the lower substrate, wherein at least one of said upper substrate and said insulative layer comprises a crosslinked or chain extended polymer formed by crosslinking or chain extending a precursor polymer having terminal end groups and monomer repeat units, said precursor polymer being of the formula

10

20

30

35

40

45

50

55

60



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



or a mixture of



wherein R is a hydrogen atom, an alkyl group, an aryl group, or mixtures thereof, B is



**3**

wherein v is an integer of from 1 to about 20,



wherein z is an integer of from 2 to about 20,



wherein u is an integer of from 1 to about 20,



wherein w is an integer of from 1 to about 20,

**4**

-continued



5



10



25

wherein p is an integer of 0 or 1,



30

wherein t is an integer of from 1 to about 20,



35



40



45



50



55



60

wherein (1) Z is



65

5



wherein p is 0 or 1; (2) Ar is



(3) G is an alkyl group selected from alkyl or isoalkyl groups containing from about 2 to about 10 carbon atoms; (4) Ar' is



(5) X is



6



20 wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, said crosslinking or chain extension occurring through crosslinking substituents contained on at least some of the monomer repeat units of the precursor polymer.

40 Another embodiment of the present invention is directed to a process for forming an ink jet printhead which comprises: (a) providing a lower substrate in which one surface thereof has an array of heating elements and addressing electrodes having terminal ends formed thereon; (b) depositing onto the surface of the lower substrate having the heating elements and addressing electrodes thereon a layer comprising a photopatternable polymer; (c) exposing the layer to actinic radiation in an imagewise pattern such that the photopatternable polymer in exposed areas becomes crosslinked or chain extended and the photopatternable polymer in unexposed areas does not become crosslinked or chain extended, wherein the unexposed areas correspond to areas of the lower substrate having thereon the heating elements and the terminal ends of the addressing electrodes; (d) removing the photopatternable polymer from the unexposed areas, thereby forming recesses in the layer, said recesses exposing the heating elements and the terminal ends of the addressing electrodes; (e) providing an upper substrate comprising a supporting substrate and, coated thereon, a material formed by crosslinking or chain extending a composition comprising a crosslinked or chain extended polymer formed by crosslinking or chain extending a precursor polymer having terminal end groups and monomer repeat units, said precursor polymer being of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



or a mixture of



wherein R is a hydrogen atom, an alkyl group, an aryl group, or mixtures thereof, B is



-continued



35

wherein v is an integer of from 1 to about 20,



40

wherein z is an integer of from 2 to about 20,



45

wherein u is an integer of from 1 to about 20,



50

55

60

65

-continued



wherein w is an integer of from 1 to about 20,



wherein  $R_1$  and  $R_2$  each, independently of the other, are hydrogen atoms, alkyl groups, or aryl groups, and  $p$  is an integer of 0 or 1,

wherein p is 0 or 1; (2) Ar is

wherein  $t$  is an integer of from 1 to about 20,



wherein (1) Z is



wherein  $n$  is an integer of 0 or 1.



-continued



(3) G is an alkyl group selected from alkyl or isoalkyl groups containing from about 2 to about 10 carbon atoms; (4) Ar' is



,



or



(5) X is



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and (f)

bonding the upper substrate to the lower substrate to form a thermal ink jet printhead having droplet emitting nozzles defined by the upper substrate, the photopatternable polymer on the lower substrate, and the heating elements in the lower substrate.

Yet another embodiment of the present invention is directed to a process for forming an ink jet printhead which comprises: (a) depositing a layer comprising a precursor polymer having terminal end groups and monomer repeat units, said precursor polymer being of the formula



25 wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units 30 of the polymer, A is



or a mixture of



45

wherein R is a hydrogen atom, an alkyl group, an aryl group, or mixtures thereof, B is



55



60



13

-continued



wherein v is an integer of from 1 to about 20,



14

wherein z is an integer of from 2 to about 20,



10 wherein u is an integer of from 1 to about 20,



wherein w is an integer of from 1 to about 20,



**15**

5

wherein  $R_1$  and  $R_2$  each, independently of the other, are hydrogen atoms, alkyl groups, or aryl groups, and  $p$  is an integer of 0 or 1,



15

wherein  $p$  is an integer of 0 or 1,



wherein  $t$  is an integer of from 1 to about 20,



20

25

30

35

40

45

50

55

60

65

**16**

-continued

or  $-\text{Ar}-(\text{X})_p-\text{Ar}-$ wherein  $p$  is 0 or 1; (2)  $\text{Ar}$  is

or



30

35

40

45

50

55

60

65



or

(5)  $\text{X}$  is

wherein (1)  $Z$  is



-continued



wherein s is 0, 1, or 2,



and (6) q is 0 or 1; or mixtures thereof, hydroxy-substituted, 25 hydroxyalkyl-substituted, or hydroxyaryl-substituted derivatives thereof, or mixtures thereof, and n is an integer representing the number of repeating monomer units onto a lower substrate in which one surface thereof has an array of heating elements and addressing electrodes having terminal 30 ends formed thereon, said polymer being deposited onto the surface having the heating elements and addressing electrodes thereon; (b) exposing the layer to actinic radiation in an imagewise pattern such that the precursor polymer in exposed areas becomes crosslinked or chain extended and the precursor polymer in unexposed areas does not become 35 crosslinked or chain extended, wherein the unexposed areas correspond to areas of the lower substrate having thereon the heating elements and the terminal ends of the addressing electrodes; (c) removing the precursor polymer from the 40 unexposed areas, thereby forming recesses in the layer, said recesses exposing the heating elements and the terminal ends of the addressing electrodes; (d) providing an upper substrate; and (e) bonding the upper substrate to the lower 45 substrate to form a thermal ink jet printhead having droplet emitting nozzles defined by the upper substrate, the crosslinked or chain extended polymer on the lower substrate, and the heating elements in the lower substrate.

In one specific embodiment of the present invention, the 50 precursor polymer is prepared by a process which comprises (1) providing a pre-precursor polymer of the formula



wherein A is



B is



**19**

wherein v is an integer of from 1 to about 20,



wherein z is an integer of from 2 to about 20,



wherein u is an integer of from 1 to about 20,



wherein w is an integer of from 1 to about 20,

**20**

-continued

wherein R<sub>1</sub> and R<sub>2</sub> each, independently of the other, are hydrogen atoms, alkyl groups, or aryl groups, and p is an integer of 0 or 1,

25

wherein p is an integer of 0 or 1,



30



wherein t is an integer of from 1 to about 20,



35



40



45



50



55



60

wherein (1) Z is



65

21



wherein p is 0 or 1; (2) Ar is



(3) G is an alkyl group selected from alkyl or isoalkyl groups containing from about 2 to about 10 carbon atoms; (4) Ar' is



(5) X is



22



wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and (2) reacting the pre-precursor polymer with borane, resulting in formation of a precursor polymer of the formula



wherein A is



or a mixture of



60 wherein R is a hydrogen atom, an alkyl group, an aryl group, or mixtures thereof.

In another specific embodiment of the present invention, 65 the precursor polymer is prepared by a process which comprises (1) providing a pre-precursor polymer of the formula

23



5

wherein A is



B is



20



25



30



35



45



50



55



60



65



24

-continued



10



15



20

wherein v is an integer of from 1 to about 20,



30

wherein z is an integer of from 2 to about 20,



40

wherein u is an integer of from 1 to about 20,



45



50



55



60



65

**25**

wherein w is an integer of from 1 to about 20,



wherein  $R_1$  and  $R_2$  each, independently of the other, are 35 hydrogen atoms, alkyl groups, or aryl groups, and  $p$  is an integer of 0 or 1,

wherein  $p$  is an integer of 0 or 1, $-(CH_2O)_t-$ wherein  $t$  is an integer of from 1 to about 20,**26**wherein (1)  $Z$  isor  $-\text{Ar}-(X)_p-\text{Ar}-$ wherein  $p$  is 0 or 1; (2)  $\text{Ar}$  is

or



-continued  
or



;

(5) X is



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the pre-precursor polymer with a reagent of the formula  $RMgX$ , wherein R is a hydrogen atom, an alkyl group, an aryl group, or mixtures thereof and X is a halogen atom, and (3) subsequent to step 2, adding water or acid to the pre-precursor polymer, thereby resulting in formation of a precursor polymer of the formula



wherein A is



or a mixture of



15

wherein R is a hydrogen atom, an alkyl group, an aryl group, or mixtures thereof.

In microelectronics applications, there is a great need for low dielectric constant, high glass transition temperature, 20 thermally stable, photopatternable polymers for use as interlayer dielectric layers and as passivation layers which protect microelectronic circuitry. Poly(imides) are widely used to satisfy these needs; these materials, however, have disadvantageous characteristics such as relatively high water 25 sorption and hydrolytic instability. There is thus a need for high performance polymers which can be effectively photopatterned and developed at high resolution.

One particular application for such materials is the fabrication of ink jet printheads. Ink jet printing systems 30 generally are of two types: continuous stream and drop-on-demand. In continuous stream ink jet systems, ink is emitted in a continuous stream under pressure through at least one orifice or nozzle. The stream is perturbed, causing it to break up into droplets at a fixed distance from the orifice. At the 35 break-up point, the droplets are charged in accordance with digital data signals and passed through an electrostatic field which adjusts the trajectory of each droplet in order to direct it to a gutter for recirculation or a specific location on a recording medium. In drop-on-demand systems, a droplet is 40 expelled from an orifice directly to a position on a recording medium in accordance with digital data signals. A droplet is not formed or expelled unless it is to be placed on the recording medium.

Since drop-on-demand systems require no ink recovery, 45 charging, or deflection, the system is much simpler than the continuous stream type. There are different types of drop-on-demand ink jet systems. One type of drop-on-demand system has as its major components an ink filled channel or 50 passageway having a nozzle on one end and a piezoelectric transducer near the other end to produce pressure pulses. The relatively large size of the transducer prevents close spacing of the nozzles, and physical limitations of the transducer result in low ink drop velocity. Low drop velocity seriously diminishes tolerances for drop velocity variation 55 and directionality, thus impacting the system's ability to produce high quality copies. Drop-on-demand systems which use piezoelectric devices to expel the droplets also suffer the disadvantage of a slow printing speed.

The other type of drop-on-demand system is known as 60 thermal ink jet, or bubble jet, and produces high velocity droplets and allows very close spacing of nozzles. The major components of this type of drop-on-demand system are an ink filled channel having a nozzle on one end and a heat generating resistor near the nozzle. Printing signals representing digital information originate an electric current pulse 65 in a resistive layer within each ink passageway near the orifice or nozzle, causing the ink in the immediate vicinity

to vaporize almost instantaneously and create a bubble. The ink at the orifice is forced out as a propelled droplet as the bubble expands. When the hydrodynamic motion of the ink stops, the process is ready to start all over again. With the introduction of a droplet ejection system based upon thermally generated bubbles, commonly referred to as the "bubble jet" system, the drop-on-demand ink jet printers provide simpler, lower cost devices than their continuous stream counterparts, and yet have substantially the same high speed printing capability.

The operating sequence of the bubble jet system begins with a current pulse through the resistive layer in the ink filled channel, the resistive layer being in close proximity to the orifice or nozzle for that channel. Heat is transferred from the resistor to the ink. The ink becomes superheated far above its normal boiling point, and for water based ink, finally reaches the critical temperature for bubble formation or nucleation of around 280° C. Once nucleated, the bubble or water vapor thermally isolates the ink from the heater and no further heat can be applied to the ink. This bubble expands until all the heat stored in the ink in excess of the normal boiling point diffuses away or is used to convert liquid to vapor, which removes heat due to heat of vaporization. The expansion of the bubble forces a droplet of ink out of the nozzle, and once the excess heat is removed, the bubble collapses. At this point, the resistor is no longer being heated because the current pulse has passed and, concurrently with the bubble collapse, the droplet is propelled at a high rate of speed in a direction towards a recording medium. The surface of the printhead encounters a severe cavitation force by the collapse of the bubble, which tends to erode it. Subsequently, the ink channel refills by capillary action. This entire bubble formation and collapse sequence occurs in about 10 microseconds. The channel can be refired after 100 to 500 microseconds minimum dwell time to enable the channel to be refilled and to enable the dynamic refilling factors to become somewhat damped. Thermal ink jet equipment and processes are well known and are described in, for example, U.S. Pat. No. 4,601,777, U.S. Pat. No. 4,251,824, U.S. Pat. No. 4,410,899, U.S. Pat. No. 4,412,224, U.S. Pat. No. 4,532,530, and U.S. Pat. No. 4,774,530, the disclosures of each of which are totally incorporated herein by reference.

The present invention is suitable for ink jet printing processes, including drop-on-demand systems such as thermal ink jet printing, piezoelectric drop-on-demand printing, and the like.

In ink jet printing, a printhead is usually provided having one or more ink-filled channels communicating with an ink supply chamber at one end and having an opening at the opposite end, referred to as a nozzle. These printheads form images on a recording medium such as paper by expelling droplets of ink from the nozzles onto the recording medium. The ink forms a meniscus at each nozzle prior to being expelled in the form of a droplet. After a droplet is expelled, additional ink surges to the nozzle to reform the meniscus.

In thermal ink jet printing, a thermal energy generator, usually a resistor, is located in the channels near the nozzles a predetermined distance therefrom. The resistors are individually addressed with a current pulse to momentarily vaporize the ink and form a bubble which expels an ink droplet. As the bubble grows, the ink bulges from the nozzle and is contained by the surface tension of the ink as a meniscus. The rapidly expanding vapor bubble pushes the column of ink filling the channel towards the nozzle. At the end of the current pulse the heater rapidly cools and the vapor bubble begins to collapse. However, because of

inertia, most of the column of ink that received an impulse from the exploding bubble continues its forward motion and is ejected from the nozzle as an ink drop. As the bubble begins to collapse, the ink still in the channel between the nozzle and bubble starts to move towards the collapsing bubble, causing a volumetric contraction of the ink at the nozzle and resulting in the separation of the bulging ink as a droplet. The acceleration of the ink out of the nozzle while the bubble is growing provides the momentum and velocity of the droplet in a substantially straight line direction towards a recording medium, such as paper.

Ink jet printheads include an array of nozzles and may, for example, be formed of silicon wafers using orientation dependent etching (ODE) techniques. The use of silicon wafers is advantageous because ODE techniques can form structures, such as nozzles, on silicon wafers in a highly precise manner. Moreover, these structures can be fabricated efficiently at low cost. The resulting nozzles are generally triangular in cross-section. Thermal ink jet printheads made by using the above-mentioned ODE techniques typically comprise a channel plate which contains a plurality of nozzle-defining channels located on a lower surface thereof bonded to a heater plate having a plurality of resistive heater elements formed on an upper surface thereof and arranged so that a heater element is located in each channel. The upper surface of the heater plate typically includes an insulative layer which is patterned to form recesses exposing the individual heating elements. This insulative layer is referred to as a "pit layer" and is sandwiched between the channel plate and heater plate. For examples of printheads employing this construction, see U.S. Pat. No. 4,774,530 and U.S. Pat. No. 4,829,324, the disclosures of each of which are totally incorporated herein by reference. Additional examples of thermal ink jet printheads are disclosed in, for example, U.S. Pat. No. 4,835,553, U.S. Pat. No. 5,057,853, and U.S. Pat. No. 4,678,529, the disclosures of each of which are totally incorporated herein by reference.

The photopatternable polymers of the present invention are also suitable for other photoresist applications, including other microelectronics applications, printed circuit boards, lithographic printing processes, interlayer dielectrics, and the like.

The formation and development of images on the surface of photoconductive materials by electrostatic means is well known. The basic electrophotographic imaging process, as taught by C. F. Carlson in U.S. Pat. No. 2,297,691, entails placing a uniform electrostatic charge on a photoconductive imaging member, exposing the imaging member to a light and shadow image to dissipate the charge on the areas of the imaging member exposed to the light, and developing the resulting electrostatic latent image by depositing on the image a finely divided electroscopic material known as toner. In charge area development (CAD) systems, the toner will normally be attracted to those areas of the imaging member which retain a charge, thereby forming a toner image corresponding to the electrostatic latent image. In discharge area development (DAD) systems, the toner will normally be attracted to those areas of the imaging member which have less or no charge as a result of exposure to light, thereby forming a toner image corresponding to the electrostatic latent image. This developed image may then be transferred to a substrate such as paper. The transferred image may subsequently be permanently affixed to the substrate by heat, pressure, a combination of heat and pressure, or other suitable fixing means such as solvent or overcoating treatment.

Imaging members for electrophotographic imaging systems comprising selenium alloys vacuum deposited on sub-

substrates are known. Imaging members have also been prepared by coating substrates with photoconductive particles dispersed in an organic film forming binder. Coating of rigid drum substrates has been effected by various techniques such as spraying, dip coating, vacuum evaporation, and the like. Flexible imaging members can also be manufactured by processes that entail coating a flexible substrate with the desired photoconducting material.

Some photoresponsive imaging members consist of a homogeneous layer of a single material such as vitreous selenium, and others comprise composite layered devices containing a dispersion of a photoconductive composition. An example of a composite xerographic photoconductive member is described in U.S. Pat. No. 3,121,006, which discloses finely divided particles of a photoconductive inorganic compound dispersed in an electrically insulating organic resin binder. Imaging members prepared according to the teachings of this patent contain a binder layer with particles of zinc oxide uniformly dispersed therein coated on a paper backing. The binders disclosed in this patent include materials such as polycarbonate resins, polyester resins, polyamide resins, and the like.

Photoreceptor materials comprising inorganic or organic materials wherein the charge generating and charge transport functions are performed by discrete contiguous layers are also known. Additionally, layered photoreceptor members are disclosed in the prior art, including photoreceptors having an overcoat layer of an electrically insulating polymeric material. Other layered photoresponsive devices have been disclosed, including those comprising separate photo-generating layers and charge transport layers as described in U.S. Pat. No. 4,265,990, the disclosure of which is totally incorporated herein by reference. Photoresponsive materials containing a hole injecting layer overcoated with a hole transport layer, followed by an overcoating of a photogenerating layer, and a top coating of an insulating organic resin, are disclosed in U.S. Pat. No. 4,251,612, the disclosure of which is totally incorporated herein by reference. Examples of photogenerating layers disclosed in these patents include trigonal selenium and phthalocyanines, while examples of transport layers include certain aryl diamines as illustrated therein.

In addition, U.S. Pat. No. 3,041,167 discloses an overcoated imaging member containing a conductive substrate, a photoconductive layer, and an overcoating layer of an electrically insulating polymeric material. This member can be employed in electrophotographic imaging processes by initially charging the member with an electrostatic charge of a first polarity, followed by exposing it to form an electrostatic latent image that can subsequently be developed to form a visible image.

U.S. Pat. No. 3,914,194 (Smith), the disclosure of which is totally incorporated herein by reference, discloses a formaldehyde copolymer resin having dependent unsaturated groups with the repeating unit



wherein R is an aliphatic acyl group derived from saturated acids having 2 to 6 carbons, olefinically unsaturated acids having 3 to 20 carbons, or an omega-carboxy-aliphatic acyl

group derived from olefinically unsaturated dicarboxylic acids having 4 to 12 carbons or mixtures thereof, R<sub>1</sub> is independently hydrogen, an alkyl group of 1 to 10 carbon atoms, or halogen, Z is selected from oxygen, sulfur, the group represented by Z taken with the dotted line represents dibenzofuran and dibenzothiophene moieties, or mixtures thereof, n is a whole number sufficient to give a weight average molecular weight greater than about 500, m is 0 to 2, p and q have an average value of 0 to 1 with the proviso that the total number of p and q groups are sufficient to give greater than one unsaturated group per resin molecule. These resins are useful to prepare coatings on various substrates or for potting electrical components by mixing with reactive diluents and curing agents and curing.

“Chloromethylation of Condensation Polymers Containing an oxy-1,4-phenylene Backbone,” W. H. Daly et al., *Polymer Preprints*, Vol. 20, No. 1, 835 (1979), the disclosure of which is totally incorporated herein by reference, discloses the chloromethylation of polymers containing oxy-phenylene repeat units to produce film forming resins with high chemical reactivity. The utility of 1,4-bis (chloromethoxy) butane and 1-chloromethoxy-4-chlorobutane as chloromethylating agents are also described.

European Patent Application EP-0,698,823-A1 (Fahey et al.), the disclosure of which is totally incorporated herein by reference, discloses a copolymer of benzophenone and bisphenol A which was shown to have deep ultraviolet absorption properties. The copolymer was found useful as an antireflective coating in microlithography applications.

Incorporating anthracene into the copolymer backbone enhanced absorption at 248 nm. The encapper used for the copolymer varied depending on the needs of the user and was selectable to promote adhesion, stability, and absorption of different wavelengths.

M. Camps, M. Chatzopoulos, and J. Montheard, “Chloromethyl Styrene: Synthesis, Polymerization, Transformations, Applications,” *JMS—Rev. Macromol. Chem. Phys.*, C22(3), 343–407 (1982–3), the disclosure of which is totally incorporated herein by reference, discloses processes for the preparation of chloromethyl-substituted polystyrenes, as well as applications thereof.

Y. Tabata, S. Tagawa, and M. Washio, “Pulse Radiolysis Studies on the Mechanism of the High Sensitivity of Chloromethylated Polystyrene as an Electron Negative Resist,” *Lithography*, 25(1), 287 (1984), the disclosure of which is totally incorporated herein by reference, discloses the use of chloromethylated polystyrene in resist applications.

M. J. Jurek, A. E. Novembre, I. P. Heyward, R. Gooden, and E. Reichmanis, “Deep UV Photochemistry of Copolymers of Trimethyl-Silylmethyl Methacrylate and Chloromethylstyrene,” *Polymer Preprints*, 29(1) (1988), the disclosure of which is totally incorporated herein by reference, discloses the use of an organosilicon polymer of chloromethylstyrene for resist applications.

P. M. Hergenrother, B. J. Jensen, and S. J. Havens, “Poly(arylene ethers),” *Polymer*, 29, 358 (1988), the disclosure of which is totally incorporated herein by reference, discloses several arylene ether homopolymers and copolymers prepared by the nucleophilic displacement of aromatic

dihalides with aromatic potassium bisphenates. Polymer glass transition temperatures ranged from 114 to 310° C. and some were semicrystalline. Two ethynyl-terminated poly(arylene ethers) were synthesized by reacting hydroxy-terminated oligomers with 4-ethynylbenzoyl chloride. Heat induced reaction of the acetylenic groups provided materials with good solvent resistance. The chemistry, physical, and mechanical properties of the polymers are also disclosed.

S. J. Havens, "Ethynyl-Terminated Polyarylates: Synthesis and Characterization," *Journal of Polymer Science: Polymer Chemistry Edition*, vol. 22, 3011–3025 (1984), the disclosure of which is totally incorporated herein by reference, discloses hydroxy-terminated polyarylates with number average molecular weights of about 2500, 5000, 7500, and 10,000 which were synthesized and converted to corresponding 4-ethynylbenzoyloxy-terminated polyarylates by reaction with 4-ethynylbenzoyl chloride. The terminal ethynyl groups were thermally reacted to provide chain extension and crosslinking. The cured polymer exhibited higher glass transition temperatures and better solvent resistance than a high molecular weight linear polyarylate. Solvent resistance was further improved by curing 2,2-bis (4-ethynylbenzoyloxy-4'-phenyl)propane, a coreactant, with the ethynyl-terminated polymer at concentrations of about 10 percent by weight.

N. H. Hendricks and K. S. Y. Lau, "Flare, a Low Dielectric Constant, High T<sub>g</sub>, Thermally Stable Poly(arylene ether) Dielectric for Microelectronic Circuit Interconnect Process Integration: Synthesis, Characterization, Thermomechanical Properties, and Thin-Film Processing Studies," *Polymer Preprints*, 37(1), 150 (1996), the disclosure of which is totally incorporated herein by reference, discloses non-carbonyl containing aromatic polyethers such as fluorinated poly(arylene ethers) based on decafluorobiphenyl as a class of intermetal dielectrics for applications in sub-half micron multilevel interconnects.

J. J. Zupancic, D. C. Blazej, T. C. Baker, and E. A. Dinkel, "Styrene Terminated Resins as Interlevel Dielectrics for Multichip Models," *Polymer Preprints*, 32, (2), 178 (1991), the disclosure of which is totally incorporated herein by reference, discloses vinylbenzyl ethers of polyphenols (styrene terminated resins) which were found to be photochemically and thermally labile, generating highly crosslinked networks. The resins were found to yield no volatile by-products during the curing process and high glass transition, low dielectric constant coatings. One of the resins was found to be spin coatable to varying thickness coatings which could be photodefined, solvent developed, and then hard baked to yield an interlevel dielectric.

Japanese Patent Kokai JP 04294148-A, the disclosure of which is totally incorporated herein by reference, discloses a liquid injecting recording head containing the cured matter of a photopolymerizable composition comprising (1) a graft polymer comprising (A) alkyl methacrylate, acrylonitrile, and/or styrene as the trunk chain and an —OH group-containing acryl monomer, (B) amino or alkylamino group-containing acryl monomer, (C) carboxyl group-containing acryl or vinyl monomers, (D) N-vinyl pyrrolidone, vinyl pyridine or its derivatives, and/or (F) an acrylamide as the side chain; (2) a linear polymer containing constitutional units derived from methyl methacrylate, ethyl methacrylate, isobutyl methacrylate, t-butyl methacrylate, benzyl methacrylate, acrylonitrile, isobornyl methacrylate, tricyclodecane acrylate, tricyclodecane oxyethyl methacrylate, styrene, dimethylaminoethyl methacrylate, and/or cyclohexyl methacrylate, and constitutional unit derived from the above compounds (A), (B), (C), (D), (E), or (F) above; (3) an ethylenic unsaturated bond containing monomer; and (4) a photopolymerization initiator which contains (a) an organic peroxide, s-triazine derivative, benzophenone or its derivatives, quinones, N-phenylglycine, and/or alkylarylketones as a radical generator and (b) coumarin dyes, keto-coumarin dyes, cyanine dyes, merocyanine dyes, and/or xanthene dyes as a sensitizer.

"Functional Polymers and Sequential Copolymers by Phase Transfer Catalysis, 2a: Synthesis and Characterization

of Aromatic Poly(ether sulfone)s Containing Vinylbenzyl and Ethynylbenzyl Chain Ends," V. Percec and B. C. Auman, *Makromol. Chem.*, 185, 1867–1880 (1984), the disclosure of which is totally incorporated herein by reference, discloses a method for the synthesis of  $\alpha,\omega$ -bis(vinylbenzyl) aromatic poly(ether sulfone)s and their transformation into  $\alpha,\omega$ -bis(ethynylbenzyl) aromatic poly(ether sulfone)s. The method entails a fast and quantitative Williamson etherification of the  $\alpha,\omega$ -bis(hydroxyphenyl) polysulfone with a mixture of p- and m-chloromethylstyrenes in the presence of tetrabutylammonium hydrogen sulfate as phase transfer catalyst, a subsequent bromination, and then a dehydrobromination with potassium tert-butoxide. The DSC study of the thermal curing of the  $\alpha,\omega$ -bis(vinylbenzyl) aromatic poly(ether sulfone)s and  $\alpha,\omega$ -bis(ethynylbenzyl) aromatic poly(ether sulfone)s demonstrates high thermal reactivity for the styrene-terminated oligomers.

"Functional Polymers and Sequential Copolymers by Phase Transfer Catalysis, 3a: Synthesis and Characterization of Aromatic Poly(ether sulfone)s and Poly(oxy-2,6-dimethyl-1,4-phenylene) Containing Pendent Vinyl Groups," V. Percec and B. C. Auman, *Makromol. Chem.*, 185, 2319–2336 (1984), the disclosure of which is totally incorporated herein by reference, discloses a method for the syntheses of  $\alpha,\omega$ -benzyl aromatic poly(ether sulfone)s (PSU) and poly(oxy-2,6-dimethyl-1,4-phenylene) (POP) containing pendant vinyl groups. The first step of the synthetic procedure entails the chloromethylation of PSU and POP to provide polymers with chloromethyl groups. POP, containing bromomethyl groups, was obtained by radical bromination of the methyl groups. Both chloromethylated and bromomethylated starting materials were transformed into their phosphonium salts, and then subjected to a phase transfer catalyzed Wittig reaction to provide polymers with pendant vinyl groups. A PSU with pendant ethynyl groups was prepared by bromination of the PSU containing vinyl groups, followed by a phase transfer catalyzed dehydrobromination. DSC of the thermal curing of the polymers containing pendant vinyl and ethynyl groups showed that the curing reaction is much faster for the polymers containing vinyl groups. The resulting network polymers are flexible when the starting polymer contains vinyl groups, and very rigid when the starting polymer contains ethynyl groups.

"Functional Polymers and Sequential Copolymers by Phase Transfer Catalysis," V. Percec and P. L. Rinaldi, *Polymer Bulletin*, 10, 223 (1983), the disclosure of which is totally incorporated herein by reference, discloses the preparation of p- and m-hydroxymethylphenylacetylenes by a two step sequence starting from a commercial mixture of p- and m-chloromethylstyrene, i.e., by the bromination of the vinylic monomer mixture followed by separation of m- and p-brominated derivatives by fractional crystallization, and simultaneous dehydrobromination and nucleophilic substitution of the —Cl with —OH.

U.S. Pat. No. 4,110,279 (Nelson et al.), the disclosure of which is totally incorporated herein by reference, discloses a polymer derived by heating in the presence of an acid catalyst at between about 65° C. and about 250° C.: I. a reaction product, a cogeneric mixture of alkoxy functional compounds, having average equivalent weights in the range of from about 220 to about 1200, obtained by heating in the presence of a strong acid at about 50° C. to about 250° C.: (A) a diaryl compound selected from naphthalene, diphenyl oxide, diphenyl sulfide, their alkylated or halogenated derivatives, or mixtures thereof, (B) formaldehyde or form-aldehyde yielding derivative, (C) water, and (D) a hydroxy

aliphatic hydrocarbon compound having at least one free hydroxyl group and from 1 to 4 carbon atoms, which mixture contains up to 50 percent unreacted (A); with II. at least one monomeric phenolic reactant selected from the group



wherein R is selected from the group consisting of hydrogen, alkyl radical of 1 to 20 carbon atoms, aryl radical of 6 to 20 carbon atoms, wherein R<sub>1</sub> represents hydrogen, alkyl, or aryl, m represents an integer from 1 to 3, o represents an integer from 1 to 5, p represents an integer from 0 to 3, X represents oxygen, sulfur, or alkylidene, and q represents an integer from 0 to 1; and III. optionally an aldehyde or aldehyde-yielding derivative or ketone, for from several minutes to several hours. The polymeric materials are liquids or low melting solids which are capable of further modification to thermoset resins. These polymers are capable of being thermoset by heating at a temperature of from about 130° C. to about 260° C. for from several minutes to several hours in the presence of a formaldehyde-yielding compound. These polymers are also capable of further modification by reacting under basic conditions with formaldehyde with or without a phenolic compound. The polymers, both base catalyzed resoles and acid catalyzed novolacs, are useful as laminating, molding, film-forming, and adhesive materials. The polymers, both resoles and novolacs, can be epoxidized as well as reacted with a drying oil to produce a varnish resin.

U.S. Pat. No. 3,367,914 (Herbert), the disclosure of which is totally incorporated herein by reference, discloses thermosetting resinous materials having melting points in the range of from 150° C. to 350° C. which are made heating at a temperature of from -10° C. to 100° C. for 5 to 30 minutes an aldehyde such as formaldehyde or acetaldehyde with a mixture of poly(aminomethyl) diphenyl ethers having an average of from about 1.5 to 4.0 aminomethyl groups. After the resins are cured under pressure at or above the melting point, they form adherent tough films on metal substrates and thus are useful as wire coatings for electrical magnet wire for high temperature service at 180° C. or higher.

J. S. Amato, S. Karady, M. Sletzinger, and L. M. Weinstock, "A New Preparation of Chloromethyl Methyl Ether Free of Bis(chloromethyl) Ether," *Synthesis*, 970 (1979), the disclosure of which is totally incorporated herein by reference, discloses the synthesis of chloromethyl methyl ether by the addition of acetyl chloride to a slight excess of anhydrous dimethoxymethane containing a catalytic amount of methanol at room temperature. The methanol triggers a series of reactions commencing with formation of hydrogen chloride and the reaction of hydrogen chloride with dimethoxymethane to form chloromethyl methyl ether and methanol in an equilibrium process. After 36 hours, a near-quantitative conversion to an equimolar mixture of chloromethyl methyl ether and methyl acetate is obtained.

A. McKillop, F. A. Madjdabadi, and D. A. Long, "A Simple and Inexpensive Procedure for Chloromethylation of Certain Aromatic Compounds," *Tetrahedron Letters*, Vol. 24, No. 18, pp. 1933-1936 (1983), the disclosure of which is totally incorporated herein by reference, discloses the

reaction of a range of aromatic compounds with methoxyacetyl chloride and aluminum chloride in either nitromethane or carbon disulfide to result in chloromethylation in good to excellent yield.

E. P. Tepenitsyna, M. I. Farberov, and A. P. Ivanovskii, "Synthesis of Intermediates for Production of Heat Resistant Polymers (Chloromethylation of Diphenyl Oxide)," *Zhurnal Prikladnoi Khimii*, Vol. 40, No. 11, pp. 2540-2546 (1967), the disclosure of which is totally incorporated herein by reference, discloses the chloromethylation of diphenyl oxide by (1) the action of paraformaldehyde solution in glacial acetic acid saturated with hydrogen chloride, and by (2) the action of paraformaldehyde solution in concentrated hydrochloric acid.

U.S. Pat. No. 2,125,968 (Theimer), the disclosure of which is totally incorporated herein by reference, discloses the manufacture of aromatic alcohols by the Friedel-Crafts reaction, in which an alkylene oxide is condensed with a Friedel-Crafts reactant in the presence of an anhydrous metal halide.

Copending application U.S. Ser. No. 08/705,375, filed Aug. 29, 1996, now U.S. Pat. No. 5,994,425, entitled "Curable Compositions Containing Photosensitive High Performance Aromatic Ether Polymers," and Copending application U.S. Ser. No. 09/221,024, filed Dec. 23, 1998, now U.S. Pat. No. 6,022,095, entitled "Curable Compositions," with the named inventors Timothy J. Fuller, Ram S. Narang, Thomas W. Smith, David J. Luca, and Ralph A. Mosher, the disclosures of each of which are totally incorporated herein by reference, disclose an improved composition comprising a photopatternable polymer containing at least some monomer repeat units with photosensitivity-imparting substituents, said photopatternable polymer being of the general formula



wherein x is an integer of 0 or 1, A is one of several specified groups, such as



B is one of several specified groups, such as



or mixtures thereof, and n is an integer representing the number of repeating monomer units. Also disclosed is a process for preparing a thermal ink jet printhead with the aforementioned polymer and a thermal ink jet printhead containing therein a layer of a crosslinked or chain extended polymer of the above formula.

U.S. Pat. No. 5,849,809, filed Aug. 29, 1996, and Copending application U.S. Ser. No. 09/159,426, filed Sep. 23, 1998, entitled "Hydroxyalkylated High Performance Curable Polymers," with the named inventors Ram S. Narang and Timothy J. Fuller, the disclosures of each of which are totally incorporated herein by reference, disclose a composition which comprises (a) a polymer containing at least some monomer repeat units with photosensitivity-imparting substituents which enable crosslinking or chain extension of the polymer upon exposure to actinic radiation, said polymer being of the formula



wherein x is an integer of 0 or 1, A is one of several specified groups, such as



39

Direct Substitution of High Performance Polymers with Unsaturated Ester Groups," with the named inventors Timothy J. Fuller, Ram S. Narang, Thomas W. Smith, David J. Luca, and Raymond K. Crandall, the disclosures of each of which are totally incorporated herein by reference, disclose a process which comprises reacting a polymer of the general formula



W. Smith, David J. Luca, and Raymond K. Crandall, the disclosures of each of which are totally incorporated herein by reference, disclose a process which comprises reacting a polymer of the general formula

40

5



wherein x is an integer of 0 or 1, A is one of several specified groups, such as



25

B is one of several specified groups, such as



30

B is one of several specified groups, such as



35



40



45



50

or mixtures thereof, and n is an integer representing the number of repeating monomer units, with an acetyl halide and dimethoxymethane in the presence of a halogen-containing Lewis acid catalyst and methanol, thereby forming a haloalkylated polymer. In a specific embodiment, the 60 haloalkylated polymer is then reacted further to replace at least some of the haloalkyl groups with photosensitivity-imparting groups. Also disclosed is a process for preparing a thermal ink jet printhead with the aforementioned polymer.

U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas

or mixtures thereof, and n is an integer representing the number of repeating monomer units, with (i) a formaldehyde source, and (ii) an unsaturated acid in the presence of an acid catalyst, thereby forming a curable polymer with unsaturated ester groups. Also disclosed is a process for preparing an ink jet printhead with the above polymer.

U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas

65

S. Narang, Thomas W. Smith, David J. Luca, and Raymond K. Crandall, the disclosure of which is totally incorporated herein by reference, discloses a process which comprises reacting a haloalkylated aromatic polymer with a material selected from the group consisting of unsaturated ester salts, alkoxide salts, alkylcarboxylate salts, and mixtures thereof, thereby forming a curable polymer having functional groups corresponding to the selected salt. Another embodiment of the invention is directed to a process for preparing an ink jet printhead with the curable polymer thus prepared.

Copending application U.S. Ser. No. 08/705,376, filed Aug. 29, 1996, now U.S. Pat. No. 5,958,995, entitled "Blends Containing Photosensitive High Performance Aromatic Ether Curable Polymers," and Copending application U.S. Ser. No. 09/220,273, filed Dec. 23, 1998, entitled "Blends Containing Curable Polymers," with the named inventors Ram S. Narang and Timothy J. Fuller, the disclosures of each of which are totally incorporated herein by reference, disclose a composition which comprises a mixture of (A) a first component comprising a polymer, at least some of the monomer repeat units of which have at least one photosensitivity-imparting group thereon, said polymer having a first degree of photosensitivity-imparting group substitution measured in milliequivalents of photosensitivity-imparting group per gram and being of the general formula



wherein x is an integer of 0 or 1, A is one of several specified groups, such as



B is one of several specified groups, such as



-continued



or mixtures thereof, and n is an integer representing the number of repeating monomer units, and (B) a second component which comprises either (1) a polymer having a second degree of photosensitivity-imparting group substitution measured in milliequivalents of photosensitivity-imparting group per gram lower than the first degree of photosensitivity-imparting group substitution, wherein said second degree of photosensitivity-imparting group substitution may be zero, wherein the mixture of the first component and the second component has a third degree of photosensitivity-imparting group substitution measured in milliequivalents of photosensitivity-imparting group per gram which is lower than the first degree of photosensitivity-imparting group substitution and higher than the second degree of photosensitivity-imparting group substitution, or (2) a reactive diluent having at least one photosensitivity-imparting group per molecule and having a fourth degree of photosensitivity-imparting group substitution measured in milliequivalents of photosensitivity-imparting group per gram, wherein the mixture of the first component and the second component has a fifth degree of photosensitivity-imparting group substitution measured in milliequivalents of photosensitivity-imparting group per gram which is higher than the first degree of photosensitivity-imparting group substitution and lower than the fourth degree of photosensitivity-imparting group substitution; wherein the weight average molecular weight of the mixture is from about 10,000 to about 50,000; and wherein the third or fifth degree of photosensitivity-imparting group substitution is from about 0.25 to about 2 milliequivalents of photosensitivity-imparting groups per gram of mixture. Also disclosed is a process for preparing a thermal ink jet print-head with the aforementioned composition.

Copending application U.S. Ser. No. 08/705,372, filed Aug. 29, 1996, now U.S. Pat. No. 5,945,253, and Copending application U.S. Ser. No. 09/246,167, filed Feb. 8, 1999, now abandoned entitled "High Performance Curable Polymers and Processes for the Preparation Thereof," with the named inventors Ram S. Narang and Timothy J. Fuller, the disclosures of each of which are totally incorporated herein by reference, disclose a composition which comprises a polymer containing at least some monomer repeat units with photosensitivity-imparting substituents which enable crosslinking or chain extension of the polymer upon exposure to actinic radiation, said polymer being of the formula

43



wherein x is an integer of 0 or 1, A is one of several specified groups, such as



B is one of several specified groups, such as



or mixtures thereof, and n is an integer representing the number of repeating monomer units, wherein said photosensitivity-imparting substituents are allyl ether groups, epoxy groups, or mixtures thereof. Also disclosed are a process for preparing a thermal ink jet printhead containing the aforementioned polymers and processes for preparing the aforementioned polymers.

U.S. Pat. No. 5,863,963, filed Aug. 29, 1996, and Copending application U.S. Ser. No. 09/163,672, filed Sep. 30, 1998, now U.S. Pat. No. 6,090,453, entitled "Halomethylated High Performance Curable Polymers," with the named inventors Ram S. Narang and Timothy J. Fuller, the disclosures of each of which are totally incorporated herein by reference, disclose a process which comprises the steps of (a) providing a polymer containing at least some monomer repeat units with halomethyl group substituents which enable crosslinking or chain extension of the polymer upon

44

exposure to a radiation source which is electron beam radiation, x-ray radiation, or deep ultraviolet radiation, said polymer being of the formula



wherein x is an integer of 0 or 1, A is one of several specified groups, such as



25 B is one of several specified groups, such as



or mixtures thereof, and n is an integer representing the number of repeating monomer units, and (b) causing the polymer to become crosslinked or chain extended through the photosensitivity-imparting groups. Also disclosed is a process for preparing a thermal ink jet printhead by the aforementioned curing process.

60 Copending application U.S. Ser. No. 08/697,760, filed Aug. 29, 1996, now U.S. Pat. No. 6,007,877, entitled "Aqueous Developable High Performance Curable Aromatic Ether Polymers," and Copending application U.S. Ser. No. 09/247,104, filed Feb. 9, 1999, entitled "Aqueous Developable High Performance Curable Polymers," with the named inventors Ram S. Narang and Timothy J. Fuller, the disclosures of each of which are totally incorporated herein

45

by reference, disclose a composition which comprises a polymer containing at least some monomer repeat units with water-solubility-imparting substituents and at least some monomer repeat units with photosensitivity-imparting substituents which enable crosslinking or chain extension of the polymer upon exposure to actinic radiation, said polymer being of the formula



46

-continued



wherein x is an integer of 0 or 1, A is one of several specified groups, such as



B is one of several specified groups, such as



20 or mixtures thereof, and n is an integer representing the number of repeating monomer units. In one embodiment, a single functional group imparts both photosensitivity and water solubility to the polymer. In another embodiment, a 25 first functional group imparts photosensitivity to the polymer and a second functional group imparts water solubility to the polymer. Also disclosed is a process for preparing a thermal ink jet printhead with the aforementioned polymers.

30

U.S. Pat. No. 5,814,426, filed Nov. 21, 1997, entitled "Imaging Members Containing High Performance Polymers," with the named inventors Kathleen M. Carmichael, Timothy J. Fuller, Edward F. Grabowski, Damodar M. Pai, Leon A. Teuscher, John F. Yanus, and Paul F. Zukoski, the disclosure of which is totally incorporated herein by reference, discloses an imaging member which 35 comprises a conductive substrate, a photogenerating material, and a binder which comprises a polymer of the 40 formulae I, II, III, IV, V, VI, VII, VIII, IX, or X:

I



II



-continued

III



IV



V



VI



-continued



VII



VIII



IX





25

wherein x is an integer of 0 or 1, A is



30



35



40



45



or mixtures thereof, B is



50



55



60



65

53

-continued



wherein v is an integer of from 1 to about 20,

—(CH<sub>2</sub>O)<sub>t</sub>—

wherein t is an integer of from 1 to about 20,



54

wherein z is an integer of from 2 to about 20,



10 wherein u is an integer of from 1 to about 20,



wherein w is an integer of from 1 to about 20,



**55****56**

or mixtures thereof, C is



or mixtures thereof, wherein R is an alkyl group, an aryl group, an arylalkyl group, or mixtures thereof, and m and n are integers representing the number of repeating units.

20

U.S. Pat. No. 5,882,814, filed Nov. 21, 1997, entitled "Imaging Members Containing High Performance Charge Transporting Polymers," with the named inventors Timothy 25 J. Fuller, Damodar M. Pai, Leon A. Teuscher, and John F. Yanus, the disclosure of which is totally incorporated herein by reference, discloses an imaging member which comprises a conductive substrate, a photogenerating layer, and a charge transport layer comprising a polymer of the formulae I, II, III, IV, V, VI, VII, VIII, IX, or X:

I



II



III



-continued

IV



V



VI



VII



-continued



VIII



IX



X



61

wherein x is an integer of 0 or 1, A is



or mixtures thereof. B is



62

-continued

H<sub>3</sub>C



wherein v is an integer of from 1 to about 20,

65

$$-\text{-(CH}_2\text{O)}_i\text{-}$$

**63**

wherein t is an integer of from 1 to about 20,



wherein z is an integer of from 2 to about 20,



wherein u is an integer of from 1 to about 20,



wherein w is an integer of from 1 to about 20,

**64**

-continued



35 wherein (1) Z is



or —Ar—(X)p—Ar—

60 wherein p is 0 or 1; (2) Ar is



-continued



or



(3) G is an alkyl group selected from alkyl or isoalkyl groups containing from about 2 to about 10 carbon atoms; (4) Ar' is

15



or



(5) X is



wherein s is 0, 1, or 2,



10 and (6) q is 0 or 1; or mixtures thereof, wherein at least some of the "B" groups are of the formula



C is



45 or mixtures thereof, wherein R is an alkyl group, an aryl group, an arylalkyl group, or mixtures thereof, and m and n are integers representing the number of repeating units.

50 U.S. Pat. No. 5,874,192, filed Nov. 21, 1997, entitled "Imaging Members with Charge Transport Layers Containing High Performance Polymer Blends," with the named inventors Kathleen M. Carmichael, Timothy J. Fuller, Edward F. Grabowski, Damodar M. Pai, Leon A. Teuscher, John F. Yanus, and Paul F. Zukoski, the disclosure of which is totally incorporated herein by reference, discloses an 55 imaging member which comprises a conductive substrate, a photogenerating material, a charge transport material, and a polymeric binder comprising (a) a first polymer comprising a polycarbonate, and (b) a second polymer of the formulae I, II, III, IV, V, VI, VII, VIII, IX, or X:





-continued



X



35

wherein x is an integer of 0 or 1, A is



-continued



40



45



50



55



60



65

73

-continued



or mixtures thereof, B is



74

-continued



20 wherein v is an integer of from 1 to about 20,  
 $-(CH_2O)_t-$

wherein t is an integer of from 1 to about 20,



30 wherein z is an integer of from 2 to about 20,



35 wherein u is an integer of from 1 to about 20,



65

75

wherein w is an integer of from 1 to about 20,



76

-continued



10 or mixtures thereof, wherein R is an alkyl group, an aryl group, an arylalkyl group, or mixtures thereof, and m and n are integers representing the numbers of repeating units.

Copending application U.S. Ser. No. 09/105,501, filed Jun. 26, 1998, entitled "Bonding Process," with the named inventors Lisa A. DeLouise and David J. Luca, the disclosure of which is totally incorporated herein by reference, 15 discloses a process for bonding a first article to a second article which comprises (a) providing a first article comprising a polymer having photosensitivity-imparting substituents; (b) providing a second article comprising metal, plasma nitride, silicon, or glass; (c) applying to at least one 20 of the first article and the second article an adhesion promoter selected from silanes, titanates, or zirconates having (i) alkoxy, aryloxy, or arylalkyloxy functional groups and (ii) functional groups including at least one photosensitive aliphatic  $>C=C<$  linkage; (d) placing the first article in 25 contact with the second article; and (e) exposing the first article, second article, and adhesion promoter to radiation, thereby bonding the first article to the second article with the adhesion promoter. In one embodiment of the present invention, the adhesion promoter is employed in microelectrical mechanical systems such as thermal ink jet printheads.

Copending application U.S. Ser. No. 09/120,746, filed Jul. 23, 1998, entitled "Improved Thermal Ink Jet Printhead and Process for the Preparation Thereof," with the named inventors Ram S. Narang, Gary A. Kneezel, Bidan Zhang, Almon P. Fisher, and Timothy J. Fuller, the disclosure of which is totally incorporated herein by reference, discloses an ink jet 35 printhead which comprises (i) an upper substrate with a set of parallel grooves for subsequent use as ink channels and a recess for subsequent use as a manifold, the grooves being open at one end for serving as droplet emitting nozzles, and (ii) a lower substrate in which one surface thereof has an array of heating elements and addressing electrodes formed thereon, said lower substrate having an insulative layer 40 deposited on the surface thereof and over the heating elements and addressing electrodes and patterned to form recesses therethrough to expose the heating elements and terminal ends of the addressing electrodes, the upper and lower substrates being aligned, mated, and bonded together 45 to form the printhead with the grooves in the upper substrate being aligned with the heating elements in the lower substrate to form droplet emitting nozzles, said upper substrate comprising a material formed by crosslinking or chain extending a polymer of formula I

55

I



60 or II

65



77

-continued



wherein x is an integer of 0 or 1, P is a substituent which imparts photosensitivity to the polymer, a, b, c, and d are each integers of 0, 1, 2, 3, or 4, provided that at least one of a, b, c, and d is equal to or greater than 1 in at least some of the monomer repeat units of the polymer, A is



or mixtures thereof, B is



78

-continued

II

5

10

14

25

30

35

40

50

55

60

65

wherein  $v$  is an integer of from 1 to about 20, and preferably from 1 to about 10,



wherein z is an integer of from 2 to about 20, and preferably from 2 to about 10,



wherein u is an integer of from 1 to about 20, and preferably from 1 to about 10,



wherein w is an integer of from 1 to about 20, and preferably from 1 to about 10,



-continued



or mixtures thereof, and n is an integer representing the number of repeating monomer units.

Copending application U.S. Ser. No. 09/217,330, filed Dec. 21, 1998, entitled "Improved Photoresist Compositions," with the named inventors Thomas W. Smith, David J. Luca, and Kathleen M. McGrane, the disclosure of which is totally incorporated herein by reference, discloses a composition comprising a blend of (a) a thermally reactive polymer selected from the group consisting of resoles, novolacs, thermally reactive polyarylene ethers, and mixtures thereof; and (b) a photoreactive epoxy resin that is photoreactive in the absence of a photocationic initiator.

U.S. Pat. No. 5,738,799, filed Sep. 12, 1996, the disclosure of which is totally incorporated herein by reference, discloses an ink-jet printhead fabrication technique which enables capillary channels for liquid ink to be formed with square or rectangular cross-sections. A sacrificial layer is placed over the main surface of a silicon chip, the sacrificial layer being patterned in the form of the void formed by the desired ink channels. A permanent layer, comprising permanent material, is applied over the sacrificial layer, and, after polishing the two layers to form a uniform surface, the sacrificial layer is removed. Preferred materials for the sacrificial layer include polyimide while preferred materials for the permanent layer include polyarylene ether, although a variety of material combinations are possible.

Copending application U.S. Ser. No. 08/705,914, filed Aug. 29, 1996, entitled "Thermal Ink Jet Printhead With Ink Resistant Heat Sink Coating," with the named inventors Ram S. Narang and Timothy J. Fuller, the disclosure of which is totally incorporated herein by reference, discloses a heat sink for a thermal ink jet printhead having improved resistance to the corrosive effects of ink by coating the surface of the heat sink with an ink resistant film formed by electrophoretically depositing a polymeric material on the heat sink surface. In one described embodiment, a thermal ink jet printer is formed by bonding together a channel plate and a heater plate. Resistors and electrical connections are formed in the surface of the heater plate. The heater plate is bonded to a heat sink comprising a zinc substrate having an electrophoretically deposited polymeric film coating. The film coating provides resistance to the corrosion of higher pH inks. In another embodiment, the coating has conductive fillers dispersed therethrough to enhance the thermal conductivity of the heat sink. In one embodiment, the polymeric material is selected from the group consisting of polyethersulfones, polysulfones, polyamides, polyimides, polyamide-imides, epoxy resins, polyetherimides, polyarylene ether ketones, chloromethylated polyarylene ether ketones, acryloylated polyarylene ether ketones, polystyrene and mixtures thereof.

U.S. Pat. No. 5,843,259, filed Aug. 29, 1996, entitled "Method for Applying an Adhesive Layer to a Substrate Surface," with the named inventors Ram S. Narang, Stephen F. Pond, and Timothy J. Fuller, the disclosure of which is totally incorporated herein by reference, discloses a method for uniformly coating portions of the surface of a substrate

which is to be bonded to another substrate. In a described embodiment, the two substrates are channel plates and heater plates which, when bonded together, form a thermal ink jet printhead. The adhesive layer is electrophoretically deposited over a conductive pattern which has been formed on the binding substrate surface. The conductive pattern forms an electrode and is placed in an electrophoretic bath comprising a colloidal emulsion of a preselected polymer adhesive. The other electrode is a metal container in which the solution is placed or a conductive mesh placed within the container. The electrodes are connected across a voltage source and a field is applied. The substrate is placed in contact with the solution, and a small current flow is carefully controlled to create an extremely uniform thin deposition of charged adhesive micelles on the surface of the conductive pattern. The substrate is then removed and can be bonded to a second substrate and cured. In one embodiment, the polymer adhesive is selected from the group consisting of polyamides, polyimides, polyamide-imides, epoxy resins, polyetherimides, polysulfones, polyether sulfones, polyarylene ether ketones, polystyrenes, chloromethylated polyarylene ether ketones, acryloylated polyarylene ether ketones, and mixtures thereof.

Copending application U.S. Ser. No. 08/697,750, filed Aug. 29, 1996, now abandoned entitled "Electrophoretically Deposited Coating For the Front Face of an Ink Jet Printhead," with the named inventors Ram S. Narang, Stephen F. Pond, and Timothy J. Fuller, the disclosure of which is totally incorporated herein by reference, discloses an electrophoretic deposition technique for improving the hydrophobicity of a metal surface, in one embodiment, the front face of a thermal ink jet printhead. For this example, a thin metal layer is first deposited on the front face. The front face is then lowered into a colloidal bath formed by a fluorocarbon-doped organic system dissolved in a solvent and then dispersed in a non-solvent. An electric field is created and a small amount of current through the bath causes negatively charged particles to be deposited on the surface of the metal coating. By controlling the deposition time and current strength, a very uniform coating of the fluorocarbon compound is formed on the metal coating. The electrophoretic coating process is conducted at room temperature and enables a precisely controlled deposition which is limited only to the front face without intrusion into the front face orifices. In one embodiment, the organic compound is selected from the group consisting of polyimides, polyamides, polyamide-imides, polysulfones, polyarylene ether ketones, polyethersulfones, polytetrafluoroethylenes, polyvinylidene fluorides, polyhexafluoro-propylenes, epoxies, polyperfluorostyrenes, polystyrenes, copolymers thereof, terpolymers thereof, and mixtures thereof.

Copending application U.S. Ser. No. 08/705,916, filed Aug. 29, 1996, now U.S. Pat. No. 5,939,206, entitled "Stabilized Graphite Substrates," with the named inventors Gary A. Kneezeel, Ram S. Narang, Timothy J. Fuller, and Peter J. John, the disclosure of which is totally incorporated herein by reference, discloses an apparatus which comprises at least one semiconductor chip mounted on a substrate, said substrate comprising a graphite member having electrophoretically deposited thereon a coating of a polymeric material. In one embodiment, the semiconductor chips are thermal ink jet printhead subunits. In one embodiment, the polymeric material is of the general formula



or



wherein x is an integer of 0 or 1, A is one of several specified groups, such as



B is one of several specified groups, such as



or mixtures thereof, and n is an integer representing the number of repeating monomer units.

Japanese Patent Publication 63-247757 A2, the disclosure of which is totally incorporated herein by reference, discloses an electrophotographic photosensitive body consisting of a body in which a photoconductive layer laminated on a conductive support contains a charge generating substance and/or a charge transporting substance, and at least one polyether ketone polymer consisting of structural units which can be expressed by the following general formulae (I) and (II)



wherein m is 0 or 1 and Ar indicates



wherein R is an alkyl group, n is 0, 1, or 2, and X indicates



with R' and R'' each independently indicating —H, —CH<sub>3</sub>, —C<sub>2</sub>H<sub>5</sub>,



wherein the proportion of structural units in the polymer expressed by the general formula (I) is from 0.1 to 1.0 and the proportion of structural units in the polymer expressed by the general formula (II) is 0 to 0.9.

U.S. Pat. No. 5,336,577 (Spiewak et al.), the disclosure of which is totally incorporated herein by reference, discloses a thick organic ambipolar layer on a photoresponsive device which is simultaneously capable of charge generation and charge transport. In particular, the organic photoresponsive layer contains an electron transport material such as a fluorenylidene malonitrile derivative and a hole transport material such as a dihydroxy tetraphenyl benzidine containing polymer. These may be complexed to provide photoresponsivity, and/or a photoresponsive pigment or dye may also be included.

U.S. Pat. No. 4,806,517 (Frechet et al.), the disclosure of which is totally incorporated herein by reference, discloses an electrostatographic imaging member and an electrophotographic imaging process for using the imaging member in which the imaging member comprises a substrate and at least one electroconductive layer, the imaging member comprising a polymeric arylamine compound represented by the formula



wherein n is between about 5 and 5,000, m is 0 or 1, Z is selected from certain specified aromatic and fused ring groups, Ar is selected from certain specified aromatic groups, R is selected from certain specified alkyl groups, Ar' is selected from certain specified aromatic groups, and R'' and R''' are independently selected from certain specified alkylene groups.

U.S. Pat. No. 4,806,443 (Yanus et al.), the disclosure of which is totally incorporated herein by reference, discloses an electrostatographic imaging member and an electrophotographic imaging process for using the imaging member in which the imaging member comprises a substrate and an electroconductive layer, the imaging member comprising a polymeric arylamine compound represented by the formula



wherein n is between 5 and about 5,000, m is 0 or 1, y is 1, 2, or 3, Z is selected from certain specified aromatic and fused ring groups, Ar is selected from certain specified aromatic groups, Ar' is selected from certain specified aromatic groups, and X' is an alkylene radical selected from the group consisting of alkylene and isoalkylene groups containing 2 to 10 carbon atoms. The imaging member may comprise a substrate, charge generation layer, and a charge transport layer.

U.S. Pat. No. 4,806,444 (Yanus et al.) and U.S. Pat. No. 4,935,487 (Yanus et al.), the disclosures of each of which are totally incorporated herein by reference, disclose an electrostatographic imaging member and an electrophotographic imaging process for using the imaging member in which the imaging member comprises a substrate and an electroconductive layer, the imaging member comprising a polymeric arylamine compound represented by the formula



wherein n is between about 5 and about 5,000, m is 0 or 1, Z is selected from certain specified aromatic and fused ring groups, Ar is selected from certain specified aromatic groups, and Ar' is selected from certain specified aromatic groups. The imaging member may comprise a substrate, charge generation layer, and a charge transport layer.

U.S. Pat. No. 4,818,650 (Limburg et al.) and U.S. Pat. No. 4,956,440 (Limburg et al.), the disclosures of each of which are totally incorporated herein by reference, disclose an electrostatographic imaging member and an electrophotographic imaging process for using the imaging member in which the imaging member comprises a substrate and at least one electroconductive layer, the imaging member comprising a polymeric arylamine compound represented by the formula



wherein R is selected from the group consisting of —H, —CH<sub>3</sub>, and —C<sub>2</sub>H<sub>5</sub>, m is between about 4 and about 1,000, A is selected from the group consisting of an arylamine group represented by the formula



wherein m is 0 or 1, Z is selected from certain specified aromatic and fused ring groups that also contain an oxygen or sulfur atom, certain linear or cyclic hydrocarbon groups, and certain amine groups, Ar is selected from certain speci-

fied aromatic groups, Ar' is selected from certain specified aromatic groups, and B is selected from the group consisting of the arylamine group as defined for A and



wherein Ar is as defined above and V is selected from an oxygen or sulfur atom, certain linear or cyclic hydrocarbon groups, or a phenylene group, and at least A or B contains the arylamine group. The imaging member may comprise a substrate, charge generation layer, and a charge transport layer.

U.S. Pat. No. 5,030,532 (Limburg et al.), the disclosure of which is totally incorporated herein by reference, discloses an electrostatographic imaging member comprising a support layer and at least one electrophotoconductive layer, said imaging member comprising a polyarylamine polymer represented by the formula



wherein n is between about 5 and about 5,000, or 0 if p>0, o is between about 9 and about 5,000, or is 0 if p>0 or n=0, p is between about 2 and about 100, or is 0 if n>0, X' and X'' are independently selected from a group having bifunctional linkages, Q is a divalent group derived from certain hydroxy terminated arylamine reactants, Q' is a divalent group derived from a hydroxy terminated polyarylamine containing the group defined for Q and having a weight average molecular weight between about 1,000 and about 80,000, and the weight average molecular weight of the polyarylamine polymer is between about 10,000 and about 1,000,000.

U.S. Pat. No. 5,438,082 (Helmer-Metzmann et al.) and U.S. Pat. No. 5,561,202 (Helmer-Metzmann et al.), the disclosures of each of which are totally incorporated herein by reference, disclose the production of a polymer electrolyte membrane from sulfonated aromatic polyether ketones. An aromatic polyether ketone of the formula



in which Ar is a phenylene ring having p- and/or m-bonds, Ar' is a phenylene, naphthylene, biphenylene, anthrylene, or other divalent aromatic unit, X, N, and M, independently of one another, are 0 or 1, Y is 0, 1, 2, or 3, and P is 1, 2, 3, or 4, is sulfonated and the sulfonic acid is isolated. At least 5 percent of the sulfonic groups in the sulfonic acid are converted into sulfonyl chloride groups, and these groups are reacted with an amine containing at least one crosslinkable substituent or a further functional group, and unreacted sulfonyl chloride groups are subsequently hydrolyzed. The resultant aromatic sulfonamide is isolated and dissolved in an organic solvent, the solution is converted into a film, and the crosslinkable substituents in the film are then crosslinked. In specific cases, the crosslinkable substituents can be omitted, in which case, sulfonated polyether ketone is converted into a film from solution. In another embodiment of the disclosed invention, the polymer may contain, in addition to units of the above formula, non-sulfonatable units such as those of the formula



In yet another embodiment of the disclosed invention, as disclosed in columns 8 and 9, mixtures of polymeric, crosslinkable sulfonamides and polymeric, non-crosslinkable, aromatic sulfonic acids can be converted jointly into membranes.

U.S. Pat. No. 4,623,558 (Lin), the disclosure of which is totally incorporated herein by reference, discloses a thermo-

setting plastisol dispersion composition comprising (1) poly(phenylene oxide) in powder form, which is insoluble in the reactive plasticizer at room temperature and plasticizable at a temperature at or above the fluxing temperature; (2) a liquid reactive plasticizer member of the group consisting of (a) at least one epoxide resin having an average of more than one epoxide group in the molecule, (b) at least one liquid monomer, oligomer, or prepolymer containing at least one ethylenically unsaturated group, and (c) a mixture of (a) and (b), said reactive plasticizer being capable of solvating the poly(phenylene oxide) at the fluxing temperature and being present in an amount ranging from 5 to 2,000 parts per 100 parts by weight of (1); and (3) 0.01 to 10 percent by weight of (2) of either a thermal initiator or photoinitiator for plasticizers present in the composition. The plastisol dispersion after fluxing can form a thermoset after the crosslinking reaction.

U.S. Pat. No. 4,667,010 (Eldin), the disclosure of which is totally incorporated herein by reference, discloses linear polyether resins containing 100 to 10 mol % of the repeating structural unit of formula I

I



and 90 to 0 mol % of the repeating structural unit of formula II

II



wherein A is a linear unsubstituted or methyl-substituted alkylene group containing 4 to 100 carbon atoms in the linear alkylene chain, X is



wherein R is C1-C8 alkyl or



wherein each of R<sup>1</sup> and R<sup>2</sup> is a hydrogen or a halogen atom, and Y is



wherein R<sup>3</sup> and R<sup>4</sup> are the same or different and each is a halogen atom, C<sub>1</sub>-C<sub>4</sub> alkyl, or C<sub>1</sub>-C<sub>4</sub> alkoxy, m and n are 0 or an integer from 1 to 4, and Z is a direct bond or a radical selected from the group consisting of



wherein each of R<sup>5</sup> and R<sup>6</sup> independently of the other is a hydrogen atom, C<sub>1</sub>-C<sub>4</sub> alkyl, or phenyl,



The resins are self-crosslinkable and can be crosslinked by heating to a temperature of not less than 250° C. or by 45 irradiation with energy-rich electromagnetic rays, affording products which are insoluble in organic solvents and which have high glass transition temperatures. The heat crosslinking can, if desired, be carried out in the presence of radical formers such as inorganic or organic peroxides, including 50 potassium peroxide sulfate or benzoyl peroxide, azo compounds such as azoisobutyronitrile, organic hydroperoxides,  $\alpha$ -haloacetophenones, benzoin or ethers thereof, benzophenones, benzil acetals, anthraquinones, arsines, phosphines, or thioureas. Crosslinking can also be carried 55 out with energy-rich rays such as X-rays, accelerated electrons, or  $\gamma$ -rays emitted from a  $^{60}\text{Co}$  source.

U.S. Pat. No. 5,268,444 (Jensen et al.), the disclosure of which is totally incorporated herein by reference, discloses phenylethynyl-terminated poly(arylene ethers) which are 60 prepared in a wide range of molecular weights by adjusting the monomer ratio and adding an appropriate amount of 4-fluoro-4'-phenylethynylbenzophenone during polymer synthesis. The resulting phenylethynyl-terminated poly(arylene ethers) react and crosslink upon curing for one hour 65 at 350° C. to provide materials with improved solvent resistance, higher modulus, and better high temperature properties than the linear, uncrosslinked polymers.

U.S. Pat. No. 4,435,496 (Walls et al.), the disclosure of which is totally incorporated herein by reference, discloses novel photosensitive compositions containing a compound consisting essentially of repeating structural units of an alkyl aryl ether, which are endcapped with a substituent functional group containing an ethylenically unsaturated moiety, and a photosensitizing effective amount of a free radical generating compound. Through the selected exposure of films and coatings prepared from the composition, it is possible to record information in the materials in a manner to alter the physical and/or chemical properties of the films and coatings. Upon selected exposure of the film or coating to imaging energies, the photosensitive species within the composition either itself undergoes a degradative reaction or promotes degradation of one or more of the other components of the composition. This selective modification can then be simply manifested by contacting the exposed surface of the film or coating, subsequent to such exposure, with an alkaline developing solution. The compositions are useful in the graphic arts and in the manufacture of printed circuit boards for the electronics industry.

U.S. Pat. No. 3,455,868 (D'Alessandro), the disclosure of which is totally incorporated herein by reference, discloses a friction composition of particulate friction material and a binder of a heat-hardenable resin and a thermoplastic polyarylene polyether. The thermoplastic polyarylene polyether is linear and of the basic structure composed of recurring units having the formula



wherein E is the residuum of the dihydric phenol and E' is the residuum of the benzenoid compound having an inert electron withdrawing group in at least one of the positions ortho and para to the valence bonds, and wherein both of said residua are valently bonded to the ether oxygens through aromatic carbon atoms. Preferred linear thermoplastic polyarylene polyethers are composed of recurring units having the formula



wherein R represents a member of the group consisting of a bond between aromatic carbon atoms and a divalent connecting radical and R' represents a member of the group consisting of sulfone, carbonyl, vinyl, sulfoxide, azo, saturated fluorocarbon, organic phosphine oxide, and ethylidene groups, and Y and Y<sub>1</sub> each represent inert substituent groups selected from the group consisting of halogen, alkyl groups having from 1 to 4 carbon atoms, and alkoxy groups having from 1 to 4 carbon atoms, and where r and z are integers having a value from 0 to 4 inclusive, and preferably having a value of 0. In Example 14, the polyarylene polyether is of the formula



U.S. Pat. No. 5,336,720 (Richards et al.), the disclosure of which is totally incorporated herein by reference, discloses an impact resistant graft polymer and an emulsion polymerization process comprising (1) an agglomerated rubber latex

made from a rubber latex and a polymerized polymeric additive, and (2) a grafted polymer. Specifically, the graft polymer comprises:

5) 1) from about 60 to about 95 parts by weight or more (as weight of solid component) of an agglomerated rubber latex (C) having the following composition:

- (a) 100 parts by weight (as weight of solid component) of a synthetic rubber latex (A) having particle distribution between about 60 and about 200 nm, and a pH from about 8.0 to about 10.0; and
- (b) from about 0.1 to about 5.0 parts by weight (as weight of solid component) of a polymerized polymeric additive (B) having an average particle diameter of about 100 to about 300 nm, and formed by polymerizing:
  - (1) one or more monomer groups where at least one monomer group always contains at least 30% by weight of unsaturated carboxylic acid selected from acrylic acid, methacrylic acid, itaconic acid, acryloxypropionic acid, crotonic acid, and the like;
  - (2) from about 5 to about 70% (by weight) of at least one alkyl acrylate having C<sub>1</sub>–C<sub>12</sub> alkyl group (such as methyl methacrylate, hydroxyethyl methacrylate, butyl acrylate, and the like; and
  - (3) up to 80% (by weight) of other copolymerizable monomer(s); and
  - 2) from about 5 to about 40 parts by weight of a grafted polymer (D) formed by polymerizing (a) 30% by weight or more of at least one monomer selected from styrene, acrylonitrile, methyl methacrylate, hydroxyethyl methacrylate, butyl acrylate, ethyl acrylate, and the like; and (b) 30% by weight or less of a vinyl monomer having CH<sub>2</sub>=C< copolymerizable therewith. As stated at columns 4 an 5, bridging paragraph, in the preparation of the (B) component, the “other copolymerizable monomers” can be unsaturated aromatic compounds such as styrene, alpha-methylstyrene, and vinyltoluene; unsaturated nitrile compounds such as acrylonitrile and methacrylonitrile; alkyl methacrylates having C<sub>1</sub>–C<sub>12</sub> alkyl group, such as butyl acrylate and hydroxyethylmethacrylate; and diolefins such as butadiene. Crosslinkers or graftlinkers such as ethylenically unsaturated esters (e.g., allyl methacrylate and methallyl methacrylate, 1,3-butylene glycol dimethacrylate, trimethyl glycol propane triacrylate, and the like), or other ethylenically unsaturated monomers (e.g., divinyl benzene and trivinyl benzene) may be used, at levels typically less than or equal to 2% by weight.

EP 0 281 808, the disclosure of which is totally incorporated herein by reference, discloses a thermally stable radiation crosslinkable polymer system which cures without additional heat treatment which comprises a main component A which is a polyether acrylate or a compound in accordance with one of the structural formulae

CHY<sub>2</sub>

(1)

CHY<sub>2</sub>—CHY<sub>2</sub>

(2)

**91**

-continued



wherein Y denotes a radical of the structure



in which X is H, Cl, or OH and where A denotes the acyl radical of a substituted acrylic acid, and 1 to 10 percent by weight of a component B, different therefrom, as a crosslinking intensifier, which component B is selected from pentaaerythritol triacrylate or tetraacrylate, dipentaerythritol pentaacrylate, or trimethylolpropane triacrylate. In one specific embodiment, the polyether acrylate has the general structure



JP 60-57826, the disclosure of which is totally incorporated herein by reference, discloses azido group containing polyether sulfones containing a repeating unit of the formula



wherein Ar<sub>1</sub> represents an aromatic hydrocarbon group with carbon number 6 to 10 (2+p), Ar<sub>2</sub> represents an aromatic hydrocarbon group with carbon number 6 to 10 (2+q), Ar<sub>3</sub> represents a divalent aromatic group with carbon number 6 to 15, and p and q represent 0, 1, or 2 and satisfy p+q=1 to 4. Specific examples of Ar<sub>1</sub> and Ar<sub>2</sub> include



**92**  
methyl substitutes of the above,  
(3)

Examples of suitable Ar<sub>3</sub> groups include

-continued



and



The resin is heat resistant and photosensitive, and suitable 15 for use as a photoresist for microprocessing.

JP 56-050929, the disclosure of which is totally incorporated herein by reference, discloses a polysulfone characterized by having a carbon-carbon double bond in the side chain, represented by the formula 20



wherein  $\text{Ar}_1$  is a  $(2+p)$  valence aromatic hydrocarbon group having 6 to 10 carbon atoms,  $\text{Ar}_2$  is a  $(2+q)$  valence aromatic hydrocarbon group having 6 to 10 carbon atoms,  $\text{Ar}_3$  is a divalent aromatic hydrocarbon group having 6 to 15 carbon atoms,  $-\text{X}_{11}-$  and  $-\text{X}_{12}-$  are the same or different and show connecting  $-\text{O}-$  or  $-\text{NR}_3-$ ,  $\text{R}_3$  is a hydrogen atom or univalent hydrocarbon group having 1 to 10 carbon atoms,  $\text{R}_{11}$  and  $\text{R}_{12}$  are the same or different and hydrogen atoms or methyl groups,  $\text{R}_{21}$  and  $\text{R}_{22}$  are the same or different and hydrogen atoms or phenyl groups,  $\text{r}_{21}$  and  $\text{r}_{22}$  are independently 1 or 2,  $p$  and  $q$  are independently 0, 1, or 2, and the equation  $p+q=1$  to 4 must be satisfied.

JP 56-050928, the disclosure of which is totally incorporated herein by reference, discloses a polysulfone characterized by having, in the side chain, a (meth)acrylate group comprising a constituting unit represented by the following general formula (I):



wherein Ar<sub>1</sub> is a (2+p) valence aromatic hydrocarbon group having 6 to 10 carbon atoms, Ar<sub>2</sub> is a (2+q) valence aromatic hydrocarbon group having 6 to 10 carbon atoms, Ar<sub>3</sub> is a divalent aromatic hydrocarbon group having 6 to 15 carbon atoms which may contain the hetero atom S or O, —X<sub>1</sub>— and —X<sub>2</sub>— are the same or different and show connecting —O— or —NR<sub>3</sub>—, R<sub>1</sub> is a hydrogen atom or univalent hydrocarbon group having 1 to 10 carbon atoms, R<sub>2</sub> is an alkyl group having 2 to 5 carbon atoms, and furthermore, R<sub>3</sub> is a hydrogen atom or methyl group; p and 1 are independently 0, 1, or 2, and the equation p+q=1 to 4 must be satisfied.

35 U.S. Pat. No. 4,086,209 (Hara et al.), the disclosure of  
which is totally incorporated herein by reference, discloses  
substantially linear or at least partially crosslinked nitrogen-  
containing polymers having an aryleneimine or aryleneether  
40 unit in the main chain with an amino group or a group  
derived from it being bonded as a pendant group to a nuclear  
carbon atom of the arylene group of the above unit. Accord-  
ing to the number and type of the pendant groups, the  
45 polymers can have various useful properties such as thermal  
stability, hydrophilicity, oxidative reducibility,  
photosensitivity, color formability, or the ability to form  
coordination bonds. Further, the polymers have good solu-  
50 bility in aprotic polar organic solvents. Permselective mem-  
branes having good performance can be prepared from  
solutions of the polymers in these solvents.

55 EP 0 663 411, the disclosure of which is totally incorporated herein by reference, discloses a photoimaging resist ink containing (A) an unsaturated group-having polycarboxylic acid resin which is a reaction product of (c) succinic anhydride with an additive reaction product of (a) an epoxy resin with (b) an unsaturated group-having monocarboxylic acid, wherein (a) the epoxy resin is represented by the formula

95



wherein  $M$  stands for



n is at least 1 on the average, and m is 1 to n on the average. In specific embodiments, the resist further contains (B) a photopolymerization initiator, (C) a diluent, and (D) a curing component. In forming a solder resist pattern by exposing a coating film of a resist ink through a patterned film to ultraviolet light and developing the coating film to dissolve away the unexposed portions thereof, the resist ink is excellent in developability and photosensitivity, while the cure product thereof is excellent in flex resistance and folding resistance, heat resistance, and the like. The resist ink is especially suitable as a liquid solder resist ink for flexible printed circuit boards and thin pliable rigid circuit boards.

U.S. Pat. No. 4,448,948 (Tsubaki et al.), the disclosure of which is totally incorporated herein by reference, discloses an epoxy resin substantially represented by the general formula



wherein  $\text{Ar}^1$  is a residual group of a dihydric phenol derived from a compound having one or two benzene nuclei,  $\text{Ar}^2$  is a residual group of a halogen-substituted benzenoid compound having two halogen atoms on its nuclei and represented by the formula



wherein each of  $\text{Ar}^3$  and  $\text{Ar}^4$  is a hydrocarbon group having a divalent benzene nucleus and  $\text{Y}$  is a sulfone group or a 50 carbonyl group, and  $n$  is an integer of from 1 to 50.

U.S. Pat. No. 5,728,498 (Yanus et al.), the disclosure of which is totally incorporated herein by reference, discloses a flexible electrophotographic imaging member including a supporting substrate coated with at least one imaging layer 55 comprising hole transporting material containing at least two long chain alkyl carboxylate groups dissolved or molecularly dispersed in a film forming binder. Preferred charge transporting materials are of the formula



wherein m is 0 or 1, Z is selected from the group consisting of

10



and



<sup>40</sup> n is 0 or 1, Ar is selected from the group consisting of



and



60 R is selected from the group consisting of  $-\text{CH}_3$ ,  $-\text{C}_2\text{H}_5$ ,  $-\text{C}_3\text{H}_7$ , and  $-\text{C}_4\text{H}_9$ , Ar' is selected from the group consisting of





and



X is selected from the group consisting of  $-\text{CH}_2-$ ,  $-\text{C}(\text{CH}_3)_2-$ ,  $-\text{O}-$ ,  $-\text{S}-$ ,



and



s is 0, 1, or 2, and Q is represented by the formula



wherein p is 1 or 0,  $\text{R}_1$ ,  $\text{R}_2$ ,  $\text{R}_3$ ,  $\text{R}_4$  are independently selected from  $-\text{H}$ ,  $-\text{CH}_3$ ,  $-(\text{CH}_2)_v\text{CH}_3$ ,  $-\text{CH}(\text{CH}_3)_2$ ,  $-\text{C}(\text{CH}_3)_3$ , wherein v is 1 to 10, and s and n are independently selected from 0 to 10.

Copending application U.S. Ser. No. 09/326,169, filed concurrently herewith, entitled "Arylene Ether Alcohol Polymers," with the named inventors Timothy J. Fuller, John F. Yanus, Damodar M. Pai, Markus R. Silvestri, Ram S. Narang, William W. Limburg, and Dale S. Renfer, the disclosure of which is totally incorporated herein by reference, discloses a polymer of the formula



55

60 wherein A is

65



wherein A is

5



10 or a mixture of

15



wherein R is a hydrogen atom, an alkyl group, an aryl group, or mixtures thereof, B is one of specified groups, such as

25



30



35



or mixtures thereof, and n is an integer representing the number of repeating monomer units.

40

Copending application U.S. Ser. No. 09/326,170, filed concurrently herewith, entitled "Imaging Members Containing Arylene Ether Alcohol Polymers," with the named inventors Timothy J. Fuller, John F. Yanus, Damodar M. Pai, Markus R. Silvestri, Ram S. Narang, William W. Limburg, and Dale S. Renfer, the disclosure of which is totally incorporated herein by reference, discloses an imaging member which comprises a conductive substrate, a photo-generating material, and a binder comprising a polymer of the formula



50

60 wherein A is

65



or a mixture of



wherein R is a hydrogen atom, an alkyl group, an aryl group, or mixtures thereof, B is one of specified groups, such as



or mixtures thereof, and n is an integer representing the number of repeating monomer units.

While known compositions and processes are suitable for their intended purposes, a need remains for improved materials suitable for microelectronics applications. A need also remains for improved ink jet printheads. Further, there is a need for crosslinkable or chain extendable polymeric materials which are heat stable, electrically insulating, and mechanically robust. Additionally, there is a need for crosslinkable or chain extendable polymeric materials which are chemically inert with respect to the materials that might be employed in ink jet ink compositions. There is also a need for crosslinkable or chain extendable polymeric materials which exhibit low shrinkage during post-cure steps in micro-electronic device fabrication processes. In addition, a need remains for crosslinkable or chain extendable polymeric materials which exhibit a relatively long shelf life. Further, there is a need for photopatternable polymeric materials which can be patterned with relatively low photo-exposure energies. Additionally, a need remains for crosslinkable or chain extendable polymeric materials which, in the cured form, exhibit good solvent resistance. There is also a need for crosslinkable or chain extendable polymeric materials which, when applied to microelectronic devices by spin casting techniques and cured, exhibit reduced edge bead and no apparent lips and dips. In addition, there remains a need for crosslinkable or chain extendable polymeric materials which have relatively low dielectric constants. Further, there is a need for crosslinkable or chain extendable polymeric materials which exhibit reduced water sorption. Additionally, a need remains for crosslinkable or chain extendable polymeric materials which exhibit improved hydrolytic stability, especially upon exposure to alkaline solutions. A need also remains for photopatternable polymeric materials which are stable at high temperatures, typically greater than about 150° C. There is also a need for photopatternable polymeric materials which either have high glass transition temperatures or are sufficiently crosslinked that there are no low temperature phase transitions subsequent to photoexposure. Further, a need remains for photopatternable polymeric materials with low coefficients of thermal expansion. There is a need for polymers

which are thermally stable, patternable as thick films of about 30 microns or more, exhibit low  $T_g$  prior to photoexposure, have low dielectric constants, are low in water absorption, have low coefficients of expansion, have 5 desirable mechanical and adhesive characteristics, and are generally desirable for interlayer dielectric applications, including those at high temperatures, which are also photopatternable. There is also a need for photoresist compositions with good to excellent processing characteristics.

## SUMMARY OF THE INVENTION

The present invention is directed to an ink jet printhead 15 which comprises: (i) an upper substrate, and (ii) a lower substrate in which one surface thereof has an array of heating elements and addressing electrodes formed thereon, said lower substrate having an insulative layer deposited on the surface thereof and over the heating elements and addressing electrodes and patterned to form recesses there-through to expose the heating elements and terminal ends of the addressing electrodes, said upper and lower substrates being bonded together to form a thermal ink jet printhead 20 25 having droplet emitting nozzles defined by the upper substrate, the insulative layer on the lower substrate, and the heating elements in the lower substrate, wherein at least one of said upper substrate and said insulative layer comprises a crosslinked or chain extended polymer formed by crosslinking or chain extending a precursor polymer having terminal end groups and monomer repeat units, said precursor polymer being of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units 50 of the polymer, A is



or a mixture of



wherein R is a hydrogen atom, an alkyl group, an aryl group, or mixtures thereof, B is

**101****102**

wherein v is an integer of from 1 to about 20,



10 wherein z is an integer of from 2 to about 20,



20 wherein u is an integer of from 1 to about 20,



50 wherein w is an integer of from 1 to about 20,



103



wherein  $R_1$  and  $R_2$  each, independently of the other, are hydrogen atoms, alkyl groups, or aryl groups, and  $p$  is an integer of 0 or 1,

104



wherein  $p$  is 0 or 1; (2)  $\text{Ar}$  is



wherein  $p$  is an integer of 0 or 1,



wherein  $t$  is an integer of from 1 to about 20,



(3)  $\text{G}$  is an alkyl group selected from alkyl or isoalkyl groups containing from about 2 to about 10 carbon atoms; (4)  $\text{Ar}'$  is



wherein (1)  $Z$  is



-continued



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, said crosslinking or chain extension occurring through crosslinking substituents contained on at least some of the monomer repeat units of the precursor polymer.

Another embodiment of the present invention is directed to a process for forming an ink jet printhead which comprises: (a) providing a lower substrate in which one surface thereof has an array of heating elements and addressing electrodes having terminal ends formed thereon; (b) depositing onto the surface of the lower substrate having the heating elements and addressing electrodes thereon a layer comprising a photopatternable polymer; (c) exposing the layer to actinic radiation in an imagewise pattern such that the photopatternable polymer in exposed areas becomes crosslinked or chain extended and the photopatternable polymer in unexposed areas does not become crosslinked or chain extended, wherein the unexposed areas correspond to areas of the lower substrate having thereon the heating elements and the terminal ends of the addressing electrodes; (d) removing the photopatternable polymer from the unexposed areas, thereby forming recesses in the layer, said recesses exposing the heating elements and the terminal ends of the addressing electrodes; (e) providing an upper substrate comprising a supporting substrate and, coated thereon, a material formed by crosslinking or chain extending a composition comprising a crosslinked or chain extended polymer formed by crosslinking or chain extending a precursor polymer having terminal end groups and monomer repeat units, said precursor polymer being of the formula



10 wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



25 or a mixture of



35 wherein R is a hydrogen atom, an alkyl group, an aryl group, or mixtures thereof, B is



107

-continued

  
  
  
  
  
  
  
  
  


wherein  $v$  is an integer of from 1 to about 20,



wherein  $z$  is an integer of from 2 to about 20,



wherein  $u$  is an integer of from 1 to about 20.



108

-continued



20 wherein w is an integer of from 1 to about 20,



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,

65

$$-(\text{CH}_2\text{O})_r-$$

109

wherein t is an integer of from 1 to about 20,



wherein (1) Z is



wherein p is 0 or 1; (2) Ar is



wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and (f)

111

bonding the upper substrate to the lower substrate to form a thermal ink jet printhead having droplet emitting nozzles defined by the upper substrate, the photopatternable polymer on the lower substrate, and the heating elements in the lower substrate.

Yet another embodiment of the present invention is directed to a process for forming an ink jet printhead which comprises: (a) depositing a layer comprising a precursor polymer having terminal end groups and monomer repeat units, said precursor polymer being of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



or a mixture of



wherein R is a hydrogen atom, an alkyl group, an aryl group, or mixtures thereof, B is



112

-continued



wherein v is an integer of from 1 to about 20,



**113**

wherein z is an integer of from 2 to about 20,



wherein u is an integer of from 1 to about 20,



wherein w is an integer of from 1 to about 20,

**114**wherein R<sub>1</sub> and R<sub>2</sub> each, independently of the other, are hydrogen atoms, alkyl groups, or aryl groups, and p is an integer of 0 or 1,

wherein p is an integer of 0 or 1,

-(CH<sub>2</sub>O)<sub>t</sub>-

wherein t is an integer of from 1 to about 20,



wherein (1) Z is



115

-continued



wherein p is 0 or 1; (2) Ar is



or



(3) G is an alkyl group selected from alkyl or isoalkyl groups containing from about 2 to about 10 carbon atoms; (4) Ar' is



or



(5) X is



116

-continued



5



10



15



20

wherein s is 0, 1, or 2,  
 25 and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units onto a lower substrate in which one surface thereof has an array of  
 30 heating elements and addressing electrodes having terminal ends formed thereon, said polymer being deposited onto the surface having the heating elements and addressing electrodes thereon; (b) exposing the layer to actinic radiation in an imagewise pattern such that the precursor polymer in exposed areas becomes crosslinked or chain extended and the precursor polymer in unexposed areas does not become crosslinked or chain extended, wherein the unexposed areas correspond to areas of the lower substrate having thereon the heating elements and the terminal ends of the addressing electrodes; (c) removing the precursor polymer from the unexposed areas, thereby forming recesses in the layer, said recesses exposing the heating elements and the terminal ends of the addressing electrodes; (d) providing an upper substrate; and (e) bonding the upper substrate to the lower substrate to form a thermal ink jet printhead having droplet emitting nozzles defined by the upper substrate, the crosslinked or chain extended polymer on the lower substrate, and the heating elements in the lower substrate.

40  
 45  
 50 In one specific embodiment of the present invention, the precursor polymer is prepared by a process which comprises (1) providing a pre-precursor polymer of the formula



60 wherein A is



65

B is



-continued  
 $-\text{CH}_2\text{v}-$ ,

5 wherein v is an integer of from 1 to about 20,



wherein z is an integer of from 2 to about 20,



wherein u is an integer of from 1 to about 20,



wherein w is an integer of from 1 to about 20,



119



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,



wherein  $t$  is an integer of from 1 to about 20,



wherein (1)  $Z$  is



120



or

20

25

30

35

40

45

50

55

60

65

wherein  $p$  is 0 or 1; (2)  $Ar$  is



or



40 (3)  $G$  is an alkyl group selected from alkyl or isoalkyl groups containing from about 2 to about 10 carbon atoms; (4)  $Ar'$  is



or



55 (5)  $X$  is



121

-continued



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and (2) reacting the pre-precursor polymer with borane, resulting in formation of a precursor polymer of the formula



wherein A is



or a mixture of



wherein R is a hydrogen atom, an alkyl group, an aryl group, or mixtures thereof.

In another specific embodiment of the present invention, the precursor polymer is prepared by a process which comprises (1) providing a pre-precursor polymer of the formula

122



10 wherein A is



123

-continued



B is



124

-continued



20 wherein v is an integer of from 1 to about 20,



30 wherein z is an integer of from 2 to about 20,



40 wherein u is an integer of from 1 to about 20,



125

wherein w is an integer of from 1 to about 20,



wherein  $R_1$  and  $R_2$  each, independently of the other, are hydrogen atoms, alkyl groups, or aryl groups, and  $p$  is an integer of 0 or 1,

wherein  $p$  is an integer of 0 or 1, $-(CH_2O)_t-$ wherein  $t$  is an integer of from 1 to about 20,

126

wherein (1)  $Z$  isor  $-\text{Ar}-(X)_p-\text{Ar}-$ wherein  $p$  is 0 or 1; (2)  $\text{Ar}$  is

55 (3)  $G$  is an alkyl group selected from alkyl or isoalkyl groups containing from about 2 to about 10 carbon atoms; (4)  $\text{Ar}'$  is



-continued  
or



;

(5) X is



wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the pre-precursor polymer with a reagent of the formula  $RMgX$ , wherein R is a hydrogen atom, an alkyl group, an aryl group, or mixtures thereof and X is a halogen atom, and (3) subsequent to step 2, adding water or acid to the pre-precursor polymer, thereby resulting in formation of a precursor polymer of the formula



wherein A is



or a mixture of



15  
wherein R is a hydrogen atom, an alkyl group, an aryl group, or mixtures thereof.

## BRIEF DESCRIPTION OF THE DRAWINGS

20  
FIG. 1 is an enlarged schematic isometric view of an example of a printhead mounted on a daughter board showing the droplet emitting nozzles.

25  
FIG. 2 is an enlarged cross-sectional view of FIG. 1 as viewed along the line 2-2 thereof and showing the electrode passivation and ink flow path between the manifold and the ink channels.

30  
FIG. 3 is an enlarged cross-sectional view of an alternate embodiment of the printhead in FIG. 1 as viewed along the line 2-2 thereof.

## DETAILED DESCRIPTION OF THE INVENTION

35  
The present invention is directed to ink jet printheads containing polymers of the general formula



wherein A is



or a mixture of



55  
wherein R is a (a) hydrogen atom, (b) an alkyl group, including unsubstituted alkyl groups and substituted alkyl groups, such as hydroxyalkyl groups, preferably with from 1 to about 20 carbon atoms, more preferably with from 1 to about 10 carbon atoms, and even more preferably with from 1 to about 5 carbon atoms, although the number of carbon atoms can be outside of this range, (c) an aryl group, including unsubstituted aryl groups and substituted aryl groups, such as hydroxyaryl groups, preferably with from 6

129

to about 18 carbon atoms, more preferably with from 6 to about 12 carbon atoms, and even more preferably with 6 carbon atoms, although the number of carbon atoms can be outside of this range, or (d) mixtures thereof, B is



60

130

-continued



10

$-(CH_2)_v-$ ,



20



30

35

wherein  $u$  preferably is an integer of from 1 to about 20, and more preferably from 1 to about 10,



45



55



65

wherein  $w$  preferably is an integer of from 1 to about 20, and more preferably from 1 to about 10,

131



wherein  $R_1$  and  $R_2$  each, independently of the other, are (a) hydrogen atoms, (b) alkyl groups, including unsubstituted alkyl groups and substituted alkyl groups, such as hydroxy-alkyl groups, preferably with from 1 to about 20 carbon atoms, more preferably with from 1 to about 10 carbon atoms, and even more preferably with from 1 to about 5 carbon atoms, although the number of carbon atoms can be outside of this range, (c) aryl groups, including unsubstituted aryl groups and substituted aryl groups, such as hydroxyaryl groups, preferably with 6 to about 18 carbon atoms, more preferably with 6 to about 12 carbon atoms, and even more preferably with 6 carbon atoms, although the number of carbon atoms can be outside of this range, or (d) mixtures thereof, and  $p$  is an integer of 0 or 1,



wherein  $p$  is an integer of 0 or 1,



wherein  $t$  is an integer of from 1 to about 20,



132



wherein (1)  $Z$  is



or



wherein  $p$  is 0 or 1; (2)  $Ar$  is



or



(3)  $G$  is an alkyl group selected from alkyl or isoalkyl groups containing from about 2 to about 10 carbon atoms; (4)  $Ar'$  is



or



(5) X is



wherein s is 0, 1, or 2,



or



and (6) q is 0 or 1; or mixtures thereof, hydroxy-substituted derivatives thereof, hydroxyalkyl-substituted derivatives thereof, with the hydroxyalkyl substituents preferably having from 1 to about 20 carbon atoms, more preferably from 1 to about 10 carbon atoms, and even more preferably from 1 to about 5 carbon atoms, although the number of carbon atoms can be outside of this range, hydroxyaryl-substituted derivatives thereof, with the hydroxyaryl substituents preferably having from 6 to about 18 carbon atoms, more preferably from 6 to about 12 carbon atoms, and even more preferably about 6 carbon atoms, although the number of carbon atoms can be outside of this range, or mixtures thereof, and n is an integer representing the number of

repeating monomer units. Specific examples of some preferred substituted derivatives include (but are not limited to)



10



15

wherein m and n are each integers of 0, 1, or 2,



20

wherein m and n are each integers of 0, 1, or 2,



25

wherein m, n, p, and q are each integers of 0, 1, or 2,



30

wherein m and n are each integers of 0, 1, or 2, and the like.

50 Desirable values for n, and the corresponding weight average molecular weight and number average molecular weight, depend on the desired use for the polymer. For example, when the polymer is to be provided with crosslinking groups such as photosensitivity-imparting groups and used for applications such as photoresists or ink jet printheads, the value of n is preferably such that the weight average molecular weight of the material is from about 1,000 to about 100,000, preferably from about 1,000 to about 65,000, more preferably from about 1,000 to about 40,000, and even more preferably from about 3,000 to about 25,000, although the weight average molecular weight can be outside these ranges; preferably, n is an integer of from about 2 to about 70, more preferably from about 5 to about 70, and even more preferably from about 8 to about 50, although the value of n can be outside these ranges. The phenyl groups and the A and/or B groups may also be

55

60

65

135

substituted, although the presence of two or more substituents on the B group ortho to the oxygen groups can render substitution difficult when it is desired to place crosslinking functional groups onto the polymer. Substituents can be present on the polymer either prior to or subsequent to the placement of crosslinking functional groups thereon. Substituents can also be placed on the polymer during the process of placement of crosslinking functional groups thereon. Substituents and/or crosslinking groups can be placed on the polymer before, during, or after preparation of the polymer of the basic formula



Examples of suitable substituents include (but are not limited to) alkyl groups, including saturated, unsaturated, and cyclic alkyl groups, preferably with from 1 to about 6 carbon atoms, substituted alkyl groups, including saturated, unsaturated, and cyclic substituted alkyl groups, preferably with from 1 to about 6 carbon atoms, aryl groups, preferably with from 6 to about 24 carbon atoms, substituted aryl groups, preferably with from 6 to about 24 carbon atoms, arylalkyl groups, preferably with from 7 to about 30 carbon atoms, substituted arylalkyl groups, preferably with from 7 to about 30 carbon atoms, alkoxy groups, preferably with from 1 to about 6 carbon atoms, substituted alkoxy groups, preferably with from 1 to about 6 carbon atoms, aryloxy groups, preferably with from 6 to about 24 carbon atoms, substituted aryloxy groups, preferably with from 6 to about 24 carbon atoms, arylalkyloxy groups, preferably with from 7 to about 30 carbon atoms, substituted arylalkyloxy groups, preferably with from 7 to about 30 carbon atoms, hydroxy groups, and the like.

One preferred embodiment of the present invention is directed to an ink jet printhead containing a polymer of the formula



wherein n is an integer representing the number of repeating monomer units. Another preferred embodiment of the present invention is directed to an ink jet printhead containing a polymer of the formula



wherein n is an integer representing the number of repeating monomer units.

Polymers useful for the printheads of the present invention can be prepared by any desired or suitable process. For example, polymers of the formula

136



can be prepared by providing the corresponding poly(arylene ether ketone) and then reducing the poly(arylene ether ketone) with borane to form the poly(arylene ether alcohol), as follows:



Typically, about 10 parts by weight of the corresponding poly(arylene ether ketone) are dissolved in about 100 grams of a suitable solvent, such as tetrahydrofuran, to which is added under inert atmosphere (such as argon) and with mechanical stirring a one Molar solution of a borane-tetrahydrofuran complex in tetrahydrofuran (available from, for example, Aldrich Chemical Co., Milwaukee, Wis.). Generally, one mole of the borane-tetrahydrofuran complex is added for each polymeric carbonyl group to assure complete reduction of the carbonyl groups. Some or all of the keto groups can be reduced, depending on the amount of borane-tetrahydrofuran complex added. When not all of the carbonyl groups are reduced to alcohol groups, preferably at least about 0.1 percent of the carbonyl groups are reduced, more preferably at least about 10 percent of the carbonyl groups are reduced, and even more preferably at least about 25 percent of the carbonyl groups are reduced. Most preferably, about 100 percent of the carbonyl groups are reduced.

Hydroxymethyl groups can also be placed on the polymer by using as a starting material the corresponding poly(arylene ether ketone) substituted with, for example, acetyl groups, as follows:



-continued



The backbone carbonyl groups are reduced by the borane-tetrahydrofuran complex at 25° C.; the pendant acetyl groups, however, generally are reduced under elevated temperatures (e.g., tetrahydrofuran boiling at reflux for up to about 2 hours). One mole of the borane-tetrahydrofuran complex is added to reduce each mole of acetyl groups to the corresponding hydroxymethyl groups.

The polymers for the printheads of the present invention can also be prepared via a Grignard process. Specifically, about 10 parts by weight of the polymer in about 100 parts by weight of dry tetrahydrofuran are reacted with one molar equivalent of the Grignard reagent (RMgX, wherein R is the group ultimately added to the carbonyl bond in the polymer and X is a halogen, such as chlorine, bromine, or iodine) at ambient temperature (about 25° C.) with mechanical stirring under an inert atmosphere (such as argon). Subsequent addition of water or an acid yields the product. The reaction proceeds as follows:



The corresponding polyarylene ether ketone can be prepared by any desired or suitable process. Processes for the preparation of these materials are known, and disclosed in, for example, U.S. Pat. No. 5,849,809, U.S. Pat. No. 5,739,254, U.S. Pat. No. 5,753,783, U.S. Pat. No. 5,761,809, U.S. Pat. No. 5,863,963, U.S. Pat. No. 5,814,426, U.S. Pat. No.

- 5,874,192, Copending application U.S. Ser. No. 08/705,375, now U.S. Pat. No. 5,994,425, Copending application U.S. Ser. No. 09/221,024, now U.S. Pat. No. 6,022,095, Copending application U.S. Ser. No. 09/159,426, Copending application U.S. Ser. No. 08/705,488, Copending application U.S. Ser. No. 09/221,690, Copending application U.S. Ser. No. 08/697,761, now U.S. Pat. No. 5,889,077, Copending application U.S. Ser. No. 09/221,278, now U.S. Pat. No. 6,087,414, Copending application U.S. Ser. No. 08/705,376, now U.S. Pat. No. 5,958,995, Copending application U.S. Ser. No. 09/220,273, Copending application U.S. Ser. No. 08/705,372, now U.S. Pat. No. 5,945,253, Copending application U.S. Ser. No. 09/246,167, now abandoned Copending application U.S. Ser. No. 09/163,672, now U.S. Pat. No. 6,090,453, Copending application U.S. Ser. No. 08/697,760, now U.S. Pat. No. 6,007,877, Copending application U.S. Ser. No. 09/247,104, Copending application U.S. Ser. No. 08/976,238, now U.S. Pat. No. 5,882,814, Copending application U.S. Ser. No. 09/105,501, Copending application U.S. Ser. No. 09/120,746, and Copending application U.S. Ser. No. 09/217,330, the disclosures of each of which are totally incorporated herein by reference. Further background material is contained in, for example, P. M. Hergenrother, *J. Macromol. Sci. Rev. Macromol. Chem.*, C19 (1), 1-34 (1980); P. M. Hergenrother, B. J. Jensen, and S. J. Havens, *Polymer*, 29, 358 (1988); B. J. Jensen and P. M. Hergenrother, "High Performance Polymers," Vol. 1, No. 1) page 31 (1989), "Effect of Molecular Weight on Poly(arylene ether ketone) Properties"; V. Percec and B. C. Auman, *Makromol. Chem.* 185, 2319 (1984); "High Molecular Weight Polymers by Nickel Coupling of Aryl Polychlorides," I. Colon, G. T. Kwiatkowski, *J. of Polymer Science, Part A, Polymer Chemistry*, 28, 367 (1990); M. Ueda and T. Ito, *Polymer J.*, 23 (4), 297 (1991); "Ethynyl-Terminated Polyarylates: Synthesis and Characterization," S. J. Havens and P. M. Hergenrother, *J. of Polymer Science: Polymer Chemistry Edition*, 22, 3011 (1984); "Ethynyl-Terminated Polysulfones: Synthesis and Characterization," P. M. Hergenrother, *J. of Polymer Science: Polymer Chemistry Edition*, 20, 3131 (1982); K. E. Dukes, M. D. Forbes, A. S. Jeevarajan, A. M. Belu, J. M. DeDimone, R. W. Linton, and V. V. Sheares, *Macromolecules*, 29, 3081 (1996); G. Hougham, G. Tesoro, and J. Shaw, *Polym. Mater. Sci. Eng.*, 61, 369 (1989); V. Percec and B. C. Auman, *Makromol. Chem.*, 185, 617 (1984); "Synthesis and characterization of New Fluorescent Poly(arylene ethers)," S. Matsuo, N. Yakoh, S. Chino, M. Mitani, and S. Tagami, *Journal of Polymer Science: Part A: Polymer Chemistry*, 32, 1071 (1994); "Synthesis of a Novel Naphthalene-Based Poly(arylene ether ketone) with High Solubility and Thermal Stability," Mami Ohno, Toshikazu Takata, and Takeshi Endo, *Macromolecules*, 27, 3447 (1994); "Synthesis and Characterization of New Aromatic Poly(ether ketones)," F. W. Mercer, M. T. McKenzie, G. Merlino, and M. M. Fone, *J. of Applied Polymer Science*, 56, 1397 (1995); H. C. Zhang, T. L. Chen, Y. G. Yuan, Chinese Patent CN 85108751 (1991); "Static and laser light scattering study of novel thermoplastics. 1. Phenolphthalein poly(aryl ether ketone)," C. Wu, S. Bo, M. Siddiq, G. Yang, and T. Chen, *Macromolecules*, 29, 2989 (1996); "Synthesis of t-Butyl-Substituted Poly(ether ketone) by Nickel-Catalyzed Coupling Polymerization of Aromatic Dichloride," M. Ueda, Y. Seino, Y. Haneda, M. Yoneda, and J.-I. Sugiyama, *Journal of Polymer Science: Part A: Polymer Chemistry*, 32, 675 (1994); "Reaction Mechanisms: Comb-Like Polymers and Graft Copolymers from Macromers 2. Synthesis, Characterization and Homopolymerization of a Styrene Macromer

139

of Poly(2,6-dimethyl-1,4-phenylene Oxide)," V. Percec, P. L. Rinaldi, and B. C. Auman, *Polymer Bulletin*, 10, 397 (1983); *Handbook of Polymer Synthesis Part A*, Hans R. Kricheldorf, ed., Marcel Dekker, Inc., New York-Basel-Hong Kong (1992); and "Introduction of Carboxyl Groups into Crosslinked Polystyrene," C. R. Harrison, P. Hodge, J. Kemp, and G. M. Perry, *Die Makromolekulare Chemie*, 176, 267 (1975), the disclosures of each of which are totally incorporated herein by reference. Further background on high performance polymers is disclosed in, for example, U.S. Pat. No. 2,822,351; U.S. Pat. No. 3,065,205; British Patent 1,060,546; British Patent 971,227; British Patent 1,078,234; U.S. Pat. No. 4,175,175; N. Yoda and H. Hiramoto, *J. Macromol. Sci.-Chem.*, A21(13 & 14) pp. 1641 (1984) (Toray Industries, Inc., Otsu, Japan; B. Sillion and L. Verdet, "Polyimides and other High-Temperature polymers", edited by M. J. M. Abadie and B. Sillion, Elsevier Science Publishers B.V. (Amsterdam 1991); "Polyimides with Alicyclic Diamines. II. Hydrogen Abstraction and Photocrosslinking Reactions of Benzophenone Type Polyimides," Q. Jin, T. Yamashita, and K. Horie, *J. of Polymer Science: Part A: Polymer Chemistry*, 32, 503 (1994); Probimide™ 300, product bulletin, Ciba-Geigy Microelectronics Chemicals, "Photosensitive Polyimide System;" High Performance Polymers and Composites, J. I. Kroschwitz (ed.), John Wiley & Sons (New York 1991); and T. E. Atwood, D. A. Barr, T. A. King, B. Newton, and B. J. Rose, *Polymer*, 29, 358 (1988), the disclosures of each of which are totally incorporated herein by reference. Further information on radiation curing is disclosed in, for example, *Radiation Curing: Science and Technology*, S. Peter Pappas, ed., Plenum Press (New York 1992), the disclosures of each of which are totally incorporated herein by reference.

Substituted poly(arylene ether alcohol)s can also be prepared by this method; for example, a haloalkylated poly(arylene ether ketone) or an acryloylated poly(arylene ether ketone) can be reacted with borane to yield the corresponding poly(arylene ether alcohol)s as follows:



140

-continued



The acetyl or acetoxy group can be converted to a hydroxyl group by continuing the reaction with borane at from about 70 to about 80° C., as follows:



In some instances, the desired substituents on the final polymer can be present on the ketone precursor polymer prior to reduction thereof; for example, haloalkyl groups or cyano groups can be present on the polymer during the reduction process and emerge therefrom unchanged. Other groups may react with the borane reducing agent; for example, amide groups might be reduced to amino groups, hydroxyl groups might be converted to borate esters, acid groups and ester groups might be reduced to alcohols, and the like.

The poly(arylene ether alcohol) can be further reacted with diisocyanates, acryloyl halides such as acryloyl chloride, methacryloyl halides such as methacryloyl chloride, isocyanato-ethyl acrylate moieties, isocyanato-ethyl methacrylate moieties, or the like to allow thermal and/or photochemical crosslinking of the modified resins. Generally, a molar equivalent of the hydroxy-substituted polymer is combined with a molar equivalent of the reacting agent, such as an isocyanate, and the reaction is allowed to proceed in a solvent, such as tetrahydrofuran, other polar aprotic solvents, or the like, at ambient temperature (about 25° C.) for about 16 hours. For example, the reaction of a poly(arylene ether alcohol) with isocyanato-ethyl methacrylate proceeds as follows:



The hydroxymethyl-substituted poly(arylene ether alcohol), 25 such as



with one specific example being



are like phenolic resins, which can be thermally cured without further modification, especially with acidic catalysts. In particular, light activated cationic initiators can be used in this situation.

The polymers of the present invention suitable for use as photoresists or in other applications wherein crosslinking or chain extension of the polymer can occur via exposure to actinic radiation, heat, crosslinking agents, or combinations thereof, contain in at least some of the monomer repeat units thereof crosslinking substituents which enable crosslinking or chain extension of the polymer upon exposure to actinic radiation. Crosslinking substituents include photosensitivity-imparting substituents, which enable crosslinking or chain extension of the polymer upon exposure to actinic radiation, thermal sensitivity-imparting substituents, which enable crosslinking or chain extension of the polymer upon exposure to heat, chemical crosslinking substituents, which enable crosslinking or chain extension of the polymer upon reaction with a crosslinking agent, substituents which require two or more of actinic radiation, heat, and/or contact with a crosslinking agent to cause crosslinking or chain extension of the polymer, and the like. 55 These polymers, while being encompassed by the more general formula



are more specifically represented by the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



35 or a mixture of



wherein R is a (a) hydrogen atom, (b) an alkyl group, including unsubstituted alkyl groups and substituted alkyl groups, such as hydroxyalkyl groups, preferably with from 1 to about 20 carbon atoms, more preferably with from 1 to about 10 carbon atoms, and even more preferably with from 1 to about 5 carbon atoms, (c) an aryl group, including unsubstituted aryl groups and substituted aryl groups, such as hydroxyaryl groups, preferably with from 6 to about 18 carbon atoms, more preferably with from 6 to about 12 carbon atoms, and even more preferably with 6 carbon atoms, or (d) mixtures thereof, B is



143



$-\text{CH}_2\text{CH}_2\text{v}$ ,

wherein v preferably is an integer of from 1 to about 20, and more preferably from 1 to about 10,



wherein z preferably is an integer of from 2 to about 20, and more preferably from 2 to about 10,

144



10 wherein u preferably is an integer of from 1 to about 20, and more preferably from 1 to about 10,



35

40 wherein w preferably is an integer of from 1 to about 20, and more preferably from 1 to about 10,



**145**

5

wherein R<sub>1</sub> and R<sub>2</sub> each, independently of the other, are (a) hydrogen atoms, (b) alkyl groups, including unsubstituted alkyl groups and substituted alkyl groups, such as hydroxy-alkyl groups, preferably with from 1 to about 20 carbon atoms, more preferably with from 1 to about 10 carbon atoms, and even more preferably with from 1 to about 5 carbon atoms, although the number of carbon atoms can be outside of this range, (c) aryl groups, including unsubstituted aryl groups and substituted aryl groups, such as hydroxyaryl groups, preferably with from 6 to about 18 carbon atoms, more preferably with from 6 to about 12 carbon atoms, and even more preferably with 6 carbon atoms, although the number of carbon atoms can be outside of this range, or (d) mixtures thereof, and p is an integer of 0 or 1,

10

15  
20

wherein p is 0 or 1; (2) Ar is



25

wherein p is an integer of 0 or 1,

30

-(CH<sub>2</sub>O)<sub>t</sub>-

wherein t is an integer of from 1 to about 20,

35



40

45

50

55

60

65

**146**or —Ar—(X)<sub>p</sub>—Ar—

or



or



40

45

50

55

60

65

wherein (1) Z is



-continued



wherein s is 0, 1, or 2,



or



and (6) q is 0 or 1; or mixtures thereof, hydroxy-substituted derivatives thereof, hydroxyalkyl-substituted derivatives thereof, with the hydroxyalkyl substituents preferably having from 1 to about 20 carbon atoms, more preferably from 1 to about 10 carbon atoms, and even more preferably from 1 to about 5 carbon atoms, although the number of carbon atoms can be outside of this range, hydroxyaryl-substituted derivatives thereof, with the hydroxyaryl substituents preferably having from 6 to about 18 carbon atoms, more preferably from 6 to about 12 carbon atoms, and even more preferably about 6 carbon atoms, although the number of carbon atoms can be outside of this range, or mixtures thereof, and n is an integer representing the number of repeating monomer units.

Actinic radiation which activates crosslinking or chain extension of photosensitivity imparting crosslinking groups can be of any desired source and any desired wavelength, including (but not limited to) visible light, infrared light, ultraviolet light, electron beam radiation, x-ray radiation, or the like. Examples of suitable photosensitivity imparting groups include unsaturated ester groups, such as acryloyl groups, methacryloyl groups, cinnamoyl groups, crotonoyl groups, ethacryloyl groups, oleoyl groups, linoleoyl groups, maleoyl groups, fumaroyl groups, itaconoyl groups, citraconoyl groups, phenylmaleoyl groups, esters of 3-hexene-1,6-dicarboxylic acid, and the like. Also suitable are alkylcarboxymethylene and ether groups. Under certain conditions, such as imaging with electron beam, deep ultraviolet, or x-ray radiation, halomethyl groups are also photoactive. Epoxy groups, allyl ether groups, hydroxyalkyl groups, and unsaturated ammonium, phosphonium, and ether groups are also suitable photoactive groups.

The photopatternable polymers containing these groups can be prepared by any suitable or desired process. For example, unsaturated ester groups can be placed directly on the polymer having no photosensitive groups by a process which comprises reacting the polymer with (i) a formalde-

hyde source, and (ii) an unsaturated acid in the presence of an acid catalyst, thereby forming a curable polymer with unsaturated ester groups, as disclosed in, for example, Copending application U.S. Ser. No. 08/697,761, filed Aug. 5 29, 1996, now U.S. Pat. No. 5,889,077 and Copending application U.S. Ser. No. 09/221,278, filed Dec. 23, 1998, now U.S. Pat. No. 6,087,414, entitled "Process for Direct Substitution of High Performance Polymers with Unsaturated Ester Groups," with the named inventors Timothy J. Fuller, Ram S. Narang, Thomas W. Smith, David J. Luca, and Raymond K. Crandall, the disclosures of each of which are totally incorporated herein by reference.

Alternatively, one or more intermediate materials can be prepared. For example, the polymer backbone can be functionalized with a substituent which allows for the facile derivatization of the polymer backbone, such as hydroxyl groups, carboxyl groups, haloalkyl groups such as chloromethyl groups, hydroxyalkyl groups such as hydroxy methyl groups, methoxy methyl groups, alkylcarboxymethylene groups, and the like. For example, the polymer can be substituted with photosensitivity-imparting groups such as unsaturated ester groups or the like by first preparing the haloalkylated derivative and then replacing at least some of the haloalkyl groups with unsaturated ester groups, as disclosed in U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas W. Smith, David J. Luca, and Raymond K. Crandall, and in U.S. Pat. No. 5,761,809, filed Aug. 29, 1996, entitled "Processes for Substituting Haloalkylated Polymers With Unsaturated Ester, Ether, and Alkylcarboxymethylene Groups," with the named inventors Timothy J. Fuller, Ram S. Narang, Thomas W. Smith, David J. Luca, and Raymond K. Crandall, the disclosures of each of which are totally incorporated herein by reference. For example, the haloalkylated polymer can be substituted with unsaturated ester groups by reacting the haloalkylated polymer with an unsaturated ester salt in solution. Ether groups and alkylcarboxymethylene groups can also be placed on the haloalkylated polymer by a process analogous to that employed to place unsaturated ester groups on the haloalkylated polymer, except that the corresponding alkylcarboxylate or alkoxide salt is employed as a reactant. Some or all of the haloalkyl groups can be replaced with unsaturated ester, ether, or alkylcarboxymethylene substituents. Longer reaction times generally lead to greater degrees of substitution of haloalkyl groups with unsaturated ester, ether, or alkylcarboxymethylene substituents.

The haloalkylated polymer can be allyl ether substituted or epoxidized by first reacting the haloalkylated polymer with an unsaturated alcohol salt, such as an allyl alcohol salt, in solution, to generate the allyl-substituted polymer; if desired, the allyl-substituted polymer can be converted to an epoxy-substituted polymer by reacting it with a peroxide, such as hydrogen peroxide, m-chloroperoxybenzoic acid, acetyl peroxide, and the like, as well as mixtures thereof, to yield the epoxidized polyarylene ether, as disclosed in Copending application U.S. Ser. No. 08/705,372, filed Aug. 5 29, 1996, now U.S. Pat. No. 5,945,253, and Copending application U.S. Ser. No. 09/246,167, filed Feb. 8, 1999, now abandoned, entitled "High Performance Curable Polymers and Processes for the Preparation Thereof," with the named inventors Ram S. Narang and Timothy J. Fuller, the disclosures of each of which are totally incorporated herein by reference. Some or all of the haloalkyl groups can be replaced with allyl ether or epoxy substituents. Longer

reaction times generally lead to greater degrees of substitution of haloalkyl groups with allyl ether or epoxy substituents. As also disclosed in the aforementioned references, the epoxidized polymer can also be prepared by reaction of the haloalkylated polymer with an epoxy-group-containing alcohol salt, such as a glycidolate salt, or an unsaturated alcohol salt, such as those set forth hereinabove, in the presence of a molar excess of base (with respect to the unsaturated alcohol salt or epoxy-group-containing alcohol salt), such as sodium hydride, sodium hydroxide, potassium carbonate, quaternary alkyl ammonium salts, or the like, under phase transfer conditions. Unsaturated or allyl ether groups can also be placed on the haloalkylated polymer by other methods, such as by a Grignard reaction, a Wittig reaction, or the like.

The haloalkylated polymer can be substituted with a photosensitivity-imparting, water-solubility-enhancing (or water-dispersability-enhancing) group by reacting the haloalkylated polymer with an unsaturated amine, phosphine, or alcohol, as disclosed in Copending application U.S. Ser. No. 08/697,760, filed Aug. 29, 1996, now U.S. Pat. No. 6,007,877, entitled "Aqueous Developable High Performance Curable Aromatic Ether Polymers," and Copending application U.S. Ser. No. 09/247,104, filed Feb. 9, 1999, entitled "Aqueous Developable High Performance Curable Polymers," with the named inventors Ram S. Narang and Timothy J. Fuller, the disclosures of each of which are totally incorporated herein by reference. Some or all of the haloalkyl groups can be replaced with photosensitivity-imparting, water-solubility-enhancing or water-dispersability-enhancing) substituents. Longer reaction times generally lead to greater degrees of substitution of haloalkyl groups with photosensitivity-imparting, water-solubility-enhancing (or water-dispersability-enhancing) substituents. As also disclosed in the aforementioned references, the unsubstituted polymer can be substituted with two different functional groups, one of which imparts photosensitivity to the polymer and one of which imparts water solubility or water dispersability to the polymer. Examples of reactants which can be reacted with the polymer to substitute the polymer with suitable water solubility enhancing groups or water dispersability enhancing groups include tertiary amines, tertiary phosphines, alkyl thio ethers, and the like. These water solubility imparting substituents or water dispersability imparting substituents can be placed on the polymer by any suitable or desired process. For example, two equivalents of the nucleophilic reagent (amine, phosphine, or thio ether) can be allowed to react with one equivalent of the haloalkylated polymer at 25° C. in a polar aprotic solvent such as dimethylacetamide, dimethyl sulfoxide, N-methyl pyrrolidinone, dimethyl formamide, or the like, with the reactants present in the solvent in a concentration of about 30 percent by weight solids. Reaction times typically are from about 1 to about 24 hours, with 2 hours being typical. Alternatively, the water solubility imparting group or water dispersability imparting group can be nonionic. Nonionic substituents can be placed on the polymer by, for example, reacting from about 2 to about 10 milliequivalents of a salt of the nonionic group (such as an alkali metal salt or the like) with 1 equivalent of the haloalkylated polymer in a polar aprotic solvent such as tetrahydrofuran, dimethylacetamide, dimethyl sulfoxide, N-methyl pyrrolidinone, dimethyl formamide, or the like, in the presence of a base, such as at least about 2 equivalents of sodium hydroxide, at least about 1 equivalent of sodium hydride, or the like, at about 80° C. for about 16 hours. The substitution of poly(vinyl benzyl chloride) polymers with

polyether chains is disclosed in further detail in, for example, Japanese Patent Kokai 78-79,833 (1978) and in *Chem. Abstr.*, 89, 180603 (1978), the disclosures of each of which are totally incorporated herein by reference. Higher degrees of haloalkylation generally enable higher degrees of substitution with water solubility imparting groups or water dispersability imparting groups.

The hydroxymethylation of a polymer of the above formula can be accomplished by reacting the polymer in solution with formaldehyde or paraformaldehyde and a base, such as sodium hydroxide, potassium hydroxide, calcium hydroxide, ammonium hydroxide, tetramethylammonium hydroxide, or the like, as disclosed in U.S. Pat. No. 5,849,809, filed Aug. 29, 1996, and Copending application U.S. Ser. No. 09/159,426, filed Sep. 23, 1998, entitled "Hydroxymethylated High Performance Curable Polymers," with the named inventors Ram S. Narang and Timothy J. Fuller, the disclosures of each of which are totally incorporated herein by reference. Longer reaction times generally result in higher degrees of hydroxymethylation. As also disclosed in the aforementioned references, the unsubstituted polymers can also be hydroxyalkylated by first preparing the haloalkylated derivative and then replacing at least some of the haloalkyl groups with hydroxyalkyl groups. Higher degrees of haloalkylation generally enable higher degrees of substitution with hydroxyalkyl groups, and thereby enable greater photosensitivity of the polymer. Some or all of the haloalkyl groups can be replaced with hydroxyalkyl substituents. Longer reaction times generally lead to greater degrees of substitution of haloalkyl groups with hydroxyalkyl substituents.

Intermediate derivatives can also be prepared by any suitable or desired process. For example, suitable processes for haloalkylating polymers include reaction of the polymers with formaldehyde and hydrochloric acid, bischloromethyl ether, chloromethyl methyl ether, octylchloromethyl ether, or the like, generally in the presence of a Lewis acid catalyst. Bromination of a methyl group on the polymer can also be accomplished with elemental bromine via a free radical process initiated by, for example, a peroxide initiator or light. Halogen atoms can be substituted for other halogens already on a halomethyl group by, for example, reaction with the appropriate hydrohalic acid or halide salt. Methods for the haloalkylation of polymers are also disclosed in, for example, "Chloromethylation of Condensation Polymers Containing an Oxy-1,4-Phenylene Backbone," W. H. Daly et al., *Polymer Preprints*, Vol. 20, No. 1, 835 (1979), the disclosure of which is totally incorporated herein by reference. One specific process suitable for haloalkylating the polymer entails reacting the polymer with an acetyl halide, such as acetyl chloride, and dimethoxymethane in the presence of a halogen-containing Lewis acid catalyst, as disclosed in U.S. Pat. No. 5,739,254, filed Aug. 29, 1996, and U.S. Pat. No. 5,753,783, filed Aug. 28, 1997, entitled "Process for Haloalkylation of High Performance Polymers," with the named inventors Timothy J. Fuller, Ram S. Narang, Thomas W. Smith, David J. Luca, and Raymond K. Crandall, the disclosures of each of which are totally incorporated herein by reference.

Other procedures for placing functional groups on aromatic polymers are disclosed in, for example, W. H. Daly, S. Chotiwana, and R. Nielsen, *Polymer Preprints*, 20(1), 835 (1979); "Functional Polymers and Sequential Copolymers by Phase Transfer Catalysis, 3. Synthesis And Characterization of Aromatic Poly(ether sulfone)s and Poly(oxy-2,6-dimethyl-1,4-phenylene) Containing Pendant Vinyl Groups," V. Percec and B. C. Auman, *Makromol. Chem.*,

151

185, 2319 (1984); F. Wang and J. Roovers, *Journal of Polymer Science: Part A: Polymer Chemistry*, 32, 2413 (1994); "Details Concerning the Chloromethylation of Soluble High Molecular Weight Polystyrene Using Dimethoxymethane, Thionyl Chloride, And a Lewis Acid: A Full Analysis," M. E. Wright, E. G. Toplikar, and S. A. Svejda, *Macromolecules*, 24, 5879 (1991); "Functional Polymers and Sequential Copolymers by Phase Transfer Catalysts," V. Percec and P. L. Rinaldi, *Polymer Bulletin*, 10, 223 (1983); "Preparation of Polymer Resin and Inorganic Oxide Supported Peroxy-Acids and Their Use in the Oxidation of Tetrahydrothiophene," J. A. Greig, R. D. Hancock, and D. C. Sherrington, *Euopeon Polymer J.*, 16, 293 (1980); "Preparation of Poly(vinylbenzyltriphenylphosphonium Perbromide) and Its Application in the Bromination of Organic Compounds," A. Akelah, M. Hassanein, and F. Abdel-Galil, *European Polymer J.*, 20 (3) 221 (1984); J. M. J. Frechet and K. K. Haque, *Macromolecules*, 8, 130 (1975); U.S. Pat. No. 3,914,194; U.S. Pat. No. 4,110,279; U.S. Pat. No. 3,367,914; "Synthesis of Intermediates for Production of Heat Resistant Polymers (Chloromethylation of Diphenyl oxide)," E. P. Tepenitsyna, M. I. Farberov, and A. P. Ivanovski, *Zhurnal Prikladnoi Khimii*, Vol. 40, No. 11, 2540 (1967); U.S. Pat. No. 3,000,839; Chem Abst. 56, 590f (1962); U.S. Pat. No. 3,128,258; Chem Abstr. 61, 4560a (1964); J. D. Doedens and H. P. Cordts, *Ind. Eng. Ch.*, 83, 59 (1961); British Patent 863,702; and Chem Abstr. 55, 18667b (1961); the disclosures of each of which are totally incorporated herein by reference.

Thermal sensitivity-imparting groups are also suitable crosslinking groups for the polymers of the present invention. Examples of thermal sensitivity-imparting crosslinking groups include those disclosed in Copending application U.S. Ser. No. 08/705,488, filed Aug. 29, 1996, entitled "High Performance Polymer Compositions Having Photosensitivity-Imparting Substituents and Thermal Sensitivity-Imparting Substituents," and Copending application U.S. Ser. No. 09/221,690, filed Dec. 23, 1998, entitled "High Performance Polymer Compositions," with the named inventors Thomas W. Smith, Timothy J. Fuller, Ram S. Narang, and David J. Luca, the disclosures of each of which are totally incorporated herein by reference. The thermal sensitivity imparting groups can be placed on the polymer by any suitable or desired synthetic method. Processes for putting the above mentioned thermal sensitivity imparting groups on polymers are disclosed in, for example, "Polyimides," C. E. Sroog, *Prog. Polym. Sci.*, Vol. 16, 561-694 (1991); F. E. Arnold and L. S. Tan, *Symposium on Recent Advances in Polyimides and Other High Performance Polymers*, Reno, Nev. (July 1987); L. S. Tan and F. E. Arnold, *J. Polym. Sci. Part A*, 26, 1819 (1988); U.S. Pat. No. 4,973,636; and U.S. Pat. No. 4,927,907; the disclosures of each of which are totally incorporated herein by reference. Other procedures for placing thermally curable end groups on aromatic polymers are disclosed in, for example, P. M. Hergenrother, *J. Macromol. Sci. Rev. Macromol. Chem.*, C19 (1), 1-34 (1980); V. Percec and B. C. Auman, *Makromol. Chem.*, 185,2319 (1984); S. J. Havens, and P. M. Hergenrother, *J. of Polymer Science: Polymer Chemistry Edition*, 22, 3011 (1984); P. M. Hergenrother, *J. of Polymer Science: Polymer Chemistry Edition*, 20, 3131 (1982); V. Percec, P. L. Rinaldi, and B. C. Auman, *Polymer Bulletin*, 10, 215 (1983); "Functional Polymers and Sequential Copolymers by Phase Transfer Catalysis, 2. Synthesis and Characterization of Aromatic Poly(ether sulfones Containing Vinylbenzyl and Ethynylbenzyl Chain Ends," V. Percec and B. C. Auman, *Makromol. Chem.* 185, 1867 (1984);

152

"Functional Polymers and Sequential Copolymers by Phase Transfer Catalysis, 6. On the Phase Transfer Catalyzed Williamson Polyetherification as a New Method for the Preparation of Alternating Block copolymers," V. Percec, B. C. Auman, and P. L. Rinaldi, *Polymer Bulletin*, 10, 391 (1983); "Functional Polymers and Sequential Copolymers by Phase Transfer Catalysis, 3 Synthesis and Characterization of Aromatic Poly(ether sulfone)s and Poly(oxy-2,6-dimethyl-1,4-phenylene) Containing Pendant Vinyl Groups," V. Percec and B. C. Auman, *Makromol. Chem.*, 185, 2319 (1984); and "Phase Transfer Catalysis, Functional Polymers and Sequential Copolymers by PTC,5. Synthesis and Characterization of Polyformals of Polyether Sulfones," *Polymer Bulletin*, 10, 385 (1983); the disclosures of each of which are totally incorporated herein by reference. When both photosensitivity-imparting crosslinking groups and thermal sensitivity-imparting crosslinking groups are present on the polymers of the present invention, as disclosed in Copending application U.S. Ser. No. 08/705,488 and Copending application U.S. Ser. No. 09/221,690, the polymers can also be cured in a two-stage process which entails (a) exposing the polymer to actinic radiation, thereby causing the polymer to become crosslinked or chain extended through the photosensitivity-imparting groups; and (b) subsequent to step (a), heating the polymer to a temperature sufficient to cause the thermal sensitivity-imparting groups to react, thereby causing further crosslinking or chain extension of the polymer through the thermal sensitivity imparting groups.

Examples of suitable thermal sensitivity imparting groups include ethynyl groups, such as those of the formula



wherein R is



153

-continued



a is an integer of 0 or 1, and R' is a hydrogen atom or a phenyl group, ethylenic linkage-containing groups, such as allyl groups, including those of the formula



wherein X and Y each, independently of the other, are hydrogen atoms or halogen atoms, such as fluorine, chlorine, bromine, or iodine, vinyl groups, including those of the formula



wherein R is an alkyl group, including both saturated, unsaturated, linear, branched, and cyclic alkyl groups, preferably with from 1 to about 30 carbon atoms, more preferably with from 1 to about 11 carbon atoms, even more preferably with from 1 to about 5 carbon atoms, a substituted alkyl group, an aryl group, preferably with from 6 to about 24 carbon atoms, more preferably with from 6 to about 18 carbon atoms, a substituted aryl group, an arylalkyl group, preferably with from 7 to about 30 carbon atoms, more preferably with from 7 to about 19 carbon atoms, or a substituted arylalkyl group, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring, vinyl ether groups, such as those of the formula



154

epoxy groups, including those of the formula

5



- 10 R is an alkyl group, including both saturated, unsaturated, linear, branched, and cyclic alkyl groups, preferably with from 1 to about 30 carbon atoms, more preferably with from 1 to about 11 carbon atoms, even more preferably with from 1 to about 5 carbon atoms, a substituted alkyl group, an aryl group, preferably with from 6 to about 24 carbon atoms, more preferably with from 6 to about 18 carbon atoms, a substituted aryl group, an arylalkyl group, preferably with from 7 to about 30 carbon atoms, more preferably with from 7 to about 19 carbon atoms, or a substituted arylalkyl group, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring, halomethyl groups, such as fluoromethyl groups, chloromethyl groups, bromomethyl groups, and iodomethyl groups, hydroxymethyl groups, benzocyclobutene groups, including those of the formula



- 45 50 phenolic groups (- $\phi$ -OH), provided that the phenolic groups are present in combination with either halomethyl groups or hydroxymethyl groups; the halomethyl groups or hydroxymethyl groups can be present on the same polymer bearing the phenolic groups or on a different polymer, or on a monomeric species present with the phenolic group substituted polymer; maleimide groups, such as those of the formula

55



60

65

155

biphenylene groups, such as those of the formula



5-norbornene-2,3-dicarboximido (nадимидо) groups, such as those of the formula



alkylcarboxylate groups, such as those of the formula



wherein R is an alkyl group (including saturated, unsaturated, and cyclic alkyl groups), preferably with from 1 to about 30 carbon atoms, more preferably with from 1 to about 6 carbon atoms, a substituted alkyl group, an aryl group, preferably with from 6 to about 30 carbon atoms, more preferably with from 1 to about 2 carbon atoms, a substituted aryl group, an arylalkyl group, preferably with from 7 to about 35 carbon atoms, more preferably with from 7 to about 15 carbon atoms, or a substituted arylalkyl group, wherein the substituents on the substituted alkyl, aryl, and arylalkyl groups can be (but are not limited to) alkoxy groups, preferably with from 1 to about 6 carbon atoms, aryloxy groups, preferably with from 6 to about 24 carbon atoms, arylalkyloxy groups, preferably with from 7 to about 30 carbon atoms, hydroxy groups, amine groups, imine groups, ammonium groups, pyridine groups, pyridinium groups, ether groups, ester groups, amide groups, carbonyl groups, thiocarbonyl groups, sulfate groups, sulfonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein two or more substituents can be joined together to form a ring, and the like. Any desired or suitable degree of substitution can be employed. Preferably, the degree of substitution is from about 1 to about 4 thermal sensitivity imparting groups per repeat monomer unit, although the degree of substitution can be outside this range. Preferably, the degree of substitution is from about 0.5 to about 5 milliequivalents of thermal sensitivity imparting group per gram of polymer, and more preferably from about 0.75 to about 1.5 milliequivalents per gram, although the degree of substitution can be outside this range.

The temperature selected for the thermal crosslinking generally depends on the thermal sensitivity imparting group which is present on the polymer. For example, ethynyl groups preferably are cured at temperatures of from about 150 to about 300° C. Halomethyl groups preferably are cured at temperatures of from about 150 to about 260° C. Hydroxymethyl groups preferably are cured at temperatures

156

of from about 150 to about 250° C. Phenylethynyl phenyl groups preferably are cured at temperatures of greater than about 250° C. Vinyl groups preferably are cured at temperatures of from about 80 to about 250° C. Allyl groups preferably are cured at temperatures of over about 200° C. Epoxy groups preferably are cured at temperatures of about 150° C. Maleimide groups preferably are cured at temperatures of from about 200 to about 300° C. Benzocyclobutene groups preferably are cured at temperatures of over about 200° C. 5-Norbornene-2,3-dicarboximidogroups preferably are cured at temperatures of from about 200 to about 300° C. Vinyl ether groups preferably are cured at temperatures of about 150° C. Phenolic groups in the presence of hydroxymethyl or halomethyl groups preferably are cured at temperatures of from about 150 to about 210° C. Alkylcarboxylate groups preferably are cured at temperatures of from about 150 to about 250° C. Curing temperatures usually do not exceed about 400° C., although higher temperatures can be employed provided that decomposition of the polymer does not occur. Higher temperature cures preferably take place in an oxygen-excluded environment.

Further examples of suitable crosslinking groups include isocyanate groups, acryloyl halide groups such as acryloyl chloride groups, vinyl benzyl halide groups such as vinyl benzyl chloride groups, ethynyl benzyl halide groups such as ethynyl benzyl chloride groups, methacryloyl halide groups such as methacryloyl chloride groups, 2-isocyanatoethyl methacrylate groups, diisocyanate groups, including toluene diisocyanate, hexane diisocyanate, and the like, and any other suitable functional group which enables crosslinking or chain extension of the polymer upon exposure to actinic radiation, heat, crosslinking agents, mixtures thereof, or the like.

Further information regarding photoresist compositions is disclosed in, for example, J. J. Zupancic, D. C. Blazej, T. C. Baker, and E. A. Dinkel, *Polymer Preprints*, 32, (2), 178 (1991); "High Performance Electron Negative Resist, Chloromethylated Polystyrene. A Study on Molecular Parameters," S. Imamura, T. Tamamura, and K. Harada, *J. of Applied Polymer Science*, 27, 937 (1982); "Chloromethylated Polystyrene as a Dry Etching-Resistant Negative Resist for Submicron Technology", S. Imamura, *J. Electrochem. Soc.: Solid-state Science and Technology*, 126(9), 1628 (1979); "UV curing of composites based on modified unsaturated polyesters," W. Shi and B. Ranby, *J. of Applied Polymer Science*, Vol. 51, 1129 (1994); "Cinnamates VI. Light-Sensitive Polymers with Pendant o-, m- and p-hydroxycinnamate Moieties," F. Scigalski, M. Toczek, and J. Paczkowski, *Polymer*, 35, 692 (1994); and "Radiation-cured Polyurethane Methacrylate Pressure-sensitive Adhesives," G. Ansell and C. Butler, *Polymer*, 35 (9), 2001 (1994), the disclosures of each of which are totally incorporated herein by reference.

When the crosslinking groups are photosensitivity imparting groups, the photopatternable polymer can be cured by uniform exposure to actinic radiation at wavelengths and/or energy levels capable of causing crosslinking or chain extension of the polymer through the photosensitivity-imparting groups. Alternatively, the photopatternable polymer is developed by imagewise exposure of the material to radiation at a wavelength and/or at an energy level to which the photosensitivity-imparting groups are sensitive. Typically, a photoresist composition will contain the photopatternable polymer, an optional solvent for the photopatternable polymer, an optional sensitizer, and an optional photoinitiator. Solvents may be particularly desirable when the uncrosslinked photopatternable polymer has a high  $T_g$ .

The solvent and photopatternable polymer typically are present in relative amounts of from 0 to about 99 percent by weight solvent and from about 1 to 100 percent polymer, preferably are present in relative amounts of from about 20 to about 60 percent by weight solvent and from about 40 to about 80 percent by weight polymer, and more preferably are present in relative amounts of from about 30 to about 60 percent by weight solvent and from about 40 to about 70 percent by weight polymer, although the relative amounts can be outside these ranges.

While not being limited to any particular theory, it is believed that exposure to, for example, ultraviolet radiation generally leads to crosslinking or chain extension at the "long" bond sites as shown below for the unsaturated ester-substituted polymer having, for example, acryloyl functional groups, wherein the ethylenic linkage in the acryloyl group is opened to form the link:



Similarly, it is believed that exposure to, for example, ultraviolet radiation generally leads to crosslinking or chain extension at the "long" bond sites as shown below for the acrylate-isocyanate modified polymer, wherein the ethylenic linkage in the functional group is opened to form the link:



An analogous opening of the ethylenic linkage occurs for other unsaturated groups. The alkylcarboxymethylene and ether substituted polymers are curable by exposure to ultra-

violet light, preferably in the presence of heat and one or more cationic initiators, such as triarylsulfonium salts, diaryliodonium salts, and other initiators as disclosed in, for example, Ober et al., *J.M.S.—Pure Appl. Chem.*, A30 (12), 877-897 (1993); G. E. Green, B. P. Stark, and S. A. Zahir, "Photocrosslinkable Resin Systems," *J. Macro. Sci.—Revs. Macro. Chem.*, C21(2), 187 (1981); H. F. Gruber, "Photo-initiators for Free Radical Polymerization," *Prog. Polym. Sci.*, Vol. 17, 953 (1992); Johann G. Kloosterboer, "Network Formation by Chain Crosslinking Photopolymerization and Its Applications in Electronics," *Advances in Polymer Science*, 89, Springer-Verlag Berlin Heidelberg (1988); and "Diaryliodonium Salts as Thermal Initiators of Cationic Polymerization," J. V. Crivello, T. P. Lockhart, and J. L. Lee, *J. of Polymer Science: Polymer Chemistry Edition*, 21, 97 (1983), the disclosures of each of which are totally incorporated herein by reference. While not being limited to any particular theory, it is believed that the cationic mechanism is as shown below for the methylcarboxymethylene polymer, wherein acetic acid is liberated and the "long" bond indicates the crosslinking or chain extension site:



The reaction is similar for the ether-substituted polymer, except that the corresponding alkanol is liberated.

The allyl ether substituted polymer is developed by imagewise exposure of the material to radiation at a wavelength to which it is sensitive. While not being limited to any particular theory, it is believed that exposure to, for example, ultraviolet radiation generally opens the ethylenic linkage in the allyl ether groups and leads to crosslinking or chain extension at the "long" bond sites as shown below:



159



160



For the epoxy-substituted polymer, while not being limited to any particular theory, it is believed that exposure to, for example, ultraviolet radiation generally causes generation of acidic species by the initiator, followed by reaction 15 of the acidic species with the epoxy groups to cause ring opening and crosslinking or chain extension at the "long" bond sites as shown below:



Amine curing of the epoxidized polymer is also possible, with curing occurring upon the application of heat. While 45 not being limited to any particular theory, it is believed that the curing scheme in one example is as follows:



For the halomethylated polymer, while not being limited to any particular theory, it is believed that exposure to, for example, e-beam, deep ultraviolet, or x-ray radiation generally results in free radical cleavage of the halogen atom from the methyl group to form a benzyl radical. Crosslinking or chain extension then occurs at the "long" bond sites as 25 illustrated below:



For the unsaturated ammonium or unsaturated phosphonium substituted polymers of the present invention, while not being limited to any particular theory, it is believed that 60 exposure to, for example, ultraviolet radiation generally opens the ethylenic linkage in the photosensitivity-imparting groups and leads to crosslinking or chain extension at the "long" bond sites as shown below:

161



For the hydroxyalkylated, haloalkylated, and allyl-substituted polymers of the present invention, one specific example of a class of suitable sensitizers or initiators is that of bis(azides), of the general formula



wherein R is



or



wherein  $\text{R}_1$ ,  $\text{R}_2$ ,  $\text{R}_3$ , and  $\text{R}_4$  each, independently of the others, is a hydrogen atom, an alkyl group, including saturated, unsaturated, and cyclic alkyl groups, preferably with from 1 to about 30 carbon atoms, and more preferably with from 1 to about 6 carbon atoms, a substituted alkyl group, an aryl group, preferably with from 6 to about 18 carbon atoms, and more preferably with about 6 carbon

162

atoms, a substituted aryl group, an arylalkyl group, preferably with from 7 to about 48 carbon atoms, and more preferably with from about 7 to about 8 carbon atoms, or a substituted arylalkyl group, and x is 0 or 1, wherein the substituents on the substituted alkyl, aryl, and aryl groups can be (but are not limited to) alkyl groups, including saturated, unsaturated, linear, branched, and cyclic alkyl groups, preferably with from 1 to about 6 carbon atoms, substituted alkyl groups, preferably with from 1 to about 6 carbon atoms, aryl groups, preferably with from 6 to about 24 carbon atoms, substituted aryl groups, preferably with from 6 to about 24 carbon atoms, arylalkyl groups, preferably with from 7 to about 30 carbon atoms, substituted arylalkyl groups, preferably with from 7 to about 30 carbon atoms, alkoxy groups, preferably with from 1 to about 6 carbon atoms, substituted alkoxy groups, preferably with from 1 to about 6 carbon atoms, aryloxy groups, preferably with from 6 to about 24 carbon atoms, substituted aryloxy groups, preferably with from 6 to about 24 carbon atoms, arylalkyloxy groups, preferably with from 7 to about 30 carbon atoms, substituted arylalkyloxy groups, preferably with from 7 to about 30 carbon atoms, amine groups, imine groups, ammonium groups, pyridine groups, pyridinium groups, ether groups, ester groups, amide groups, carbonyl groups, thiocarbonyl groups, sulfate groups, sulfonate groups, sulfide groups, sulfoxide groups, phosphine groups, phosphonium groups, phosphate groups, mercapto groups, nitroso groups, sulfone groups, acyl groups, acid anhydride groups, azide groups, and the like, wherein the substituents on the substituted alkyl groups, substituted aryl groups, substituted arylalkyl groups, substituted alkoxy groups, substituted aryloxy groups, and substituted arylalkyloxy groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, mixtures thereof, and the like, wherein any two or more substituents can be joined together to form a ring. Examples of suitable bis(azides) include 4,4'-diazidostilbene, of the formula



55

4,4'-diazidobenzophenone, of the formula



60

2,6-di-(4'-azidobenzal)-4-methylcyclohexanone, of the formula



4,4'-diazidobenzalacetone, of the formula



and the like. While not being limited to any particular theory, it is believed that exposure to, for example, ultraviolet radiation enables curing, as illustrated below for the hydroxymethylated polymer:



wherein X and X' each, independently of the other, is —H or —OH (or —H or a halogen atom in the case of the haloalkylated polymer). Similarly, for the allyl-substituted polymer, it is believed that the curing reaction scheme is as follows:



165

Alternatively, a hydroxyalkylated polymer can be further reacted to render it more photosensitive. For example, a hydroxymethylated polymer of the formula



can react with isocyanato-ethyl methacrylate, of the formula



(available from Polysciences, Warrington, Pa.) to form a photoactive polymer of the formula



This reaction can be carried out in tetrahydrofuran at 25° C. with 1 part by weight polymer, 1 part by weight isocyanato-ethyl methacrylate, and 50 parts by weight methylene chloride. Typical reaction temperatures are from about 0 to about 50° C., with 10 to 25° C. preferred. Typical reaction times are between about 1 and about 24 hours, with about 16 hours preferred. During exposure to, for example, ultraviolet radiation, the ethylenic bond opens and crosslinking or chain extension occurs at that site.

While not being limited to any particular theory, it is believed that thermal cure can also lead to extraction of the hydroxy group and to crosslinking or chain extension at the "long" bond sites as shown below:



If desired, the hydroxyalkylated polymer can be further reacted with an unsaturated acid chloride to substitute some or all of the hydroxyalkyl groups with photosensitive groups such as acryloyl or methacryloyl groups or other unsaturated

166

ester groups, as disclosed in U.S. Pat. No. 5,849,809 and Copending application U.S. Ser. No. 09/159,426. Some or all of the hydroxyalkyl groups can be replaced with unsaturated ester substituents. Longer reaction times generally lead to greater degrees of substitution of hydroxyalkyl groups with unsaturated ester substituents.

Crosslinkable or chain extendable polymeric materials of the present invention can be used as components in ink jet printheads. The printheads of the present invention can be of any suitable configuration. An example of a suitable configuration, suitable in this instance for thermal ink jet printing, is illustrated schematically in FIG. 1, which depicts an enlarged, schematic isometric view of the front face 29 of a printhead 10 showing the array of droplet emitting nozzles 27. Referring also to FIG. 2, discussed later, the lower electrically insulating substrate or heating element plate 28 has the heating elements 34 and addressing electrodes 33 patterned on surface 30 thereof, while the upper substrate or channel plate 31 has parallel grooves 20 which extend in one direction and penetrate through the upper substrate front face edge 29. The other end of grooves 20 terminate at slanted wall 21, the floor 41 of the internal recess 24 which is used as the ink supply manifold for the capillary filled ink channels 20, has an opening 25 therethrough for use as an ink fill hole. The surface of the channel plate with the grooves are aligned and bonded to the heater plate 28, so that a respective one of the plurality of heating elements 34 is positioned in each channel, formed by the grooves and the lower substrate or heater plate. Ink enters the manifold formed by the recess 24 and the lower substrate 28 through the fill hole 25 and by capillary action, fills the channels 20 by flowing through an elongated recess 38 formed in the thick film insulative layer 18. The ink at each nozzle forms a meniscus, the surface tension of which prevents the ink from weeping therefrom. The addressing electrodes 33 on the lower substrate or channel plate 28 terminate at terminals 32. The upper substrate or channel plate 31 is smaller than that of the lower substrate in order that the electrode terminals 32 are exposed and available for wire bonding to the electrodes on the daughter board 19, on which the printhead 10 is permanently mounted. Layer 18 is a thick film passivation layer, discussed later, sandwiched between the upper and lower substrates. This layer is etched to expose the heating elements, thus placing them in a pit, and is etched to form the elongated recess to enable ink flow between the manifold 24 and the ink channels 20. In addition, the thick film insulative layer is etched to expose the electrode terminals.

A cross sectional view of FIG. 1 is taken along view line 50 2-2 through one channel and shown as FIG. 2 to show how the ink flows from the manifold 24 and around the end 21 of the groove 20 as depicted by arrow 23. As is disclosed in U.S. Pat. No. 4,638,337, U.S. Pat. No. 4,601,777, and U.S. Pat. No. Re. 32,572, the disclosures of each of which are 55 totally incorporated herein by reference, a plurality of sets of bubble generating heating elements 34 and their addressing electrodes 33 can be patterned on the polished surface of a single side polished (100) silicon wafer. Prior to patterning, the multiple sets of printhead electrodes 33, the resistive 60 material that serves as the heating elements 34, and the common return 35, the polished surface of the wafer is coated with an underglaze layer 39 such as silicon dioxide, having a typical thickness of from about 5,000 Angstroms to about 2 microns, although the thickness can be outside this range. The resistive material can be a doped polycrystalline silicon, which can be deposited by chemical vapor deposition (CVD) or any other well known resistive material such

as zirconium boride ( $ZrB_2$ ). The common return and the addressing electrodes are typically aluminum leads deposited on the underglaze and over the edges of the heating elements. The common return ends or terminals 37 and addressing electrode terminals 32 are positioned at predetermined locations to allow clearance for wire bonding to the electrodes (not shown) of the daughter board 19, after the channel plate 31 is attached to make a printhead. The common return 35 and the addressing electrodes 33 are deposited to a thickness typically of from about 0.5 to about 3 microns, although the thickness can be outside this range, with the preferred thickness being 1.5 microns.

If polysilicon heating elements are used, they may be subsequently oxidized in steam or oxygen at a relatively high temperature, typically about 1,100° C. although the temperature can be above or below this value, for a period of time typically of from about 50 to about 80 minutes, although the time period can be outside this range, prior to the deposition of the aluminum leads, in order to convert a small portion of the polysilicon to  $SiO_2$ . In such cases, the heating elements are thermally oxidized to achieve an overglaze (not shown) of  $SiO_2$  with a thickness typically of from about 500 Angstroms to about 1 micron, although the thickness can be outside this range, which has good integrity with substantially no pinholes.

In one embodiment, polysilicon heating elements are used and an optional silicon dioxide thermal oxide layer 17 is grown from the polysilicon in high temperature steam. The thermal oxide layer is typically grown to a thickness of from about 0.5 to about 1 micron, although the thickness can be outside this range, to protect and insulate the heating elements from the conductive ink. The thermal oxide is removed at the edges of the polysilicon heating elements for attachment of the addressing electrodes and common return, which are then patterned and deposited. If a resistive material such as zirconium boride is used for the heating elements, then other suitable well known insulative materials can be used for the protective layer thereover. Before electrode passivation, a tantalum (Ta) layer (not shown) can be optionally deposited, typically to a thickness of about 1 micron, although the thickness can be above or below this value, on the heating element protective layer 17 for added protection thereof against the cavitation forces generated by the collapsing ink vapor bubbles during printhead operation. The tantalum layer is etched off all but the protective layer 17 directly over the heating elements using, for example,  $CF_4/O_2$  plasma etching. For polysilicon heating elements, the aluminum common return and addressing electrodes typically are deposited on the underglaze layer and over the opposing edges of the polysilicon heating elements which have been cleared of oxide for the attachment of the common return and electrodes.

For electrode passivation, a film 16 is deposited over the entire wafer surface, including the plurality of sets of heating elements and addressing electrodes. The passivation film 16 provides an ion barrier which will protect the exposed electrodes from the ink. Examples of suitable ion barrier materials for passivation film 16 include polyimide, plasma nitride, phosphorous doped silicon dioxide, materials disclosed hereinafter as being suitable for insulative layer 18, and the like, as well as any combinations thereof. An effective ion barrier layer is generally achieved when its thickness is from about 1000 Angstroms to about 10 microns, although the thickness can be outside this range. In 300 dpi printheads, passivation layer 16 preferably has a thickness of about 3 microns, although the thickness can be above or below this value. In 600 dpi printheads, the thickness of passivation layer 16 preferably is such that the combined thickness of layer 16 and layer 18 is about 25 microns, although the thickness can be above or below this

value. The passivation film or layer 16 is etched off of the terminal ends of the common return and addressing electrodes for wire bonding later with the daughter board electrodes. This etching of the silicon dioxide film can be by either the wet or dry etching method. Alternatively, the electrode passivation can be by plasma deposited silicon nitride ( $Si_3N_4$ ).

Next, a thick film type insulative layer 18, of a polymeric material discussed in further detail herein, is formed on the passivation layer 16, typically having a thickness of from about 10 to about 100 microns and preferably in the range of from about 25 to about 50 microns, although the thickness can be outside these ranges. Even more preferably, in 300 dpi printheads, layer 18 preferably has a thickness of about 30 microns, and in 600 dpi printheads, layer 18 preferably has a thickness of from about 20 to about 22 microns, although other thicknesses can be employed. The insulative layer 18 is photolithographically processed to enable etching and removal of those portions of the layer 18 over each heating element (forming recesses 26), the elongated recess 38 for providing ink passage from the manifold 24 to the ink channels 20, and over each electrode terminal 32, 37. The elongated recess 38 is formed by the removal of this portion of the thick film layer 18. Thus, the passivation layer 16 alone protects the electrodes 33 from exposure to the ink in this elongated recess 38. Optionally, if desired, insulative layer 18 can be applied as a series of thin layers of either similar or different composition. Typically, a thin layer is deposited, photoexposed, partially cured, followed by deposition of the next thin layer, photoexposure, partial curing, and the like. The thin layers constituting thick film insulative layer 18 contain a polymer of the formula indicated hereinabove. In one embodiment of the present invention, a first thin layer is applied to contact layer 16, said first thin layer containing a mixture of a polymer of the formula indicated hereinabove and an epoxy polymer, followed by photoexposure, partial curing, and subsequent application of one or more successive thin layers containing a polymer of the formula indicated hereinabove.

FIG. 3 is a similar view to that of FIG. 2 with a shallow anisotropically etched groove 40 in the heater plate, which is silicon, prior to formation of the underglaze 39 and patterning of the heating elements 34, electrodes 33 and common return 35. This recess 40 permits the use of only the thick film insulative layer 18 and eliminates the need for the usual electrode passivating layer 16. Since the thick film layer 18 is impervious to water and relatively thick (typically from about 20 to about 40 microns, although the thickness can be outside this range), contamination introduced into the circuitry will be much less than with only the relatively thin passivation layer 16 well known in the art. The heater plate is a fairly hostile environment for integrated circuits. Commercial ink generally entails a low attention to purity. As a result, the active part of the heater plate will be at elevated temperature adjacent to a contaminated aqueous ink solution which undoubtedly abounds with mobile ions. In addition, it is generally desirable to run the heater plate at a voltage of from about 30 to about 50 volts, so that there will be a substantial field present. Thus, the thick film insulative layer 18 provides improved protection for the active devices and provides improved protection, resulting in longer operating lifetime for the heater plate.

When a plurality of lower substrates 28 are produced from a single silicon wafer, at a convenient point after the underglaze is deposited, at least two alignment markings (not shown) preferably are photolithographically produced at predetermined locations on the lower substrates 28 which make up the silicon wafer. These alignment markings are used for alignment of the plurality of upper substrates 31 containing the ink channels. The surface of the single sided wafer containing the plurality of sets of heating elements is

bonded to the surface of the wafer containing the plurality of ink channel containing upper substrates subsequent to alignment.

As disclosed in U.S. Pat. No. 4,601,777 and U.S. Pat. No. 4,638,337, the disclosures of each of which are totally incorporated herein by reference, the channel plate is formed from a two side polished, (100) silicon wafer to produce a plurality of upper substrates 31 for the printhead. After the wafer is chemically cleaned, a pyrolytic CVD silicon nitride layer (not shown) is deposited on both sides. Using conventional photolithography, a via for fill hole 25 for each of the plurality of channel plates 31 and at least two vias for alignment openings (not shown) at predetermined locations are printed on one wafer side. The silicon nitride is plasma etched off of the patterned vias representing the fill holes and alignment openings. A potassium hydroxide (KOH) anisotropic etch can be used to etch the fill holes and alignment openings. In this case, the [111] planes of the (100) wafer typically make an angle of about 54.7 degrees with the surface of the wafer. The fill holes are small square surface patterns, generally of 5 about 20 mils (500 microns) per side, although the dimensions can be above or below this value, and the alignment openings are from about 60 to about 80 mils (1.5 to 3 millimeters) square, although the dimensions can be outside this range. Thus, the alignment openings are etched entirely through the 20 mil (0.5 millimeter) thick wafer, while the fill holes are etched to a terminating apex at about halfway through to three-quarters through the wafer. The relatively small square fill hole is invariant to further size increase with continued etching so that the etching of the alignment openings and fill holes are not significantly time constrained.

Next, the opposite side of the wafer is photolithographically patterned, using the previously etched alignment holes as a reference to form the relatively large rectangular recesses 24 and sets of elongated, parallel channel recesses that will eventually become the ink manifolds and channels of the printheads. The surface 22 of the wafer containing the manifold and channel recesses are portions of the original wafer surface (covered by a silicon nitride layer) on which an adhesive, such as a thermosetting epoxy, will be applied later for bonding it to the substrate containing the plurality of sets of heating elements. The adhesive is applied in a manner such that it does not run or spread into the grooves or other recesses. The alignment markings can be used with, for example, a vacuum chuck mask aligner to align the channel wafer on the heating element and addressing electrode wafer. The two wafers are accurately mated and can be tacked together by partial curing of the adhesive. Alternatively, the heating element and channel wafers can be given precisely diced edges and then manually or automatically aligned in a precision jig. Alignment can also be performed with an infrared aligner-bonder, with an infrared microscope using infrared opaque markings on each wafer to be aligned, or the like. The two wafers can then be cured in an oven or laminator to bond them together permanently. The channel wafer can then be milled to produce individual upper substrates. A final dicing cut, which produces end face 29, opens one end of the elongated groove 20 producing nozzles 27. The other ends of the channel groove 20 remain closed by end 21. However, the alignment and bonding of the channel plate to the heater plate places the ends 21 of channels 20 directly over elongated recess 38 in the thick film insulative layer 18 as shown in FIG. 2 or directly above the recess 40 as shown in FIG. 3 enabling the flow of ink into the channels from the manifold as depicted by arrows 23. The plurality of individual printheads produced by the final dicing are bonded to the daughter board and the printhead electrode terminals are wire bonded to the daughter board electrodes.

In one embodiment, a heater wafer with a phosphosilicate glass layer is spin coated with a solution of Z6020 adhesion

promoter (0.01 weight percent in 95 parts methanol and 5 parts water, Dow Corning) at 3000 revolutions per minute for 10 seconds and dried at 100° C. for between 2 and 10 minutes. The wafer is then allowed to cool at 25° C. for 5 minutes before spin coating the photoresist containing the photopatternable polymer onto the wafer at between 1,000 and 3,000 revolutions per minute for between 30 and 60 seconds. The photoresist solution is made by dissolving the polyarylene ether alcohol modified with 2-isocyanato-ethyl methacrylate and having from about 1 to about 3 acryloyl groups per repeat unit and a weight average molecular weight of 25,000 in N-methylpyrrolidinone at 40 weight percent solids with Michler's ketone (1.2 parts ketone per every 10 parts of 40 weight percent solids polymer solution). The film is heated (soft baked) in an oven for between 10 and 15 minutes at 70° C. After cooling to 25° C. over 5 minutes, the film is covered with a mask and exposed to 365 nanometer ultraviolet light, amounting to between 150 and 1500 millijoules per cm<sup>2</sup>. The exposed wafer is then heated at 70° C. for 2 minutes post exposure bake, followed by cooling to 25° C. over 5 minutes. The film is developed with 60:40 chloroform/cyclohexanone developer, washed with 90:10 hexanes/cyclohexanone, and then dried at 70° C. for 2 minutes. A second developer/wash cycle is carried out if necessary to obtain a wafer with clean features. The processed wafer is transferred to an oven at 25° C., and the oven temperature is raised from 25 to 90° C. at 2° C. per minute. The temperature is maintained at 90° C. for 2 hours, and then increased to 260° C. at 2° C. per minute. The oven temperature is maintained at 260° C. for 2 hours and then the oven is turned off and the temperature is allowed to cool gradually to 25° C. When thermal cure of the photoresist films is carried out under an inert atmosphere, such as nitrogen or one of the noble gases, such as argon, neon, krypton, xenon, or the like, there is markedly reduced oxidation of the developed film and improved thermal and hydrolytic stability of the resultant devices. Moreover, adhesion of developed photoresist film is improved to the underlying substrate. If a second layer is spin coated over the first layer, the heat cure of the first developed layer can be stopped between 80 and 260° C. before the second layer is spin coated onto the first layer. A second thicker layer is deposited by repeating the above procedure a second time. This process is intended to be a guide in that procedures can be outside the specified conditions depending on film thickness and photoresist molecular weight. Films at 30 microns have been developed with clean features at 600 dots per inch.

For best results with respect to well-resolved features and high aspect ratios, photoresist compositions of the present invention are free of particulates prior to coating onto substrates. In one preferred embodiment, the photoresist composition containing the photopatternable polymer is subjected to filtration through a 2 micron nylon filter cloth (available from Teitko). The photoresist solution is filtered through the cloth under yellow light or in the dark as a solution containing from about 30 to about 60 percent by weight solids using compressed air (up to about 60 psi) and a pressure filtration funnel. No dilution of the photoresist solution is required, and concentrations of an inhibitor (such as, for example, MEHQ) can be as low as, for example, 500 parts per million or less by weight without affecting shelf life. No build in molecular weight of the photopatternable polymer is observed during this filtration process. While not being limited to any particular theory, it is believed that in some instances, such as those when unsaturated ester groups are present on the photopolymerizable polymer, compressed air yields results superior to those obtainable with inert atmosphere because oxygen in the compressed air acts as an effective inhibitor for the free radical polymerization of unsaturated ester groups such as acrylates and methacrylates.

In a particularly preferred embodiment, the photopatternable polymer is admixed with an epoxy resin in relative amounts of from about 75 parts by weight photopatternable polymer and about 25 parts by weight epoxy resin to about 90 parts by weight photopatternable polymer and about 10 parts by weight epoxy resin. Examples of suitable epoxy resins include EPON 1001F, available from Shell Chemical Co., Houston, Tex., believed to be of the formula



and the like, as well as mixtures thereof. Curing agents such as the "Y" curative (meta-phenylenediamine) and the like, as well as mixtures thereof, can be used to cure the epoxy resin at typical relative amounts of about 10 weight percent curative per gram of epoxy resin solids. Process conditions for the epoxy resin blended with the photopatternable polymer are generally similar to those used to process the photoresist without epoxy resin. Preferably, the epoxy or epoxy blend is selected so that its curing conditions are different from the conditions employed to apply, image, develop, and cure the photopatternable polymer. Selective stepwise curing allows development of the photoresist film before curing the epoxy resin to prevent unwanted epoxy residues on the device. Incorporation of the epoxy resin into the photopatternable polymer material improves the adhesion of the photopatternable layer to the heater plate. Subsequent to imaging and during cure of the photopatternable polymer, the epoxy reacts with the heater layer to form strong chemical bonds with that layer, improving adhesive strength and solvent resistance of the interface. The presence of the epoxy may also improve the hydrophilicity of the photopatternable polymer and thus may improve the wetting properties of the layer, thereby improving the refill characteristics of the printhead.

The printhead illustrated in FIGS. 1 through 3 constitutes a specific embodiment of the present invention. Any other suitable printhead configuration comprising ink-bearing channels terminating in nozzles on the printhead surface can also be employed with the materials disclosed herein to form a printhead of the present invention.

The present invention also encompasses printing processes with printheads according to the present invention. One embodiment of the present invention is directed to an ink jet printing process which comprises (1) providing an ink jet printhead comprising a plurality of channels, wherein the channels are capable of being filled with ink from an ink supply and wherein the channels terminate in nozzles on one surface of the printhead, said printhead comprising (i) an upper substrate with a set of parallel grooves for subsequent use as ink channels and a recess for subsequent use as a manifold, the grooves being open at one end for serving as droplet emitting nozzles, (ii) a lower substrate in which one surface thereof has an array of heating elements and addressing electrodes formed thereon, and (iii) a thick film layer deposited on the surface of the lower substrate and over the heating elements and addressing electrodes and patterned to form recesses therethrough to expose the heating elements and terminal ends of the addressing electrodes, said thick

film layer comprising a crosslinked or chain extended photopatternable polymer of the formula indicated hereinabove, the upper and lower substrates being aligned, mated, and bonded together to form the printhead with the grooves in the upper substrate being aligned with the heating elements in the lower substrate to form droplet emitting nozzles; (2) filling the channels with an ink; and (3) causing droplets of ink to be expelled from the nozzles onto a receiver sheet in

an image pattern. A specific embodiment of this process is directed to a thermal ink jet printing process, wherein the droplets of ink are caused to be expelled from the nozzles by heating selected channels in an image pattern. The droplets can be expelled onto any suitable receiver sheet, such as fabric, plain paper such as Xerox® 4024 or 4010, coated papers, transparency materials, or the like.

Specific embodiments of the invention will now be described in detail. These examples are intended to be illustrative, and the invention is not limited to the materials, conditions, or process parameters set forth in these embodiments. All parts and percentages are by weight unless otherwise indicated.

### EXAMPLE I

A polymer of the formula



(hereinafter referred to as poly(4-FPK-FBPA)) wherein n is about 130 and represents the number of repeating monomer units was prepared as follows. A 1-liter, 3-neck round-bottom flask equipped with a Dean-Stark trap (Barrett) trap, condenser, mechanical stirrer, argon inlet, and stopper was situated in a silicone oil bath. 4,4'-Difluorobenzophenone (Aldrich Chemical Co., Milwaukee, Wis., 43.47 grams, 0.1992 mole), 9,9'-bis(4-hydroxyphenyl)fluorenone (Aldrich, 75.06 grams, 0.2145 mole) potassium carbonate (65.56 grams), anhydrous N,N-dimethylacetamide (300 milliliters), and toluene (52 milliliters) were added to the flask and heated to 175° C. (oil bath temperature) while the volatile toluene component was collected and removed. After 5 hours of heating at 175° C. with continuous stirring, the reaction mixture was allowed to cool to 25° C. The solidified mass was extracted with methylene chloride, filtered and added to methanol to precipitate the polymer, which was collected by filtration, washed with water, and washed with methanol. The yield of vacuum dried product,

173

poly(4-FPK-FBPA), was 71.7 grams. The polymer was analyzed by gel permeation chromatography with tetrahydrofuran as the elution solvent with the following results:  $M_n=59,100$ ,  $M_{peak}=144,000$ , and  $M_w=136,100$ . The glass transition temperature of the polymer was 240° C., as determined by using differential scanning calorimetry at a heating rate of 20° C. per minute. Solution cast films from methylene chloride were clear, tough, and flexible. As a result of the stoichiometries used in the reaction, it is believed that this polymer had hydroxyl end groups derived from fluorenone bisphenol.

## EXAMPLE II

A polymer of the formula



was prepared as follows. A 1-liter, 3-neck round-bottom flask equipped with a condenser, mechanical stirrer, argon inlet, and rubber septum was situated in a silicone oil bath. Poly(4-FPK-FBPA) (10 grams, prepared as described in Example I) in tetrahydrofuran (200 grams) was added, followed by 1 molar borane-tetrahydrofuran complex (Aldrich Chemical Co., Milwaukee, Wis., 83.5 grams). The resultant solution gelled. After refluxing the gel with mechanical stirring for 2 hours, the reaction mixture was allowed to cool and remain at 25° C. for 16 hours. Methanol was then cautiously added dropwise to react with residual borane. The solid residue was filtered off, washed with water, and then vacuum dried. Tetrahydrofuran (300 milliliters) was added to the solid, which did not dissolve until acetic acid (20 milliliters) was added. The solution (in portions of 25 milliliters) was added to water (750 milliliters for each 25 milliliter portion of polymer solution) using a Waring blender to precipitate a white polymer. The polymer was filtered, washed extensively with water, filtered, washed with methanol, filtered, and then vacuum dried. The polymer dissolved in tetrahydrofuran but was insoluble in methylene chloride, ethyl acetate, toluene, and methyl isobutyl ketone. When dissolved in tetrahydrofuran (8.5 grams), the hydroxylated polymer (1.2 grams) with N,N'-diphenyl-N,N'-bis(3"-methylphenyl)-(1,1'-biphenyl)-4,4'-diamine (1.2 grams) was used to coat 25 micron charge (hole) transport layers for organic photoreceptors with hydroxygallium phthalocyanine photogenerator layers. Moreover, the addition of 0.1 gram of hexane diisocyanate to the above coating solution was found to improve markedly the electrical properties of the device.

The above reaction was repeated using 19.7 grams of poly(4-FPK-FBPA) in tetrahydrofuran (400 grams) and 1 molar boranetetrahydrofuran complex in tetrahydrofuran (215 grams). After 2 hours reflux and 16 hours at 25° C., the reaction mixture was cautiously treated with methanol and then acetic acid, followed by addition to water to reprecipitate the polymer. The polymer was filtered, washed with water, washed with methanol, and then vacuum dried.

174

## EXAMPLE III

A polymer of the formula



15 was prepared as follows. To a 5-liter 3-neck round-bottom flask equipped with a mechanical stirrer, reflux condenser, argon inlet and stopper that was situated in a silicone oil bath were added sequentially, acetyl chloride (388 grams, 320 milliliters), dimethoxymethane (450 milliliters), methanol (12.5 milliliters), tetrachloroethane (500 milliliters), and poly(4-FPK-FBPA) (100 grams, obtained from Scientific Polymer Products) in tetrachloroethane (1250 milliliters). To this mixture was then added tin tetrachloride (5 milliliters) 20 via an air-tight syringe. The reaction mixture was heated for 2 hours at between 90 and 100° C. oil bath set temperature. After cooling to 25° C., the reaction mixture was added to methanol to reprecipitate the polymer with 0.96 chloromethyl groups per repeat unit.

## EXAMPLE IV

A polymer of the formula



35 was prepared as follows. Chloromethylated poly(4-FPK-FBPA) (prepared as described in Example III, 78.5 grams) in N,N-dimethylacetamide (1,967 grams) was added to a 5-liter, 3-neck, round-bottom flask equipped with a mechanical stirrer, argon inlet and condenser and situated in a silicone oil bath. Sodium acetate (78.5 grams) was added 40 and the reaction mixture was heated for 24 hours at 100° C. The reaction solution was then added to water to precipitate the polymer product, which was filtered and washed with methanol. In a similar procedure, the same polymer was prepared by magnetically stirring chloromethylated poly(4-FPK-FBPA) (25 grams, prepared as described in Example III) in N,N-dimethylacetamide (700 grams) with sodium acetate (15 grams, Aldrich) for one month at 25° C. The reaction solution was then decanted from the insoluble salts that settled on centrifugation, and was added to methanol to precipitate a white polymer that was filtered, washed with water, washed with methanol, and then vacuum dried. The yield was 12.2 grams.

## 175

## EXAMPLE V

A polymer of the formula



was prepared as follows. The acetylated polymer (50 grams, prepared as described in Example IV) in tetrahydrofuran (2,000 grams) was allowed to react with 1-molar borane-tetrahydrofuran complex in tetrahydrofuran (250 milliliters, Aldrich) at reflux for 1 hour. The reaction vessel was a 5-liter, 3-neck, round-bottom flask that was situated in a silicone oil bath and equipped with a mechanical stirrer, condenser, argon inlet, and rubber septum. Methanol was added to neutralize unreacted borane and acetic acid was added to form a solution of the polymer. The reaction mixture was then added to water to precipitate a white polymer that was filtered, washed with water, washed with methanol, and then vacuum dried. The polymer product dissolved in tetrahydrofuran and in a solution of 1-part ethanol to 9-parts tetrahydrofuran.

## EXAMPLE VI

A polymer of the formula



was prepared as follows. A 5-liter, 3-neck round-bottom flask equipped with a Dean-Stark trap (Barrett) trap, condenser, mechanical stirrer, argon inlet, and stopper was situated in a silicone oil bath. 4,4'-Dichlorobenzophenone (Aldrich, 403.95 grams), bisphenol A (Aldrich, 340.87 grams), potassium carbonate (491.7 grams), anhydrous N,N-dimethylacetamide (2,250 milliliters), and toluene (412.5 milliliters, 359.25 grams) were added to the flask and heated to 170° C. (oil bath temperature) while the volatile toluene component was collected and removed. After 48 hours of heating at 170° C. with continuous stirring, the reaction mixture was allowed to cool to 25° C. The reaction mixture was thereafter filtered to remove insoluble salts, and the solution was then added to methanol to precipitate the polymer. The polymer was isolated by filtration, washed with water, washed with methanol, and then vacuum dried.

## EXAMPLE VII

A polymer of the formula



as prepared as follows. Poly(arylene ether ketone) (prepared as described in Example VI, 5 grams) in dioxane (50

## 176

milliliters) was treated with 1 molar borane-tetrahydrofuran complex in tetrahydrofuran (50 milliliters). Heating with stirring at 70° C. was carried out for about 4 hours. The polymer solution gelled at 25° C. within 10 minutes after all 5 the borane solution had been added. Vigorous gas evolution was observed. The polymer was treated with methanol and the polymer dissolved with gas evolution. The reaction mixture was concentrated using a rotary evaporator and was 10 added to water to precipitate a polymer that was extensively washed with water and then with methanol. After vacuum drying, the yield of polymer was 4.6 grams.

## EXAMPLE VIII

A polymer of the formula



was prepared by adding 2-isocyanato-ethyl methacrylate (0.18 gram, Aldrich) to the polyarylene ether alcohol (prepared in Example VII, 0.5 gram) in tetrahydrofuran (3.76 grams). A photoreceptor charge transport layer was 30 made by adding N,N'-diphenyl-N,N'-bis(3"-methylphenyl)-(1,1'-biphenyl)-4,4'-diamine (0.5 gram) to the solution. 35 When coated on a hydroxygallium binder generator layer at 29 microns ( $\pm$ 5 microns) and tested on a flat plate xerographic scanner, the  $V_o$  was 1,020 volts, the dark decay was 60 volts, and the residual voltage after light exposure was 60 volts.

## EXAMPLE IX

A polymer of the formula



was prepared as follows. To a 5-liter 3-neck round-bottom flask equipped with a mechanical stirrer, reflux condenser, argon inlet and stopper that was situated in an ice bath were 55 added sequentially, acetyl chloride (184 grams), dimethoxymethane (225 milliliters, 193 grams), methanol (6.25 milliliters), methylene chloride (500 milliliters), and poly(4-CPK-BPA) (75 grams, prepared as described in 60 Example VIII) in methylene chloride (625 milliliters). To this mixture was then added tin tetrachloride (6.5 milliliters) via an air-tight syringe. The reaction mixture was heated for 4 hours at 55° C. oil bath set temperature. After cooling to 65 25° C., the reaction mixture was added to methanol to reprecipitate the polymer with 0.96 chloromethyl groups per repeat unit.

177  
EXAMPLE X

A polymer of the formula



was prepared as follows. A 500-milliliter, 3-neck round-bottom flask equipped with a Dean-Stark trap (Barrett) trap, condenser, mechanical stirrer, argon inlet, and stopper was situated in a silicone oil bath. 4,4'-Difluorobenzophenone (Aldrich, 21.82 grams), bisphenol A (Aldrich, 22.64 grams), potassium carbonate (40 grams), anhydrous N,N-dimethylacetamide (300 milliliters), and toluene (52 milliliters) were added to the flask and heated to 175° C. (oil bath temperature) while the volatile toluene component was collected and removed. After 5 hours of heating at 175° C. with continuous stirring, phenol (5 grams) was added and the reaction mixture was heated and stirred at 175° C. for 30 more minutes. The reaction mixture was then allowed to cool to 25° C. The solidified mass was extracted with methylene chloride (500 milliliters) and filtered to remove insoluble salts. The solution was concentrated using a rotary evaporator and then was added to methanol to precipitate the polymer. The polymer was isolated by filtration, washed with water, washed with methanol, and then vacuum dried. The yield of vacuum dried product, poly(4-FPK-BPA) was 40 grams.

## EXAMPLE XI

A polymer of the formula



was prepared as follows. To a 1-liter 3-neck round-bottom flask equipped with a mechanical stirrer, reflux condenser, argon inlet and stopper that was situated in a silicone oil bath were added sequentially, acetyl chloride (140.1 grams, 128 milliliters), dimethoxymethane (157.6 grams), methanol (5 milliliters), tetrachloroethane (500 milliliters), and poly(4-FPK-BPA) (40 grams, prepared as described in Example X) in tetrachloroethane (500 milliliters). To this mixture was then added tin tetrachloride (0.6 milliliter) via an air-tight syringe. The reaction mixture was heated for 2 hours at 110° C. oil bath set temperature. After cooling to 25° C., the reaction mixture was added to methanol to reprecipitate the polymer with 1.44 chloromethyl groups per repeat unit.

5  
10



was prepared as follows. The chloromethylated polymer (prepared as described in Example IX, 15 grams) in N,N-dimethylacetamide (300 milliliters) was magnetically stirred with sodium acetate (Aldrich, 9 grams) for one month. The reaction mixture was then centrifuged, and the reaction solution was decanted off from residual salts. The solution was added to water to precipitate a white polymer that was filtered, washed with water, washed with methanol, and then vacuum dried.

## EXAMPLE XII

A polymer of the formula



25  
30  
35  
40  
45

was prepared as follows. The chloromethylated polymer (1.44 CH<sub>2</sub>Cl groups per repeat unit, prepared as described in Example XI, 15 grams) in N,N-dimethylacetamide (283 grams) was magnetically stirred with sodium acetate (Aldrich, 9 grams) for one month. The reaction mixture was then centrifuged, and the reaction solution was decanted off from residual salts. The solution was added to water to precipitate a white polymer that was filtered, washed with water, washed with methanol, and then vacuum dried. The polymer in methylene chloride was reprecipitated into methanol, filtered, and then vacuum dried.

## EXAMPLE XIV

A polymer of the formula



50  
55  
60  
65

was prepared with the chloromethylated polymer (prepared as described in Example XI, 2 grams) in dioxane (50 milliliters) to which was added 1 molar borane-tetrahydrofuran complex (50 milliliters). The solution gelled within 10 minutes at 25° C. The reaction mixture was heated at between 70–80 minutes for 2 hours. Methanol was cautiously added with vigorous gas evolution, and the resultant solution was added to water to precipitate the polymer product. The white polymer was filtered, washed with water, washed with methanol, and then vacuum dried. The polymer (0.5 grams) in tetrahydrofuran (4.5 grams) was roll milled

179

with titanium dioxide (MT500, 0.5 grams) and 60 grams of stainless steel shot for 16 hours. The dispersion was coated using a 0.5 mil Bird applicator on metallized polyethylene terephthalate film and heated from 40 to 150° C. over 40 minutes. A photogenerator layer of hydroxygallium phthalocyanine dispersed in polystyrene-vinyl pyridine in toluene was coated using a 0.25 Bird applicator, and the coating was heated for 5 minutes at 135° C. A charge transport layer solution consisting of N,N'-diphenyl-N,N'-bis(3"-methylphenyl)-(1,1'-biphenyl)-4,4'-diamine (1.2 grams) in polycarbonate (1.2 grams) in methylene chloride (13.45 grams) was coated over the binder generator layer using a 4 mil Bird applicator. The device was dried from 40 to 100° C. over 30 minutes.

## EXAMPLE XV

A polymer of the formula



was prepared as follows. The hydroxymethylated-polyarylene ether alcohol (prepared as described in Example XIV, 1.0 gram) was allowed to react with 2-isocyanoethyl methacrylate (1.10 grams) in N-methylpyrrolidinone (9 grams) for 16 hours.

## EXAMPLE XVI

A heater wafer with a phosphosilicate glass layer was spin coated with a solution of Z6020 adhesion promoter (0.01 weight percent in 95 parts by weight methanol and 5 parts by weight water, obtained from Dow Corning Co., Midland, Mich.) at 3,000 revolutions per minute for 10 seconds and dried at 100° C. for 10 minutes. The wafer was then allowed to cool at 25° C. for 5 minutes before spin coating the photoresist containing the photopatternable polymer onto the wafer at 3,000 revolutions per minute for 60 seconds. The photoresist solution was prepared by dissolving the polyarylene ether alcohol modified with 2-isocyano-ethyl methacrylate with 3 acrylate groups per repeat unit and a weight average molecular weight of 25,000 (prepared as described in Example XV) in N-methylpyrrolidinone at 40 weight percent solids with Michler's ketone (1.2 parts by weight ketone per every 10 parts by weight of 40 weight percent solids polymer solution). The film was heated (soft baked) in an oven for 15 minutes at 70° C. After cooling to 25° C. over 5 minutes, the film was covered with a mask and exposed to 365 nanometer ultraviolet light, amounting to between 150 and 1,500 milliJoules per square centimeter.

180

The exposed wafer was then heated at 70° C. for 2 minutes post exposure bake, followed by cooling to 25° C. over 5 minutes. The film was developed with 60:40 by weight chloroform/cyclohexanone developer, washed with 90:10 by weight hexanes/cyclohexanone, and then dried at 70° C. for 2 minutes. A second developer/wash cycle was carried out to obtain a wafer with clean features. The processed wafer was then transferred to an oven at 25° C., and the oven temperature was raised from 25 to 90° C. at a rate of 2° C. per minute. The temperature was maintained at 90° C. for 2 hours, and was then increased to 260° C. at a rate of 2° C. per minute. The oven temperature was maintained at 260° C. for 2 hours, and the oven was then turned off and the temperature allowed to cool gradually to 25° C. The thermal cure of the photoresist films was carried out under an inert atmosphere (nitrogen) to reduce oxidation of the developed film and to improve the thermal and hydrolytic stability of the resultant devices.

When a second layer was spin coated over the first layer, the heat cure of the first developed layer was stopped

40

between 80 and 260° C. before the second layer was spin coated onto the first layer. A second thicker layer was deposited by repeating the above procedure a second time.

This process is intended to be a guide in that procedures 45 can be outside the specified conditions depending on film thickness and photoresist molecular weight. Films at 30 microns in thickness were developed with clean features at 600 dots per inch.

Other embodiments and modifications of the present 50 invention may occur to those of ordinary skill in the art subsequent to a review of the information presented herein; these embodiments and modifications, as well as equivalents thereof, are also included within the scope of this invention.

What is claimed is:

- 55 1. An ink jet printhead which comprises:
  - (i) an upper substrate, and
  - (ii) a lower substrate in which one surface thereof has an array of heating elements and addressing electrodes formed thereon, said lower substrate having an insulative layer deposited on the surface thereof and over the heating elements and addressing electrodes and patterned to form recesses therethrough to expose the heating elements and terminal ends of the addressing electrodes, said upper and lower substrates being bonded together to form a thermal ink jet printhead having droplet emitting nozzles defined by the upper substrate, the insulative layer on the lower substrate,

181

and the heating elements in the lower substrate, wherein at least one of said upper substrate and said insulative layer comprises a crosslinked or chain extended polymer formed by crosslinking or chain extending a precursor polymer having terminal end groups and monomer repeat units, said precursor polymer being of the formula



wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is



or a mixture of



wherein R is a hydrogen atom, an alkyl group, an aryl group, or mixtures thereof, B is



40

45



50



55



60

65

182

-continued



30

35



40

45

wherein v is an integer of from 1 to about 20,



50

55

wherein z is an integer of from 2 to about 20,



60

65

183

wherein  $u$  is an integer of from 1 to about 20,wherein  $w$  is an integer of from 1 to about 20,wherein  $R_1$  and  $R_2$  each, independently of the other, are 65 hydrogen atoms, alkyl groups, or aryl groups, and  $p$  is an integer of 0 or 1,

184

10 wherein  $p$  is an integer of 0 or 1,

15

wherein  $t$  is an integer of from 1 to about 20,

40

wherein (1)  $Z$  isor  $-Ar-(X)_p-Ar-$

185

wherein p is 0 or 1; (2) Ar is



or



(3) G is an alkyl group selected from alkyl or isoalkyl groups containing from about 2 to about 10 carbon atoms; (4) Ar' is



or



(5) X is



186

wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, said crosslinking or chain extension occurring through crosslinking substituents contained on at least some of the monomer repeat units of the precursor polymer.

20 2. A printhead according to claim 1 wherein the insulative layer comprises a crosslinked or chain extended polymer formed by crosslinking or chain extending the precursor polymer.

25 3. A printhead according to claim 1 wherein the upper substrate comprises a crosslinked or chain extended polymer formed by crosslinking or chain extending the precursor polymer.

30 4. A printhead according to claim 1 wherein the weight average molecular weight of the precursor polymer is from about 1,000 to about 100,000.

35 5. A printhead according to claim 1 wherein the precursor polymer has a value of n of from about 2 to about 70.

6. A printhead according to claim 1 wherein the precursor polymer has "A" groups of the formula



45 and "B" groups of the formula



55

7. A printhead according to claim 1 wherein the precursor polymer has "A" groups of the formula



and "B" groups of the formula



5



or a mixture of



wherein R is a hydrogen atom, an alkyl group, an aryl group, or mixtures thereof, B is



8. A printhead according to claim 1 wherein the crosslinking substituent "P" is a hydroxyalkyl group, a haloalkyl group, an unsaturated ester group, an alkylcarboxymethylene group, an ether group, an epoxy group, an allyl group, an unsaturated ammonium group, an unsaturated phosphonium group, an ethynyl group, a vinyl group, a vinyl ether group, a benzocyclobutene group, a phenolic group, a maleimide group, a biphenylene group, a 5-norbornene-2,3-dicarboximido group, an isocyanate group, an acryloyl halide group, a vinyl benzyl halide group, an ethynyl benzyl halide group, a methacryloyl halide group, a 2-isocyanatoethyl methacrylate group, a diisocyanate group, or a mixture thereof.

9. A process for forming an ink jet printhead which comprises:

- providing a lower substrate in which one surface thereof has an array of heating elements and addressing electrodes having terminal ends formed thereon;
- depositing onto the surface of the lower substrate having the heating elements and addressing electrodes thereon a layer comprising a photopatternable polymer;
- exposing the layer to actinic radiation in an imagewise pattern such that the photopatternable polymer in exposed areas becomes crosslinked or chain extended and the photopatternable polymer in unexposed areas does not become crosslinked or chain extended, wherein the unexposed areas correspond to areas of the lower substrate having thereon the heating elements and the terminal ends of the addressing electrodes;
- removing the photopatternable polymer from the unexposed areas, thereby forming recesses in the layer, said recesses exposing the heating elements and the terminal ends of the addressing electrodes;
- providing an upper substrate comprising a supporting substrate and, coated thereon, a material formed by crosslinking or chain extending a composition comprising a crosslinked or chain extended polymer formed by crosslinking or chain extending a precursor polymer having terminal end groups and monomer repeat units, said precursor polymer being of the formula



50

55

60

wherein P is a substituent which enables crosslinking of the polymer, a, b, c, and d are each integers of 0, 1, 2, 3, or 4, provided that at least one of a, b, c, and d is equal to or greater than 1 in at least some of the monomer repeat units of the polymer, A is

189

-continued



wherein v is an integer of from 1 to about 20,



wherein z is an integer of from 2 to about 20,



wherein u is an integer of from 1 to about 20,



190

wherein w is an integer of from 1 to about 20,

wherein  $\text{R}_1$  and  $\text{R}_2$  each, independently of the other, are hydrogen atoms, alkyl groups, or aryl groups, and p is an integer of 0 or 1,

wherein p is an integer of 0 or 1,

 $-(\text{CH}_2\text{O})_t-$ 

wherein t is an integer of from 1 to about 20,



191



wherein (1) Z is



wherein p is 0 or 1; (2) Ar is



(3) G is an alkyl group selected from alkyl or isoalkyl groups containing from about 2 to about 10 carbon atoms; (4) Ar' is



192



wherein s is 0, 1, or 2,



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and

(f) bonding the upper substrate to the lower substrate to form a thermal ink jet printhead having droplet emitting nozzles defined by the upper substrate, the photopatternable polymer on the lower substrate, and the heating elements in the lower substrate.

65 10. A process according to claim 9 wherein the precursor polymer is prepared by a process which comprises (1) providing a pre-precursor polymer of the formula

193



wherein A is



194

-continued



15 B is



195

-continued



wherein v is an integer of from 1 to about 20,



wherein z is an integer of from 2 to about 20,



wherein u is an integer of from 1 to about 20,



196

wherein w is an integer of from 1 to about 20,

wherein R<sub>1</sub> and R<sub>2</sub> each, independently of the other, are hydrogen atoms, alkyl groups, or aryl groups, and p is an integer of 0 or 1,

45 wherein p is an integer of 0 or 1,

50 -(CH<sub>2</sub>O)<sub>t</sub>-

wherein t is an integer of from 1 to about 20,



197



wherein (1) Z is



wherein p is 0 or 1; (2) Ar is



(3) G is an alkyl group selected from alkyl or isoalkyl groups containing from about 2 to about 10 carbon atoms; (4) Ar' is

US 6,177,238 B1  
198

-continued

or



(5) X is



wherein s is 0, 1, or 2,



or

50

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or

or



and (6) q is 0 or 1; or mixtures thereof, hydroxy-substituted,

hydroxyalkyl-substituted, or hydroxyaryl-substituted

derivatives thereof, or mixtures thereof, and n is an integer

representing the number of repeating monomer units, and

(2) reacting the pre-precursor polymer with borane, resulting

in formation of a precursor polymer of the formula



wherein A is



or a mixture of



wherein R is a hydrogen atom, an alkyl group, an aryl group, or mixtures thereof.

11. A process according to claim 9 wherein the precursor polymer is prepared by a process which comprises (1) providing a pre-precursor polymer of the formula



wherein A is



-continued



30  $-(CH_2)_v-$ ,



65

35 B is



201

-continued



wherein  $v$  is an integer of from 1 to about 20,



wherein  $z$  is an integer of from 2 to about 20,



wherein  $u$  is an integer of from 1 to about 20.



202

-continued



20 wherein w is an integer of from 1 to about 20,



wherein  $R_1$  and  $R_2$  each, independently of the other, are hydrogen atoms, alkyl groups, or aryl groups, and  $p$  is an integer of 0 or 1,



wherein  $p$  is an integer of 0 or 1,  
65

$$-\text{CH}_2\text{O}-$$

203

wherein t is an integer of from 1 to about 20,



wherein (1) Z is



wherein p is 0 or 1; (2) Ar is



204

-continued



5

(3) G is an alkyl group selected from alkyl or isoalkyl groups containing from about 2 to about 10 carbon atoms; (4) Ar' is



15



or



20

(5) X is



30



35



40



45



50

wherein s is 0, 1, or 2,

55



or



60 and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2)

or

205

reacting the pre-precursor polymer with a reagent of the formula  $\text{RMgX}$ , wherein R is a hydrogen atom, an alkyl group, an aryl group, or mixtures thereof and X is a halogen atom, and (3) subsequent to step 2, adding water or acid to the pre-precursor polymer, thereby resulting in formation of a precursor polymer of the formula



5

wherein A is



or a mixture of



wherein R is a hydrogen atom, an alkyl group, an aryl group, or mixtures thereof.

12. A process according to claim 9 wherein the precursor polymer has a weight average molecular weight of from about 1,000 to about 100,000.

13. A process according to claim 9 wherein the precursor polymer has a value of n of from about 2 to about 70.

14. A process according to claim 9 wherein the crosslinking substituent "P" is a hydroxyalkyl group, a haloalkyl group, an unsaturated ester group, an alkylcarboxymethylene group, an ether group, an epoxy group, an alkyl group, an unsaturated ammonium group, an unsaturated phosphonium group, an ethynyl group, a vinyl group, a vinyl ether group, a benzocyclobutene group, a phenolic group, a maleimide group, a biphenylene group, a 5-norbornene-2,3-dicarboximido group, an isocyanate group, an acryloyl halide group, a vinyl benzyl halide group, an ethynyl benzyl halide group, a methacryloyl halide group, a 2-isocyanatoethyl methacrylate groups, a diisocyanate group, or a mixture thereof.

15. A process for forming an ink jet printhead which comprises:

(a) depositing a layer comprising a precursor polymer having terminal end groups and monomer repeat units, said precursor polymer being of the formula



55

60

wherein P is a substituent which enables crosslinking of the polymer, a, b, c, and d are each integers of 0, 1, 2, 3, or 4, provided that at least one of a, b, c, and d is

206

equal to or greater than 1 in at least some of the monomer repeat units of the polymer, A is



10 or a mixture of



wherein R is a hydrogen atom, an alkyl group, an aryl group, or mixtures thereof, B is



-continued



wherein v is an integer of from 1 to about 20,



wherein z is an integer of from 1 to about 20,



wherein u is an integer of from 1 to about 20,



-continued



wherein w is an integer of from 1 to about 20,

wherein  $\text{R}_1$  and  $\text{R}_2$  each, independently of the other, are hydrogen atoms, alkyl groups, or aryl groups, and p is an integer of 0 or 1,

wherein p is an integer of 0 or 1,

 $-(\text{CH}_2\text{O})_t-$ 

wherein t is an integer of from 1 to about 20,



-continued



wherein (1) Z is



wherein p is 0 or 1; (2) Ar is



(3) G is an alkyl group selected from alkyl or isoalkyl groups containing from about 2 to about 10 carbon atoms; (4) Ar' is

5



10



or



(5) X is

20



25



30



35



40



45

wherein s is 0, 1, or 2,

50



or



55

and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units onto a lower substrate in which one surface thereof has an array of heating elements and addressing electrodes having terminal ends formed thereon, said polymer being deposited onto the surface having the heating elements and addressing electrodes thereon;

(b) exposing the layer to actinic radiation in an imagewise pattern such that the precursor polymer is exposed

60

areas becomes crosslinked or chain extended and the precursor polymer in unexposed areas does not become crosslinked or chain extended, wherein the unexposed areas correspond to areas of the lower substrate having thereon the heating elements and the terminal ends of the addressing electrodes;

(c) removing the precursor polymer from the unexposed areas, thereby forming recesses in the layer, said recesses exposing the heating elements and the terminal ends of the addressing electrodes;

(d) providing an upper substrate; and

(e) bonding the upper substrate to the lower substrate to form a thermal ink jet printhead having droplet emitting nozzles defined by the upper substrate, the crosslinked or chain extended polymer on the lower substrate, and the heating elements in the lower substrate.

16. A process according to claim 15 wherein the precursor polymer is prepared by a process which comprises (1) providing a pre-precursor polymer of the formula



wherein A is



25

30



35

40

45

50

55

60

65

B is



213



wherein v is an integer of from 1 to about 20,



wherein z is an integer of from 2 to about 20,



wherein u is an integer of from 1 to about 20,



214

-continued



20 wherein w is an integer of from 1 to about 20,



55 wherein R<sub>1</sub> and R<sub>2</sub> each, independently of the other, are hydrogen atoms, alkyl groups, or aryl groups, and p is an integer of 0 or 1,



65 wherein p is an integer of 0 or 1,

-(CH<sub>2</sub>O)<sub>t</sub>-

215

wherein t is an integer of from 1 to about 20,



wherein (1) Z is



wherein p is 0 or 1; (2) Ar is



216

-continued



5

(3) G is an alkyl group selected from alkyl or isoalkyl groups containing from about 2 to about 10 carbon atoms; (4) Ar' is



10



15



or



20



(5) X is



25



30



35



40



45



50



wherein s is 0, 1, or 2,

55



or



60

and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, and

217

(2) reacting the pre-precursor polymer with borane, resulting in formation of a precursor polymer of the formula



wherein A is



or a mixture of



wherein R is a hydrogen atom, an alkyl group, an aryl group, or mixtures thereof.

17. A process according to claim 15 wherein the precursor polymer is prepared by a process which comprises (1) providing a pre-precursor polymer of the formula



wherein A is



218

-continued

—(CH<sub>2</sub>)<sub>v</sub>,

40

B is



50

55

60

65

-continued



wherein v is an integer of from 1 to about 20,



wherein z is an integer of from 2 to about 20,



wherein u is an integer of from 1 to about 20,

5



10



15



20



25

30 wherein w is an integer of from 1 to about 20,

35



40



45

50



55



60

65 wherein R<sub>1</sub> and R<sub>2</sub> each, independently of the other, are hydrogen atoms, alkyl groups, or aryl groups, and p is an integer of 0 or 1,

221



wherein  $p$  is an integer of 0 or 1,

wherein  $t$  is an integer of from 1 to about 20.



wherein (1) Z is



222

wherein p is 0 or 1; (2) Ar is



or



20

(3) G is an alkyl group selected from alkyl or isoalkyl groups containing from about 2 to about 10 carbon atoms; (4) Ar' is



or



(5) X is



45



50



223

wherein s is 0, 1, or 2,



or



and (6) q is 0 or 1; or mixtures thereof, hydroxy-substituted, hydroxyalkyl-substituted, or hydroxyaryl-substituted derivatives thereof, or mixtures thereof, and n is an integer representing the number of repeating monomer units, (2) reacting the pre-precursor polymer with a reagent of the formula  $\text{RMgX}$ , wherein R is a hydrogen atom, an alkyl group, an aryl group, or mixtures thereof and X is a halogen atom, and (3) subsequent to step 2, adding water or acid to the pre-precursor polymer, thereby resulting in formation of a precursor polymer of the formula



15

wherein R is a hydrogen atom, an alkyl group, an aryl group, or mixtures thereof.

18. A process according to claim 15 wherein the precursor polymer has a weight average molecular weight of from about 1,000 to about 100,000.

19. A process according to claim 15 wherein the precursor polymer has a value of n of from about 2 to about 70.

20. A process according to claim 15 wherein the crosslinking substituent "P" is a hydroxyalkyl group, a haloalkyl group, an unsaturated ester group, an alkylcarboxymethylene group, an ether group, an epoxy group, an allyl group, an unsaturated ammonium group, an unsaturated phosphonium group, an ethynyl group, a vinyl group, a vinyl ether group, a benzocyclobutene group, a phenolic group, a maleimide group, a biphenylene group, a 5-norbornene-2,3-dicarboximido group, an isocyanate group, an acryloyl halide group, a vinyl benzyl halide group, an ethynyl benzyl halide group, a methacryloyl halide group, a 2-isocyanatoethyl methacrylate groups, a diisocyanate group, or a mixture thereof.

\* \* \* \* \*

224

wherein A is



or a mixture of



15

wherein R is a hydrogen atom, an alkyl group, an aryl group, or mixtures thereof.